



US010676693B2

(12) **United States Patent**  
**Dykstra et al.**

(10) **Patent No.:** **US 10,676,693 B2**  
(b4) **Date of Patent:** \*Jun. 9, 2020

(54) **TREATMENT COMPOSITIONS**

(71) **Applicant:** **The Procter & Gamble Company**,  
Cincinnati, OH (US)

(72) **Inventors:** **Robert Richard Dykstra**, West  
Chester, OH (US); **Mark Robert Sivik**,  
Mason, OH (US); **Travis Kyle  
Hodgdon**, Cincinnati, OH (US);  
**Stephanie Ann Urbin**, Liberty  
Township, OH (US); **Alessandro  
Corona, III**, Mason, OH (US); **Jocelyn  
Michelle McCullough**, Loveland, OH  
(US); **Denise Malcuit Belanger**, West  
Chester, OH (US); **Kristi Lynn Fliter**,  
Harrison, OH (US); **Richard Timothy  
Hartshorn**, Lawrenceburg, IN (US);  
**Nicholas David Vetter**, Cleves, OH  
(US); **Tessa Xuan**, Cincinnati, OH  
(US); **Reinhold Joseph Leyrer**,  
Dannstadt (DE); **Gledison Fonseca**,  
Mannheim (DE); **Volodymyr Boyko**,  
Mannheim (DE); **Aaron  
Flores-Figueroa**, Mannheim (DE)

(73) **Assignee:** **The Procter & Gamble Company**,  
Cincinnati, OH (US)

(\*) **Notice:** Subject to any disclaimer, the term of this  
patent is extended or adjusted under 35  
U.S.C. 154(b) by 38 days.

This patent is subject to a terminal dis-  
claimer.

(21) **Appl. No.:** **15/464,599**

(22) **Filed:** **Mar. 21, 2017**

(65) **Prior Publication Data**

US 2017/0191002 A1 Jul. 6, 2017

**Related U.S. Application Data**

(63) Continuation of application No. 14/806,685, filed on  
Jul. 23, 2015, now abandoned.

(60) Provisional application No. 62/083,927, filed on Nov.  
25, 2014, provisional application No. 62/027,814,  
filed on Jul. 23, 2014.

(51) **Int. Cl.**

**CIID 3/37** (2006.01)  
**CIID 3/00** (2006.01)  
**CIID 3/12** (2006.01)  
**CIID 3/22** (2006.01)  
**CIID 1/66** (2006.01)  
**CIID 1/62** (2006.01)  
**CIID 3/30** (2006.01)  
**CIID 3/34** (2006.01)  
**CIID 3/50** (2006.01)

(52) **U.S. Cl.**

CPC ..... **CIID 3/0015** (2013.01); **CIID 1/62**  
(2013.01); **CIID 1/662** (2013.01); **CIID 1/667**  
(2013.01); **CIID 3/001** (2013.01); **CIID**

**3/1253** (2013.01); **CIID 3/227** (2013.01);  
**CIID 3/30** (2013.01); **CIID 3/349** (2013.01);  
**CIID 3/373** (2013.01); **CIID 3/3749**  
(2013.01); **CIID 3/3769** (2013.01); **CIID**  
**3/3773** (2013.01); **CIID 3/3796** (2013.01);  
**CIID 3/505** (2013.01)

(58) **Field of Classification Search**  
CPC ..... C11D 3/3769; C11D 3/3773; C11D 1/62;  
C11D 3/0015; C11D 3/001  
See application file for complete search history.

(56) **References Cited**

## U.S. PATENT DOCUMENTS

|              |         |                   |
|--------------|---------|-------------------|
| 4,137,180 A  | 1/1979  | Naik et al.       |
| 4,199,464 A  | 4/1980  | Cambre            |
| 4,528,321 A  | 7/1985  | Allen et al.      |
| 5,296,622 A  | 3/1994  | Uphues et al.     |
| 5,759,990 A  | 6/1998  | Wahl et al.       |
| 6,271,192 B1 | 8/2001  | Verstrat et al.   |
| 6,326,430 B1 | 12/2001 | Berte             |
| 6,348,541 B1 | 2/2002  | Kanda et al.      |
| 6,361,781 B2 | 3/2002  | Lorant            |
| 6,376,456 B1 | 4/2002  | Murphy et al.     |
| 6,413,920 B1 | 7/2002  | Bettoli et al.    |
| 6,494,920 B1 | 12/2002 | Weuthe et al.     |
| 6,620,777 B2 | 9/2003  | Heibel et al.     |
| 6,924,261 B2 | 8/2005  | Grandmaire et al. |
| 6,992,058 B2 | 1/2006  | Grandmaire et al. |
| 7,063,895 B2 | 6/2006  | Rodrigues et al.  |
| 7,378,033 B2 | 5/2008  | Harrison et al.   |
| 7,381,417 B2 | 6/2008  | Gamez-Garcia      |
| 7,981,850 B2 | 7/2011  | Doi et al.        |
| 8,188,022 B2 | 5/2012  | Sengupta et al.   |
| 8,211,414 B2 | 7/2012  | Chen et al.       |

(Continued)

## FOREIGN PATENT DOCUMENTS

|    |             |         |
|----|-------------|---------|
| CA | 2482306 C   | 10/2011 |
| CN | 101724132 B | 11/2011 |

(Continued)

## OTHER PUBLICATIONS

International Preliminary Report on Patentability; International Application No. PCT/US2015/041654; dated Nov. 3, 2016; 12 pages.  
Schuck, Peter, Size-Distribution Analysis of Macromolecules by Sedimentation Velocity Ultracentrifugation and Lamm Equation Modeling, Biophysical Journal, Mar. 2000, pp. 1606-1619, vol. 78, No. 3.  
ASTM D3954-94 (Reapproved 2010), Standard Test Method for Dropping Point of Waxes.  
Invitation to pay additional fees; International Application No. PCT/US2015/041654; dated Nov. 2, 2015; 6 pages.

(Continued)

*Primary Examiner* — John R Hardee

(74) *Attorney, Agent, or Firm* — Gregory S.  
Darley-Emerson

(57) **ABSTRACT**

The present invention relates to treatment compositions containing polymer systems that provide stability and benefit agent deposition as well as methods of making and using same. Such treatment compositions may be used for example as through the wash and/or through the rinse fabric enhancers as well as unit dose treatment compositions.

(56)

## References Cited

## U.S. PATENT DOCUMENTS

8,524,649 B2 9/2013 Leyrer et al.  
 8,563,498 B2 10/2013 Gizaw et al.  
 8,741,831 B2 6/2014 Jaynes et al.  
 8,835,373 B2 9/2014 Miravet Celades et al.  
 9,018,154 B2 4/2015 Blondel  
 9,441,188 B2 9/2016 Schramm, Jr. et al.  
 2002/0132749 A1 9/2002 Smith et al.  
 2004/0038851 A1 2/2004 Aubay et al.  
 2004/0065208 A1 4/2004 Hart et al.  
 2004/0071716 A1 4/2004 Jansen et al.  
 2004/0116321 A1 6/2004 Salesses et al.  
 2004/0116322 A1 6/2004 Yianakopoulos et al.  
 2004/0204337 A1 10/2004 Corona, III et al.  
 2004/0229769 A1 11/2004 Smith et al.  
 2005/0003980 A1 1/2005 Baker et al.  
 2005/0245668 A1 11/2005 Green et al.  
 2005/0256027 A1 11/2005 Heibel et al.  
 2006/0094639 A1 5/2006 Martin et al.  
 2006/0252669 A1 11/2006 Heibel et al.  
 2007/0099817 A1 5/2007 Smith et al.  
 2007/0275866 A1 11/2007 Dykstra  
 2007/0293413 A1 12/2007 McFarland et al.  
 2008/0076692 A1 3/2008 Carvell et al.  
 2008/0167453 A1 7/2008 Goettel et al.  
 2008/0295256 A1 12/2008 Broze et al.  
 2008/0312343 A1 12/2008 Braun et al.  
 2009/0062174 A1 3/2009 Green et al.  
 2010/0035791 A1 2/2010 Igarashi et al.  
 2010/0190679 A1 7/2010 Vanpachtenbeke et al.  
 2011/0245141 A1 10/2011 Gizaw et al.  
 2011/0269663 A1 11/2011 Clowes et al.  
 2011/0301312 A1 12/2011 Blondel  
 2012/0142578 A1 6/2012 Panandiker et al.  
 2013/0065813 A1 3/2013 Miravet Celades et al.  
 2013/0109612 A1 5/2013 Corona, III et al.  
 2013/0121944 A1 5/2013 Leyrer et al.  
 2013/0121945 A1 5/2013 Leyrer et al.  
 2013/0129657 A1 5/2013 Streuli  
 2013/0197101 A1 8/2013 Braun et al.  
 2013/0310300 A1 11/2013 Leyrer et al.  
 2013/0310301 A1 11/2013 Sivik et al.  
 2014/0047649 A1 2/2014 Blondel  
 2014/0315779 A1 10/2014 Zander  
 2014/0378639 A1 12/2014 Blondel et al.  
 2015/0191677 A1 7/2015 Blondel  
 2015/0197708 A1 7/2015 Jin  
 2015/0329799 A1 11/2015 Schramm, Jr. et al.  
 2015/0337239 A1 11/2015 Gonzalez de Cossio et al.  
 2016/0024426 A1 1/2016 Sivik et al.  
 2016/0024427 A1 1/2016 Sivik et al.  
 2016/0024428 A1 1/2016 Dykstra et al.  
 2016/0024429 A1 1/2016 Dykstra et al.  
 2016/0024430 A1 1/2016 Dykstra et al.  
 2016/0024431 A1 1/2016 Dykstra et al.  
 2016/0024432 A1 1/2016 Sivik et al.  
 2016/0024433 A1 1/2016 Sivik et al.  
 2016/0024434 A1 1/2016 Sivik et al.  
 2016/0032220 A1 2/2016 Sivik et al.  
 2017/0191002 A1 7/2017 Dykstra et al.

2017/0247637 A1 8/2017 Dykstra et al.  
 2017/0298295 A1 10/2017 Dykstra et al.  
 2017/0342345 A1 11/2017 Sivik et al.

## FOREIGN PATENT DOCUMENTS

EP 0 172 025 A2 2/1986  
 EP 0 172 723 A2 2/1986  
 EP 0 172 724 A2 2/1986  
 EP 0 343 840 A2 11/1989  
 EP 1 352 948 A1 10/2003  
 EP 1 625 195 B1 5/2007  
 EP 1 740 682 B1 6/2009  
 EP 1 756 168 B1 7/2009  
 EP 2 284 250 A1 2/2011  
 EP 1 781 717 B1 11/2012  
 FR 2862975 B1 2/2006  
 GB 2 002 400 A 2/1979  
 JP 2005082924 A 3/2005  
 JP 2012154010 A 8/2012  
 JP 2012158547 A 8/2012  
 JP 5034078 B2 9/2012  
 JP 5528660 B2 6/2014  
 KR 20150100549 A 9/2015  
 WO WO 96/07689 A1 3/1996  
 WO WO 99/20725 A1 4/1999  
 WO WO 02/057400 A2 7/2002  
 WO WO 03/002699 A1 1/2003  
 WO WO 03/102043 A1 12/2003  
 WO WO 2004/050812 A1 6/2004  
 WO WO 2004/061065 A1 7/2004  
 WO WO 2005/087907 A1 9/2005  
 WO WO 2005/097834 A2 10/2005  
 WO WO 2005/103215 A1 11/2005  
 WO WO 2008/005693 A2 1/2008  
 WO WO 2010/078959 A1 7/2010  
 WO WO 2010/079100 A1 7/2010  
 WO WO 2012/076432 A1 6/2012  
 WO WO 2013/068388 A1 5/2013  
 WO WO 2013/068394 A1 5/2013  
 WO WO 2013/142486 A1 9/2013  
 WO WO 2013/189010 A1 12/2013  
 WO WO 2015/130088 A1 9/2015

## OTHER PUBLICATIONS

International Search Report; International Application No. PCT/US2015/041656; dated Oct. 9, 2015; 10 pages.  
 International Search Report; International Application No. PCT/US2015/041657; dated Oct. 8, 2015; 11 pages.  
 International Search Report; International Application No. PCT/US2015/041658; dated Oct. 8, 2015; 11 pages.  
 International Search Report; International Application No. PCT/US2015/041659; dated Nov. 2, 2015; 15 pages.  
 International Search Report; International Application No. PCT/US2015/041737; dated Oct. 23, 2015; 10 pages.  
 International Search Report; International Application No. PCT/US2015/041741; dated Oct. 8, 2015; 11 pages.  
 International Search Report; International Application No. PCT/US2015/041640; dated Oct. 8, 2015; 11 pages.  
 International Search Report; International Application No. PCT/US2015/041641; dated Oct. 13, 2015; 10 pages.  
 International Search Report; International Application No. PCT/US2015/041642; dated Oct. 8, 2015; 11 pages.

## TREATMENT COMPOSITIONS

This is a continuation of U.S. patent application Ser. No. 14/806,685, filed Jul. 23, 2015, now abandoned, which claims the priority of U.S. Provisional Applications 62/027, 814, filed Jul. 23, 2014 and 62/083,927, filed Nov. 25, 2014.

## FIELD OF THE INVENTION

The present invention relates to treatment compositions and processes of making and using same.

## BACKGROUND OF THE INVENTION

Treatment compositions, such as fabric softener compositions, typically comprise benefit agents such as silicones, fabric softener actives, perfumes and perfume microcapsules. Generally there are tradeoffs associated with using multiple benefit agents in one treatment composition. Such tradeoffs include instability, as well as the loss or reduction of one or more of the benefit agents' benefits. A reduction in one of the benefit agent's levels can improve the performance of another benefit agent, yet the performance of the benefit agent that is being reduced suffers. In an effort to solve this dilemma, industry has turned to polymers. Current polymers systems can improve a treatment composition's stability but such improvement in stability comes with a decrease in freshness.

Applicants recognized that the traditional polymer system architecture was the source of the stability and freshness problems. In particular, Applicants recognized that traditional polymer systems did not contribute to the overall feel benefit that was desired. Applicants discovered that, for fabric softeners, in particular low pH fabric softeners, when a softener active reduction is coupled with the judicious selection of two polymers, one cross-linked and one with sufficient anionic monomer such that the polymer associates weakly enough with the softener vesicles to prevent phase separation but not so much to create aggregates that lead to phase separation, the composition's perfume effectiveness is improved, yet the perceived performance of softener active was surprisingly maintained. While not being bound by theory, Applicants believe that the proper selection of such polymers provides results in anionic carry over scavenging and a softener active that is in a more preferred state. Thus, the treated fabric's feel is maintained with less softener active.

## SUMMARY OF THE INVENTION

The present invention relates to treatment compositions containing polymer systems that provide stability and benefit agent deposition as well as methods of making and using same. Such treatment compositions may be used for example as through the wash and/or through the rinse fabric enhancers as well as unit dose treatment compositions.

## DETAILED DESCRIPTION OF THE INVENTION

## Definitions

As used herein, the term "fabric and home care product" is a subset of cleaning and treatment compositions that includes, unless otherwise indicated, granular or powder-form all-purpose or "heavy-duty" washing agents, especially cleaning detergents; liquid, gel or paste-form all-purpose

washing agents, especially the so-called heavy-duty liquid types; liquid fine-fabric detergents; hand dishwashing agents or light duty dishwashing agents, especially those of the high-foaming type; machine dishwashing agents, including the various tablet, granular, liquid and rinse-aid types for household and institutional use; liquid cleaning and disinfecting agents, including antibacterial hand-wash types, cleaning bars, car or carpet shampoos, bathroom cleaners including toilet bowl cleaners; and metal cleaners, fabric conditioning products including softening and/or freshening that may be in liquid, solid and/or dryer sheet form; as well as cleaning auxiliaries such as bleach additives and "stain-stick" or pre-treat types, substrate-laden products such as dryer added sheets, dry and wetted wipes and pads, nonwoven substrates, and sponges; as well as sprays and mists. All of such products which are applicable may be in standard, concentrated or even highly concentrated form even to the extent that such products may in certain aspect be non-aqueous.

As used herein "Polymer 1" is synonymous with "first polymer" and "Polymer 2" is synonymous with "second polymer".

As used herein, the term "situs" includes paper products, fabrics, garments and hard surfaces.

As used herein, articles such as "a", "an", and "the" when used in a claim, are understood to mean one or more of what is claimed or described.

Unless otherwise noted, all component or composition levels are in reference to the active level of that component or composition, and are exclusive of impurities, for example, residual solvents or by-products, which may be present in commercially available sources.

All percentages and ratios are calculated by weight unless otherwise indicated. All percentages and ratios are calculated based on the total composition unless otherwise indicated.

It should be understood that every maximum numerical limitation given throughout this specification includes every lower numerical limitation, as if such lower numerical limitations were expressly written herein. Every minimum numerical limitation given throughout this specification will include every higher numerical limitation, as if such higher numerical limitations were expressly written herein. Every numerical range given throughout this specification will include every narrower numerical range that falls within such broader numerical range, as if such narrower numerical ranges were all expressly written herein.

## Fabric Treatment Compositions

In one aspect, a composition comprising, based upon total composition weight:

a) from about 0.01% to about 1%, preferably from about 0.05% to about 0.75%, more preferably from about 0.075% to about 0.5% even more preferably from about 0.06% to about 0.3% of a polymeric material comprising:

- (i) a polymer derived from the polymerization of from about 5 to 98.5 mole percent of a cationic vinyl addition monomer, from about 1.5 to 95 mole percent of a non-ionic vinyl addition monomer, from about 50 ppm to 475 ppm of the composition of a cross-linking agent comprising three or more ethylenic functions and a chain transfer agent from about 0 to 10,000 ppm said polymer having a viscosity slope of from about 3.5 to about 12;
- (ii) a first polymer and a second polymer, preferably said first polymer and said second polymer being present in a ratio of about 1:5 to about 10:1, prefer-

ably, about 1:2 to about 5:1, more preferably about 1:1 to about 3:1, most preferably from about 3:2 to 5:1; said first polymer is derived from the polymerization of from about 5 to 100 mole percent of a cationic vinyl addition monomer, from about 0 to 95 mole percent of a non-ionic vinyl addition monomer, from about 50 ppm to 2,000 ppm, preferably from about 50 ppm to about 475 ppm, of a cross-linking agent comprising three or more ethylenic functions, 10 0 ppm to about 10,000 ppm chain transfer agent, preferably said first polymer has a viscosity slope >3.7

said second polymer being derived from the polymerization of from about 5 to 100 mole percent of 15 a cationic vinyl addition monomer, from about 0 to 95 mole percent of a non-ionic vinyl addition monomer, from about 0 ppm to 45 ppm of a cross-linking agent comprising two or more ethylenic functions, 0 ppm to about 10,000 ppm chain 20 transfer agent, preferably said second polymer has a viscosity slope <3.7; in one aspect said second polymer is a linear or branched, uncross-linked polyethyleneimine, preferably said polyethyleneimine is branched and uncross-linked; 25

(iii) a first polymer and a second polymer, preferably said first polymer and said second polymer being present in a ratio of about 1:5 to about 10:1, preferably, about 1:2 to about 5:1, more preferably about 1:1 to about 3:1, most preferably from about 3:2 to 30 5:1; said first polymer is derived from the polymerization of from about 5 to 100 mole percent of a cationic vinyl addition monomer, from about 0 to 95 mole percent of a non-ionic vinyl addition monomer, from about 310 ppm to 1,950 ppm of a cross-linking 35 agent comprising two or more ethylenic functions, 0 ppm to about 10,000 ppm chain transfer agent, preferably said first polymer has a viscosity slope >3.7;

said second polymer being derived from the polymerization of from about 5 to 100 mole percent of a cationic vinyl addition monomer, from about 0 to 95 mole percent of a non-ionic vinyl addition monomer, from about 0 ppm to 45 ppm of a cross-linking agent comprising two or more ethylenic functions, 0 ppm to about 10,000 ppm chain transfer agent, preferably said second polymer has a viscosity slope <3.7; in one aspect said second polymer is a linear or branched, uncross-linked polyethyleneimine, preferably said polyethyleneimine is branched and uncross-linked; 50

(iv) a first polymer and a second polymer, preferably said first polymer and said second polymer being present in a ratio of about 1:5 to about 10:1, preferably, about 1:2 to about 5:1, more preferably about 1:1 to about 3:1, most preferably from about 3:2 to 5:1; said first polymer is derived from the polymerization of from about 5 to 100 mole percent of a cationic vinyl addition monomer, from about 0 to 95 mole percent of a non-ionic vinyl addition monomer, 60 from about 50 ppm to 1,950 ppm of a cross-linking agent comprising two or more ethylenic functions, 0 ppm to about 10,000 ppm chain transfer agent, preferably said first polymer has a viscosity slope >3.7, with the proviso that said first polymer 65 does not comprise an acrylamide unit and/or a methacrylamide unit;

said second polymer being derived from the polymerization of from about 5 to 100 mole percent of a cationic vinyl addition monomer, from about 0 to 95 mole percent of a non-ionic vinyl addition monomer, from about 0 ppm to 45 ppm of a cross-linking agent comprising two or more ethylenic functions, 0 ppm to about 10,000 ppm chain transfer agent, preferably said second polymer has a viscosity slope <3.7; in one aspect said second polymer is a linear or branched, uncross-linked polyethyleneimine, preferably said polyethyleneimine is branched and uncross-linked;

(v) a first polymer and a second polymer, preferably said first polymer and said second polymer being present in a ratio of about 1:5 to about 10:1, preferably, about 1:2 to about 5:1, more preferably about 1:1 to about 3:1, most preferably from about 3:2 to 5:1; said first polymer is derived from the polymerization of from about 5 to 100 mole percent of a cationic vinyl addition monomer, from about 0 to 95 mole percent of a non-ionic vinyl addition monomer, from about 50 ppm to 1,950 ppm of a cross-linking agent comprising two or more ethylenic functions, 0 ppm to about 10,000 ppm chain transfer agent, preferably said first polymer has a viscosity slope >3.7;

said second polymer being derived from the polymerization of from about 5 to 100 mole percent of a cationic vinyl addition monomer, from about 0 to 95 mole percent of a non-ionic vinyl addition monomer, from about 1 ppm to 45 ppm of a cross-linking agent comprising two or more ethylenic functions, 0 ppm to about 10,000 ppm chain transfer agent, preferably said second polymer has a viscosity slope <3.7;

(vi) a first polymer and a second polymer, preferably said first polymer and said second polymer being present in a ratio of about 1:5 to about 10:1, preferably, about 1:2 to about 5:1, more preferably about 1:1 to about 3:1, most preferably from about 3:2 to 5:1; said first polymer is derived from the polymerization of from about 5 to 100 mole percent of a cationic vinyl addition monomer, from about 0 to 95 mole percent of a non-ionic vinyl addition monomer, from about 50 ppm to 1,950 ppm of a cross-linking agent comprising three or more ethylenic functions, 0 ppm to about 10,000 ppm chain transfer agent, preferably said first polymer has a viscosity slope >3.7

said second polymer being derived from the polymerization of from about 5 to 99 mole percent of a cationic vinyl addition monomer, from about 0 to 95 mole percent of a non-ionic vinyl addition monomer, from about 1 to 49 percent of an anionic vinyl addition monomer, with the proviso that the sum of the cationic vinyl addition monomer, non-ionic vinyl addition monomer, and anionic vinyl addition monomer will not exceed 100 mole percent; from about 0 ppm to 45 ppm of a cross-linking agent comprising two or more ethylenic functions, 0 ppm to about 10,000 ppm chain transfer agent, preferably said second polymer has a viscosity slope <3.7;

(vii) a polymer being derived from the polymerization of from about 5 to 99 mole percent of a cationic vinyl addition monomer, from about 0 to 95 mole percent of a non-ionic vinyl addition monomer, from about 1

to 49 percent of an anionic vinyl addition monomer, with the proviso that the sum of the cationic vinyl addition monomer, non-ionic vinyl addition monomer, and anionic vinyl addition monomer will not exceed 100 mole percent; from about 50 ppm to 2,000 ppm of a cross-linking agent comprising two or more ethylenic functions, 0 ppm to about 10,000 ppm chain transfer agent, preferably said first polymer has a viscosity slope  $>3.7$ ;

(viii) a polymer derived from the polymerization of from about 5 to 100 mole percent of a cationic vinyl addition monomer, from about 0 to 95 mole percent of a non-ionic vinyl addition monomer, from about 515 ppm to 4,975 ppm of a cross-linking agent comprising two or more ethylenic functions, a weight percent water soluble fraction greater than or equal to 25 weight percent and 0 ppm to about 10,000 ppm of a chain transfer agent, and

(v) mixtures thereof;

b.) from about 0% to about 35%, preferably from about 1% to about 35%, more preferably from about 2% to about 25%, more preferably from about 3% to about 20%, more preferably from about 5% to about 15%, most preferably from about 8% to about 12% of a fabric softener active,

said composition being a fabric and home care product, is disclosed.

In one aspect of said composition, said polymeric material comprises:

a.) a polymer derived from the polymerization of from about 10 to 95 mole percent, preferably 20 to 90 mole percent, more preferably 30 to 75 mole percent, most preferably 45 to 65 mole percent of a cationic vinyl addition monomer; from about 5 to 90 mole percent of a non-ionic vinyl addition monomer; preferably 10 to 80 mole percent from about 60 ppm to 450 ppm of the composition of a cross-linking agent comprising three or more ethylenic functions; 0 to 10,000 ppm, preferably 75 ppm to 400 ppm, of a chain transfer agent; said polymer having a viscosity slope of from about 3.5 to 40 about 12;

b.) a first polymer and a second polymer, said first polymer being derived from the polymerization of from about 10 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 to 80 mole percent, of a non-ionic vinyl addition monomer; from about 60 ppm to 1,900 ppm of a cross-linking agent comprising three or more ethylenic functions; 0 ppm to about 10,000 ppm, preferably 75 ppm to 1,800 ppm, of a chain transfer agent; preferably said first polymer has a viscosity slope  $>3.7$  said second polymer being derived from the polymerization of from about 10 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 to 80 mole percent, of a non-ionic vinyl addition monomer; 0 ppm to 40 ppm, preferably 0 ppm to 20 ppm, of a cross-linking agent comprising two or more ethylenic functions; 0 ppm to about 10,000 ppm chain transfer agent; preferably said second polymer has a viscosity slope  $<3.7$ ;

c.) a first polymer and a second polymer, said first polymer being derived from the polymerization of from

about 10 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 mole percent to 80 mole percent, of a non-ionic vinyl addition monomer; from about 325 ppm to 1,900 ppm, preferably 350 ppm to 1,800 ppm, of a cross-linking agent comprising two or more ethylenic functions; 0 ppm to about 10,000 ppm chain transfer agent; preferably said first polymer has a viscosity slope  $>3.7$ ;

said second polymer being derived from the polymerization of from about 10 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 mole to 80 mole percent, of a non-ionic vinyl addition monomer; 0 ppm to 40 ppm, preferably 0 ppm to 20 ppm, of a cross-linking agent comprising two or more ethylenic functions; 0 ppm to about 10,000 ppm chain transfer agent; preferably said second polymer has a viscosity slope  $<3.7$ ;

d.) a first polymer and a second polymer, said first polymer being derived from the polymerization of from about 10 to 95 mole, preferably 20 to 90 mole percent more preferably 30 to 75 mole percent, most preferably 45 to 65 mole percent of a cationic vinyl addition monomer; from about 5 to 90 mole percent, preferably 10 mole percent to 80 mole percent, of a non-ionic vinyl addition monomer; from about 60 ppm to 1,900 ppm, preferably 75 to 1,800 ppm, of a cross-linking agent comprising two or more ethylenic functions; 0 ppm to about 10,000 ppm chain transfer agent; preferably said first polymer has a viscosity slope  $>3.7$ , with the proviso that said first polymer does not comprise an acrylamide unit;

said second polymer being derived from the polymerization of from about 10 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 to 80 mole percent, of a non-ionic vinyl addition monomer; 0 ppm to 40 ppm, preferably 0 ppm to 20 ppm, of a cross-linking agent comprising two or more ethylenic functions; 0 ppm to about 10,000 ppm chain transfer agent; preferably said second polymer has a viscosity slope  $<3.7$ ;

e.) a first polymer and a second polymer, said first polymer being derived from the polymerization of from about 10 to 95 mole, preferably 20 to 90 mole percent more preferably 30 to 75 mole percent, most preferably 45 to 65 mole percent of a cationic vinyl addition monomer; from about 5 to 90 mole percent, preferably 10 mole percent to 80 mole percent, of a non-ionic vinyl addition monomer; from about 55 ppm to 1,900 ppm, preferably 60 ppm to 1,800 ppm, of a cross-linking agent comprising two or more ethylenic functions; 0 ppm to about 10,000 ppm chain transfer agent; preferably said first polymer has a viscosity slope  $>3.7$ ; said second polymer being derived from the polymerization of from about 10 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 mole percent to 80 mole percent, of a non-ionic vinyl

- addition monomer; from about 1 ppm to 40 ppm, preferably 1 ppm to 20 ppm, of a cross-linking agent comprising two or more ethylenic functions; 0 ppm to about 10,000 ppm chain transfer agent; preferably said second polymer has a viscosity slope  $<3.7$ ;
- f.) a first polymer and a second polymer, said first polymer being derived from the polymerization of from about 10 to 95 mole percent, preferably 20 to 90 mole percent more preferably 30 to 75 mole percent, most preferably 45 to 65 mole percent of a cationic vinyl addition monomer; from about 10 to 90 mole percent, preferably 20 to 80 mole percent, of a non-ionic vinyl addition monomer; from about 55 ppm to 1,900 ppm, preferably 60 ppm to 1,800 ppm, of a cross-linking agent comprising three or more ethylenic functions; 0 ppm to about 10,000 ppm chain transfer agent; preferably said first polymer has a viscosity slope  $>3.7$
- said second polymer being derived from the polymerization of from about 10 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 to 80 mole percent, of a non-ionic vinyl addition monomer; from about 1 to 45 mole percent, preferably 1 to 40 mole percent, of an anionic vinyl addition monomer; with the proviso that the sum of the cationic vinyl addition monomer, non-ionic vinyl addition monomer, and anionic vinyl addition monomer will not exceed 100 mole percent; 0 ppm to 40 ppm, preferably 0 ppm to 20 ppm, of a cross-linking agent comprising two or more ethylenic functions; 0 ppm to about 10,000 ppm chain transfer agent; preferably said second polymer has a viscosity slope  $<3.7$ ;
- g.) a polymer being derived from the polymerization of from about 5 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 to 80 mole percent, of a non-ionic vinyl addition monomer; from about 1 to 45 mole percent, preferably 1 to 40 mole percent, of an anionic vinyl addition monomer; with the proviso that the sum of the cationic vinyl addition monomer, non-ionic vinyl addition monomer, and anionic vinyl addition monomer will not exceed 100 mole percent; from about 55 ppm to 1,900 ppm, preferably 60 ppm to 1,800 ppm, of a cross-linking agent comprising two or more ethylenic functions; 0 ppm to about 10,000 ppm chain transfer agent; preferably said first polymer has a viscosity slope  $>3.7$ ;
- h.) a polymer derived from the polymerization of from about 10 to 95 mole percent, preferably 20 to 90 mole percent more preferably 30 to 75 mole percent, most preferably 45 to 65 mole percent of a cationic vinyl addition monomer; from about 5 to 90 mole percent, preferably 10 to 80 mole percent, of a non-ionic vinyl addition monomer; from about 525 ppm to 4,900 ppm, preferably 550 ppm to 4,800 ppm, of a cross-linking agent comprising two or more ethylenic functions; a weight percent water soluble fraction greater than or equal to 28 weight percent, and 0 ppm to about 10,000 ppm of a chain transfer agent. In one aspect of said composition, said fabric softener active is selected from the group consisting of a quaternary ammonium com-

pound, a silicone polymer, a polysaccharide, a clay, an amine, a fatty ester, a dispersible polyolefin, a polymer latex and mixtures thereof.

In one aspect of said composition:

- a.) said quaternary ammonium compound comprises an alkyl quaternary ammonium compound, preferably said alkyl quaternary ammonium compound is selected from the group consisting of a monoalkyl quaternary ammonium compound, a dialkyl quaternary ammonium compound, a trialkyl quaternary ammonium compound and mixtures thereof;
- b.) said silicone polymer is selected from the group consisting of cyclic silicones, polydimethylsiloxanes, aminosilicones, cationic silicones, silicone polyethers, silicone resins, silicone urethanes, and mixtures thereof;
- c.) said polysaccharide comprises a cationic starch;
- d.) said clay comprises a smectite clay;
- e.) said dispersible polyolefin is selected from the group consisting of polyethylene, polypropylene and mixtures thereof; and
- f.) said fatty ester is selected from the group consisting of a polyglycerol ester, a sucrose ester, a glycerol ester and mixtures thereof.

In one aspect of said composition, said fabric softener active comprises a material selected from the group consisting of monoesterquats, diesterquats, triesterquats, and mixtures thereof. Preferably, said monoesterquats and diesterquats are selected from the group consisting of bis-(2-hydroxypropyl)-dimethylammonium methylsulfate fatty acid ester and isomers of bis-(2-hydroxypropyl)-dimethylammonium methylsulfate fatty acid ester and/or mixtures thereof, 1,2-di(acyloxy)-3-trimethylammoniopropane chloride, N,N-bis(stearoyl-oxy-ethyl)-N,N-dimethyl ammonium chloride, N,N-bis(tallowoyl-oxy-ethyl)-N,N-dimethyl ammonium chloride, N,N-bis(stearoyl-oxy-ethyl)-N-(2-hydroxyethyl)-N-methyl ammonium methylsulfate, N,N-bis(stearoyl-2-hydroxypropyl)-N,N-dimethylammonium methylsulfate, N,N-bis-(tallowoyl-2-hydroxypropyl)-N,N-dimethylammonium methylsulfate, N,N-bis-(palmitoyl-2-hydroxypropyl)-N,N-dimethylammonium methylsulfate, N,N-bis(stearoyl-2-hydroxypropyl)-N,N-dimethylammonium chloride, 1,2-di-(stearoyl-oxy)-3-trimethyl ammonium chloride, dicanoladimethylammonium chloride, di(hard)tallowdimethylammonium chloride, dicanoladimethylammonium methylsulfate, 1-methyl-1-stearoylamidoethyl-2-stearoylimidazolinium methylsulfate, 1-tallowylamidoethyl-2-tallowylimidazoline, dipalmylmethyl hydroxyethylammonium methylsulfate and mixtures thereof.

In one aspect of said composition, said fabric softening active has an Iodine Value of between 0-140, preferably 5-100, more preferably 10-80, even more preferably 15-70, even more preferably 18-60, most preferably 18-25. When partially hydrogenated fatty acid quaternary ammonium compound softener is used, most preferably range is 25-60.

In one aspect of said composition, said composition comprising a quaternary ammonium compound and a silicone polymer, preferably from about 0.001% to about 10%, from about 0.1% to about 8%, more preferably from about 0.5% to about 5%, of said silicone polymer.

In one aspect of said composition, said composition comprises, in addition to said fabric softener active, from about 0.001% to about 5%, preferably from about 0.1% to about 3%, more preferably from about 0.2% to about 2% of a stabilizer that comprises a alkyl quaternary ammonium compound, preferably said alkyl quaternary ammonium

compound comprises a material selected from the group consisting of a monoalkyl quaternary ammonium compound, a dialkyl quaternary ammonium compound, a trialkyl quaternary ammonium compound and mixtures thereof, more preferably said alkyl quaternary ammonium compound comprises a monoalkyl quaternary ammonium compound and/or di-alkyl quaternary ammonium compound.

In one aspect of said composition, said polymer is derived from

- a.) a monomer selected from the group consisting of  
(i) a cationic monomer according to formula (I):



wherein:

- R<sub>1</sub> is chosen from hydrogen, or C<sub>1</sub>-C<sub>4</sub> alkyl;  
R<sub>2</sub> is chosen from hydrogen or methyl;  
R<sub>3</sub> is chosen from C<sub>1</sub>-C<sub>4</sub> alkylene;  
R<sub>4</sub>, R<sub>5</sub>, and R<sub>6</sub> are each independently chosen from hydrogen, C<sub>1</sub>-C<sub>4</sub> alkyl, C<sub>1</sub>-C<sub>4</sub> alkyl alcohol or C<sub>1</sub>-C<sub>4</sub> alkoxy;  
X is chosen from —O—, or —NH—; and  
Y is chosen from Cl, Br, I, hydrogensulfate or methylsulfate.

- (ii) a non-ionic monomer having formula (II)



wherein:

- R<sub>7</sub> is chosen from hydrogen or C<sub>1</sub>-C<sub>4</sub> alkyl;  
R<sub>8</sub> is chosen from hydrogen or methyl;  
R<sub>9</sub> and R<sub>10</sub> are each independently chosen from hydrogen, C<sub>1</sub>-C<sub>30</sub> alkyl, C<sub>1</sub>-C<sub>4</sub> alkyl alcohol or C<sub>1</sub>-C<sub>4</sub> alkoxy,

- (iii) an anionic monomer selected from the group consisting of acrylic acid, methacrylic acid, itaconic acid, crotonic acid, maleic acid, fumaric acid, as well as monomers performing a sulfonic acid or phosphonic acid functions, such as 2-acrylamido-2-methyl propane sulfonic acid, and their salts.

- b.) wherein said cross-linking agent is selected from the group consisting of methylene bisacrylamide, ethylene glycol diacrylate, polyethylene glycol dimethacrylate, diacryamide, triallylamine, cyanomethylacrylate, vinyl oxyethylacrylate or methacrylate and formaldehyde, glyoxal, divinylbenzene, tetraallylammonium chloride, allyl acrylates, allyl methacrylates, diacrylates and dimethacrylates of glycols or polyglycols, butadiene, 1,7-octadiene, allylacrylamides or allylmethacrylamides, bisacrylamidoacetic acid, N,N'-methylenebisacrylamide or polyol polyallyl ethers, pentaerythritol triacrylate, pentaerythritol tetraacrylate, 1,1,1-trimethylolpropane tri(meth)acrylate; and tri- and tetramethacrylates of polyglycols; or polyol polyallyl ethers such as polyallyl sucrose or pentaerythritol tri-

allyl ether, ditrimethylolpropane tetraacrylate, pentaerythritol tetramethacrylate, pentaerythritol triacrylate ethoxylate, triethanolamine trimethacrylate, 1,1,1-trimethylolpropane triacrylate, 1,1,1-trimethylolpropane triacrylate ethoxylate, trimethylolpropane tris(polyethylene glycol ether) triacrylate, 1,1,1-trimethylolpropane trimethacrylate, tris-(2-hydroxyethyl)-1,3,5-triazine-2,4,6-trione triacrylate, tris-(2-hydroxyethyl)-1,3,5-triazine-2,4,6-trione trimethacrylate, dipentaerythritol pentaacrylate, 3-(3-[[dimethyl-(vinyl)-silyl]-oxy]-1,1,5,5-tetramethyl-1,5-divinyl-3-trisoxanyl)-propyl methacrylate, dipentaerythritol hexaacrylate, 1-(2-propenyl-oxo)-2,2-bis[(2-propenyl-oxo)-methyl]-butane, trimethacrylic acid-1,3,5-triazin-2,4,6-triyltri-2,1-ethandiyl ester, glycerine triacrylate, propoxylated, 1,3,5-triacryloylhexahydro-1,3,5-triazine, 1,3-dimethyl-1,1,3,3-tetravinylsiloxane, pentaerythritol tetravinyl ether, 1,3-dimethyl-1,1,3,3-tetravinylsiloxane, (Ethoxy)-trivinylsilane, (Methyl)-trivinylsilane, 1,1,3,5,5-pentamethyl-1,3,5-trivinyltrisiloxane, 1,3,5-trimethyl-1,3,5-trivinylcyclotrisilazane, 2,4,6-trimethyl-2,4,6-trivinylcyclotrisiloxane, 1,3,5-trimethyl-1,3,5-trivinyltrisilazane, tris-(2-butanone oxime)-vinylsilane, 1,2,4-trivinylcyclohexane, trivinylphosphine, trivinylsilane, methyltrivinylsilane, pentaerythritol triallyl ether, phenyltrivinylsilane, triallylamine, triallyl citrate, triallyl phosphate, triallylphosphine, triallyl phosphite, triallylsilane, 1,3,5-triallyl-1,3,5-triazine-2,4,6(1H,3H,5H)-trione, trimellitic acid triallyl ester, trimethallyl isocyanurate, 2,4,6-tris-(allyloxy)-1,3,5-triazine, 1,2-Bis-(diallylarnino)-ethane, pentaerythritol tetratallate, 1,3,5,7-tetravinyl-1,3,5,7-tetramethylcyclotetrasiloxane, 1,3,5,7-tetravinyl-1,3,5,7-tetramethylcyclotetrasiloxane, tris-[2-acryloyloxy]-ethyl]-phosphate, vinylboronic anhydride pyridine, 2,4,6-trivinylcyclotriboroxanepyridine, tetraallylsilane, tetraallyloxysilane, 1,3,5,7-tetramethyl-1,3,5,7-tetravinylcyclotetrasilazane the ethoxylated compounds thereof and mixtures thereof

- c.) wherein said chain transfer agent is selected from the group consisting of mercaptanes, malic acid, lactic acid, formic acid, isopropanol and hypophosphites, and mixtures thereof.

In one aspect of said composition, said the cationic monomers are selected from the group consisting of methyl chloride quaternized dimethyl aminoethylammonium acrylate, methyl chloride quaternized dimethyl aminoethylammonium methacrylate and mixtures thereof, and the non-ionic monomers are selected from the group consisting of acrylamide, dimethyl acrylamide and mixtures thereof.

In one aspect of said composition, said composition has a Brookfield viscosity of from about 20 cps to about 1000 cps, preferably from 30 cps to about 500 cps, and most preferably 40 cps to about 300 cps.

In one aspect of said composition, said composition comprises an adjunct material selected from the group consisting of surfactants, builders, chelating agents, dye transfer inhibiting agents, dispersants, enzymes, and enzyme stabilizers, catalytic materials, bleach activators, hydrogen peroxide, sources of hydrogen peroxide, preformed peracids, polymeric dispersing agents, clay soil removal/anti-redeposition agents, brighteners, suds suppressors, dyes, hueing dyes, perfumes, perfume delivery systems, structure elasticizing agents, carriers, structurants, hydrotropes, processing aids, solvents and/or pigments and mixtures thereof.

## 11

In one aspect of said composition, said composition comprises perfume and/or a perfume delivery system, preferably said perfume delivery system comprises perfume microcapsules, preferably said perfume microcapsules comprises a cationic coating.

In one aspect of said composition, said composition comprises one or more types of perfume microcapsules.

In one aspect of said composition, said composition has a pH from about 2 to about 4, preferably from about 2.4 to about 3.6.

In one aspect the viscosity slope of any of the embodiments of Applicants' compositions that are claimed and/or disclosed is determined using Viscosity Slope Method 1, preferably viscosity slope of any of the embodiments of Applicants' compositions that are claimed and/or disclosed is determined using Viscosity Slope Method 2.

## The First and Second Polymer

Applicants recognized that traditional polymer architecture can be a source of finished product stability and dosage problems. While not being bound by theory, Applicants believe the proper selection of one or more polymers yields a stable colloidal glass comprised of linear polymers capable of entangling and crosslinked polymers that generally cannot entangle. The aforementioned polymers enable the colloidal glass formation, as the crosslinked polymers' interactions provide stability while the linear polymers interaction with the crosslinked polymers allows for the desired benefit agent deposition. Thus, fabric treatment compositions comprising such particles have a surprising combination of stability and active deposition efficiency. Such treatment compositions provide benefits such as fabric feel, antistatic, and freshness.

Here, Applicants recognized that further benefit improvements were needed, such as fabric feel (e.g., softness) and freshness; however, one approach of formulating higher and higher levels of Polymer 1 could lead to unwanted changes to finished product (FP) rheology, such as viscosity growth which could lead to increased product residue or modified aesthetics. Applicants also recognized that increasing levels of Polymer 1 tended to decrease freshness. While not being bound by theory, Applicants believe the higher level of Polymer 1 can suppress the release of perfume from the situs (e.g., cotton terry), especially when higher level of Polymer 1 is combined with relatively high levels of softening actives. The Applicants recognized that the judicious selection of Polymer 2 will achieve the desired benefits. The proper selection of Polymer 2 includes the selection of polymer architectural parameters, such as monomers, charge density, lack of cross-linking and molecular weight. The Applicants recognized that obtaining the desired increase in benefits (e.g., freshness) requires the selection of individual and combined polymer levels, the ratio of Polymer 1 to Polymer 2, and level of softening actives when the other selections are taken into account. While not being bound by theory, Applicants believe that the mass of material that will be delivered to a fabric by a fabric softener along with residual detergent materials on the fabric should be taken into account when designing a fabric softener.

Applicants found that selection of Polymer 2 to maximize benefits, such as freshness, could result in a return of stability problems addressed by the selection criteria for Polymer 1. The Applicants discovered a solution to this problem by also selecting Polymer 1 with a preferred viscosity slope (VS) value.

## Polymer 1 Level:

The level of Polymer 1 in finished product (FP) is selected to achieve the desired properties of the FP, which include but

## 12

are not limited to FP with preferred a) phase stability, b) rheology, c) freshness benefit and d) softness benefit. Without wishing to be bound by theory, the preferred level of Polymer 1 is necessary to provide structure to the finished product. Such structure enables for example particle-based benefit actives (e.g., perfume microcapsules (PMC)) to be suspended in the FP. In addition, a preferred level of Polymer 1 minimizes the risk of product instability, which can be manifested in phase splitting, which can lead to poor product aesthetics and uneven distribution of benefit actives. In addition, Polymer 1 can improve the deposition of benefit actives, leading to improved freshness and softness. Such deposition improvement can involve carry-over anionic surfactant from the wash to form flocculates that lead to improved fabric deposition of benefit actives. The selection of Polymer 1 as described in the present inventions provides for a preferred FP viscosity slope (VS). It has surprisingly been found that preferred VS values enable improved FP phase stability, including when Polymer 1 is combined with Polymer 2.

A preferred level of Polymer 1 is from about 0.01% to about 1%, preferably from about 0.02% to about 0.5%, more preferably from about 0.03% to about 0.2%, even more preferably from about 0.06% to about 0.1%. However, in one aspect when the softener active level is less than 5% by weight of FP, a preferred level of Polymer 1 is from about 0.01% to about 1%, preferably from about 0.02% to about 0.5%.

## Polymer 2 Level:

The level of Polymer 2 in finished product (FP) is selected to achieve the desired properties of the FP, which include but are not limited to FP with preferred a) phase stability, b) rheology, c) freshness benefit and d) softness benefit. Without wishing to be bound by theory, the preferred level of Polymer 2 minimizes the risk of high levels of Polymer 1 causing unwanted FP viscosity growth, which can lead to changes in product aesthetics and/or difficulty in FP pouring, dispensing and/or dispersion. Without wishing to be bound by theory, Polymer 2 can improve perfume system efficiency by enhancing perfume release to the headspace above the fabric, resulting in greater scent intensity and noticeability. The lower molecular weight and lower degree of cross-linking of Polymer 2 in comparison to Polymer 1 is necessary to enabling the improved release of perfume from the situs and/or from the perfume delivery technology (e.g., PMC). In addition, the preferred amount of Polymer 2 alone in the compositions of the present invention enables improved freshness. Selecting too low a concentration of polymer can yield minimal benefits, whereas too high a concentration of polymer can also reduce benefits. Without being bound by theory, it is believed that too much polymer leads to suppression of perfume release, in which perfume is not released in a timely manner, leading to lower intensity and inefficient and cost ineffective perfume formulations.

A preferred level of Polymer 2 is from about 0.01% to about 1%, preferably from about 0.02% to about 0.5%, more preferably from about 0.04% to about 0.3%, even more preferably from about 0.06% to about 0.2%.

## Total Level of Polymer 1 and Polymer 2:

The total level of Polymer 1 and Polymer 2 in finished product (FP) is selected to achieve the desired properties of the FP, which include those described for Polymer 1 and Polymer 2 above. Selecting too low a concentration of polymer can yield minimal benefits, whereas too high a concentration of polymer can also reduce benefits. Without being bound by theory, it is believed that too much polymer leads to suppression of perfume release, in which perfume is

not released in a timely manner, leading to lower intensity and inefficient and cost ineffective perfume formulations.

A preferred total level of Polymer 1 and Polymer 2 is from about 0.01% to about 1%, preferably from about 0.05% to about 0.75%, more preferably from about 0.075% to about 0.5%, more preferably from about 0.075% to about 0.4%, even more preferably from about 0.06% to about 0.3%.

Ratio of Polymer 1 to Polymer 2:

The ratio of Polymer 1 to Polymer 2 in finished product (FP) is selected to achieve the desired properties of the FP, which include those described for Polymer 1 and Polymer 2 above. It was surprisingly found that selecting too high a ratio of Polymer 1 to Polymer 2 reduces the freshness benefit, whereas selecting too low a ratio of Polymer 1 to Polymer 2 results in poor FP stability. For example, in one embodiment the ratio of Polymer 1 to Polymer 2 is from about 1:5 to about 10:1, preferably, about 1:2 to about 5:1, even more preferably about 1:1 to about 3:1, most preferably from about 3:2 to 5:1.

In some embodiments of the present invention, the freshness benefit is reduced when the ratio of Polymer 1 to Polymer 2 is 100:1 or less (i.e., nil Polymer 2), and is also reduced when the ratio of Polymer 1 to Polymer 2 is 1:1. One such embodiment is when the total level of Polymer 1 and Polymer 2 in the composition of the present invention is from about 0.06% to about 0.3%.

Polymer 2 Molecular Weight:

In another aspect, the polymer comprises a Weight Average Molecular Weight (Mw) from about 5,000 Daltons to about 1,000,000 Daltons, preferably from about 10,000 Daltons to about 1,000,000 Daltons, more preferably from about 25,000 Daltons to about 600,000 Daltons, more preferably from about 50,000 Daltons to about 450,000 Daltons, more preferably from about 100,000 Daltons to about 350,000 Daltons, most preferably from about 150,000 Daltons to about 350,000 Daltons; in other aspect from about 25,000 Daltons to about 150,000 Daltons.

The molecular weight can also be correlated to the k value of the polymer. In one aspect the k value is from about 10 to 100, preferably from about 15 to 60, preferably from about 20 to 60, more preferably from about 20 to 55, more preferably from about 25 to 55, more preferably from about 25 to 45, most preferably from 30 to 45; in other aspect the k value is from about 15 to 30.

Polymer 1 Molecular Weight:

In another aspect, Polymer 1 comprises a Weight Average Molecular Weight (Mw) from about 500,000 Daltons to about 15,000,000 Daltons, preferably from about 1,000,000 Daltons to about 6,000,000 Daltons, more preferably from about 2,000,000 to 4,000,000.

In another embodiment, when Polymer 1 is cross-linked with one or more cross-linking agents, Polymer 1 may consist of a mixture of polymers with different degrees of cross-linking, including polymers that are highly cross-linked and polymer that are essentially non-cross-linked. Without being bound by theory, cross-linked polymers are more water insoluble, whereas non-cross-linked polymers are more water soluble. In one embodiment, Polymer 1 consists of a fraction of water soluble (non-cross-linked) and a fraction of water insoluble (cross-linked) polymers. In one embodiment, Polymer 1 has a weight percent water soluble fraction of from about 0.1% to 80%, preferably from about 1% to 60%, more preferably from 10% to 40%, most preferably from 25% to 35%. In another embodiment, Polymer 1 has a weight percent water soluble fraction of from 5% to 25%. Without being bound by theory, the Weight Average Molecular Weights (Mw) of the soluble and

insoluble fractions of Polymer 1 are similar (i.e., both are within the Mw range for Polymer 1).

In still another embodiment, Polymer 1 comprises a Weight Average Molecular Weight (Mw) from about 5 times to about 100 times the Weight Average Molecular Weight (Mw) of Polymer 2, preferably from about 10 times to about 50 times, more preferably from about 20 times to about 40 times, wherein Polymer 2 comprises a Weight Average Molecular Weight (Mw) from about 50,000 Daltons to about 150,000 Daltons.

In one aspect, Applicants disclose a composition comprising, based upon total composition weight:

a. Polymer 1 with a Weight Average Molecular Weight (Mw) from about 500,000 Daltons to about 15,000,000 Daltons, preferably from about 1,000,000 to about 6,000,000 Daltons.

b. Optionally, Polymer 1 has a weight percent water soluble fraction of from about 1% to about 60%.

c. Polymer 1 is present in the composition from about 0.01% to about 0.5%, preferably from about 0.03% to about 0.2%.

d. Polymer 2 has a Weight Average Molecular Weight (Mw) from about 5,000 Daltons to about 500,000 Daltons, preferably from about 10,000 Daltons to about 500,000 Daltons, preferably from about 25,000 to 350,000, most preferably from about 50,000 to about 250,000 Daltons. Alternatively, Polymer 2 may have a K value of from about 15 to 100, preferably from about 20 to 60, more preferably from about 30 to 45.

e. Polymer 2 is present in the composition from about 0.01 to about 0.5%, preferably from about 0.03% to about 0.3%.

f. Optionally, the weight ratio of Polymer 1 to Polymer 2 is from about 1:5 to about 5:1, preferably from about 1:3 to about 3:1.

g. Optionally, a weight ratio of fabric softener active from about 3 percent to about 13 weight percent, more preferably from about 5 to about 10 weight percent, most preferably from about 7 to about 9 weight percent.

Preferably said composition has a Brookfield viscosity of from about 20 cps to about 1000 cps, preferably from about 30 cps to about 500 cps, more preferably from about 40 cps to about 300 cps, most preferably from about 50 cps to about 150 cps.

45 Polymer 1 and Polymer 2 Viscosity Slope

Preferably said first polymer and said second polymer when combined have a viscosity slope of greater than or equal to 3, preferably greater than or equal to 3.8, more preferably from about 4.0 to about 12, even more preferably from about 4.0 to about 6.0 or from about 4.0 to about 5.0.

50 Suitable Fabric Softening Actives

The fluid fabric enhancer compositions disclosed herein comprise a fabric softening active ("FSA"). Suitable fabric softening actives, include, but are not limited to, materials selected from the group consisting of quaternary ammonium compounds, amines, fatty esters, sucrose esters, silicones, dispersible polyolefins, clays, polysaccharides, fatty acids, softening oils, polymer latexes and mixtures thereof.

Non-limiting examples of water insoluble fabric care 60 benefit agents include dispersible polyethylene and polymer latexes. These agents can be in the form of emulsions, latexes, dispersions, suspensions, and the like. In one aspect, they are in the form of an emulsion or a latex. Dispersible polyethylenes and polymer latexes can have a wide range of particle size diameters ( $\chi_{50}$ ) including but not limited to from about 1 nm to about 100  $\mu\text{m}$ ; alternatively from about 10 nm to about 10  $\mu\text{m}$ . As such, the particle sizes of

## 15

dispersible polyethylenes and polymer latexes are generally, but without limitation, smaller than silicones or other fatty oils.

Generally, any surfactant suitable for making polymer emulsions or emulsion polymerizations of polymer latexes can be used to make the water insoluble fabric care benefit agents of the present invention. Suitable surfactants consist of emulsifiers for polymer emulsions and latexes, dispersing agents for polymer dispersions and suspension agents for polymer suspensions. Suitable surfactants include anionic, cationic, and nonionic surfactants, or combinations thereof. In one aspect, such surfactants are nonionic and/or anionic surfactants. In one aspect, the ratio of surfactant to polymer in the water insoluble fabric care benefit agent is about 1:100 to about 1:2; alternatively from about 1:50 to about 1:5, respectively. Suitable water insoluble fabric care benefit agents include but are not limited to the examples described below.

Quats—Suitable quats include but are not limited to, materials selected from the group consisting of ester quats, amide quats, imidazoline quats, alkyl quats, amidoester quats and mixtures thereof. Suitable ester quats include but are not limited to, materials selected from the group consisting of monoester quats, diester quats, triester quats and mixtures thereof. In one aspect, a suitable ester quat is bis-(2-hydroxypropyl)-dimethylammonium methylsulfate fatty acid ester having a molar ratio of fatty acid moieties to amine moieties of from 1.85 to 1.99, an average chain length of the fatty acid moieties of from 16 to 18 carbon atoms and an iodine value of the fatty acid moieties, calculated for the free fatty acid, which has an Iodine Value of between 0-140, preferably 5-100, more preferably 10-80, even more preferably 15-70, even more preferably 18-55, most preferably 18-25. When a soft tallow quaternary ammonium compound softener is used, most preferably range is 25-60. In one aspect, the cis-trans-ratio of double bonds of unsaturated fatty acid moieties of the bis (2 hydroxypropyl)-dimethylammonium methylsulfate fatty acid ester is from 55:45 to 75:25, respectively. Suitable amide quats include but are not limited to, materials selected from the group consisting of monoamide quats, diamide quats and mixtures thereof. Suitable alkyl quats include but are not limited to, materials selected from the group consisting of mono alkyl quats, dialkyl quats, trialkyl quats, tetraalkyl quats and mixtures thereof.

Amines—Suitable amines include but are not limited to, materials selected from the group consisting of amidoesteramines, amidoamines, imidazoline amines, alkyl amines, amidoester amines and mixtures thereof. Suitable ester amines include but are not limited to, materials selected from the group consisting of monoester amines, diester amines, triester amines and mixtures thereof. Suitable amido quats include but are not limited to, materials selected from the group consisting of monoamido amines, diamido amines and mixtures thereof. Suitable alkyl amines include but are not limited to, materials selected from the group consisting of mono alkylamines, dialkyl amines quats, trialkyl amines, and mixtures thereof.

In one embodiment, the fabric softening active is a quaternary ammonium compound suitable for softening fabric in a rinse step. In one embodiment, the fabric softening active is formed from a reaction product of a fatty acid and an aminoalcohol obtaining mixtures of mono-, di-, and in one embodiment, tri-ester compounds. In another embodiment, the fabric softening active comprises one or more softener quaternary ammonium compounds such, but not limited to, as a monoalkyquaternary ammonium compound,

## 16

dialkylquaternary ammonium compound, a diamido quaternary compound, a diester quaternary ammonium compound, or a combination thereof.

In one aspect, the fabric softening active comprises a diester quaternary ammonium or protonated diester ammonium (hereinafter “DQA”) compound composition. In certain embodiments of the present invention, the DQA compound compositions also encompass diamido fabric softening actives and fabric softening actives with mixed 10 amido and ester linkages as well as the aforementioned diester linkages, all herein referred to as DQA.

In one aspect, said fabric softening active may comprise, as the principal active, compounds of the following formula:



wherein each R comprises either hydrogen, a short chain C<sub>1</sub>-C<sub>6</sub>, in one aspect a C<sub>1</sub>-C<sub>3</sub> alkyl or hydroxyalkyl group, for example methyl, ethyl, propyl, hydroxyethyl, and the like, poly(C<sub>2-3</sub> alkoxy), polyethoxy, benzyl, or mixtures thereof; each X is independently (CH<sub>2</sub>)<sub>n</sub>, CH<sub>2</sub>—CH(CH<sub>3</sub>)— or CH—(CH<sub>3</sub>)—CH<sub>2</sub>—; each Y may comprise —O—(O)C—, —C(O)—O—, —NR—C(O)—, or —C(O)—NR—; each m is 2 or 3; each n is from 1 to about 4, in one aspect 2; the sum of carbons in each R<sup>1</sup>, plus one when Y is 25 —O—(O)C— or —NR—C(O)—, may be C<sub>12</sub>-C<sub>22</sub>, or C<sub>14</sub>-C<sub>20</sub>, with each R<sup>1</sup> being a hydrocarbyl, or substituted hydrocarbyl group; and X<sup>-</sup> may comprise any softener-compatible anion. In one aspect, the softener-compatible anion may comprise chloride, bromide, methylsulfate, ethylsulfate, sulfate, and nitrate. In another aspect, the softener-compatible anion may comprise chloride or methyl sulfate.

In another aspect, the fabric softening active may comprise the general formula:



wherein each Y, R, R<sup>1</sup>, and X<sup>-</sup> have the same meanings as before. Such compounds include those having the formula:



wherein each R may comprise a methyl or ethyl group. In one aspect, each R<sup>1</sup> may comprise a C<sub>15</sub> to C<sub>19</sub> group. As used herein, when the diester is specified, it can include the monoester that is present.

These types of agents and general methods of making them are disclosed in U.S. Pat. No. 4,137,180. An example of a suitable DEQA (2) is the “propyl” ester quaternary ammonium fabric softener active comprising the formula 1,2-di(acyloxy)-3-trimethylammoniopropane chloride.

A third type of useful fabric softening active has the formula:



wherein each R, R<sup>1</sup>, m and X<sup>-</sup> have the same meanings as before.

In a further aspect, the fabric softening active may comprise the formula:



wherein each R, R<sup>1</sup>, and A<sup>-</sup> have the definitions given above; R<sup>2</sup> may comprise a C<sub>1-6</sub> alkylene group, in one aspect an ethylene group; and G may comprise an oxygen atom or an —NR— group;

In a yet further aspect, the fabric softening active may comprise the formula:



(5)

wherein R<sup>1</sup>, R<sup>2</sup> and G are defined as above.

In a further aspect, the fabric softening active may comprise condensation reaction products of fatty acids with dialkylenetriamines in, e.g., a molecular ratio of about 2:1, said reaction products containing compounds of the formula:



wherein R<sup>1</sup>, R<sup>2</sup> are defined as above, and R<sup>3</sup> may comprise a C<sub>1-6</sub> alkylene group, in one aspect, an ethylene group and wherein the reaction products may optionally be quaternized by the addition of an alkylating agent such as dimethyl sulfate. Such quaternized reaction products are described in additional detail in U.S. Pat. No. 5,296,622.

In a yet further aspect, the fabric softening active may comprise the formula:



wherein R, R<sup>1</sup>, R<sup>2</sup>, R<sup>3</sup> and A<sup>-</sup> are defined as above;

In a yet further aspect, the fabric softening active may comprise reaction products of fatty acid with hydroxyalkylalkylenediamines in a molecular ratio of about 2:1, said reaction products containing compounds of the formula:



wherein R<sup>1</sup>, R<sup>2</sup> and R<sup>3</sup> are defined as above;

In a yet further aspect, the fabric softening active may comprise the formula:



(9)

wherein R, R<sup>1</sup>, R<sup>2</sup>, and A<sup>-</sup> are defined as above.

In yet a further aspect, the fabric softening active may comprise the formula:



(10)

wherein:

X<sub>1</sub> is a C<sub>2-3</sub> alkyl group, in one aspect, an ethyl group; X<sub>2</sub> and X<sub>3</sub> are independently C<sub>1-6</sub> linear or branched alkyl or alkenyl groups, in one aspect, methyl, ethyl or isopropyl groups;

R<sub>1</sub> and R<sub>2</sub> are independently C<sub>8-22</sub> linear or branched alkyl or alkenyl groups; characterized in that;

A and B are independently selected from the group comprising —O—(C=O)—, —(C=O)—O—, or mixtures thereof, in one aspect, —O—(C=O)—

Non-limiting examples of fabric softening actives comprising formula (1) are N,N-bis(stearoyl-oxy-ethyl)-N,N-dimethylammonium chloride, N,N-bis(tallowoyl-oxy-ethyl)-N,N-dimethylammonium chloride, N,N-bis(stearoyl-oxy-ethyl)-N-(2-hydroxyethyl)-N-methylammonium methylsulfate.

Non-limiting examples of fabric softening actives comprising formula (2) is 1,2-di-(stearoyl-oxy)-3-trimethyl ammoniumpropane chloride.

Non-limiting examples of fabric softening actives comprising formula (3) include dialkylenedimethylammonium salts such as dicanoladimethylammonium chloride, di(hard) tallowdimethylammonium chloride, dicanoladimethylammonium methylsulfate, and mixtures thereof. An example of commercially available dialkylenedimethylammonium salts usable in the present invention is dioleyldimethylammonium chloride available from Witco Corporation under the trade name Adogen® 472 and dihardtallow dimethylammonium chloride available from Akzo Nobel Arquad 2HT75.

A non-limiting example of fabric softening actives comprising formula (4) is 1-methyl-1-stearoylamidoethyl-2-stearoylimidazolinium methylsulfate wherein R<sup>1</sup> is an acyclic aliphatic C<sub>15</sub>-C<sub>17</sub> hydrocarbon group, R<sup>2</sup> is an ethylene group, G is a NH group, R<sup>5</sup> is a methyl group and A<sup>-</sup> is a methyl sulfate anion, available commercially from the Witco Corporation under the trade name Varisoft®.

A non-limiting example of fabric softening actives comprising formula (5) is 1-tallowylamidoethyl-2-tallowylimidazoline wherein R<sup>1</sup> is an acyclic aliphatic C<sub>15</sub>-C<sub>17</sub> hydrocarbon group, R<sup>2</sup> is an ethylene group, and G is a NH group.

A non-limiting example of a fabric softening active comprising formula (6) is the reaction products of fatty acids with diethylenetriamine in a molecular ratio of about 2:1, said reaction product mixture containing N,N"-dialkyldiethylenetriamine with the formula:



wherein R<sup>1</sup> is an alkyl group of a commercially available fatty acid derived from a vegetable or animal source, such as Emersol® 223LL or Emersol® 7021, available from Henkel Corporation, and R<sup>2</sup> and R<sup>3</sup> are divalent ethylene groups.

In one aspect, said fatty acid may be obtained, in whole or in part, from a renewable source, via extraction from plant material, fermentation from plant material, and/or obtained via genetically modified organisms such as algae or yeast.

A non-limiting example of Compound (7) is a di-fatty amidoamine based softener having the formula:



wherein R<sup>1</sup> is an alkyl group. An example of such compound is that commercially available from the Witco Corporation e.g. under the trade name Varisoft® 222LT.

An example of a fabric softening active comprising formula (8) is the reaction products of fatty acids with

N-2-hydroxyethylenediamine in a molecular ratio of about 2:1, said reaction product mixture containing a compound of the formula:



wherein  $R^1-C(O)$  is an alkyl group of a commercially available fatty acid derived from a vegetable or animal source, such as Emersol® 223LL or Emersol® 7021, available from Henkel Corporation.

An example of a fabric softening active comprising formula (9) is the diquaternary compound having the formula:



wherein  $R^1$  is derived from fatty acid. Such compound is available from Witco Company.

A non-limiting example of a fabric softening active comprising formula (10) is a dialkyl imidazoline diester compound, where the compound is the reaction product of N-(2-hydroxyethyl)-1,2-ethylenediamine or N-(2-hydroxyisopropyl)-1,2-ethylenediamine with glycolic acid, esterified with fatty acid, where the fatty acid is (hydrogenated) tallow fatty acid, palm fatty acid, hydrogenated palm fatty acid, oleic acid, rapeseed fatty acid, hydrogenated rapeseed fatty acid or a mixture of the above.

It will be understood that combinations of softener actives disclosed above are suitable for use in this invention.

#### Anion A

In the cationic nitrogenous salts herein, the anion  $A^-$ , which comprises any softener compatible anion, provides electrical neutrality. Most often, the anion used to provide electrical neutrality in these salts is from a strong acid, especially a halide, such as chloride, bromide, or iodide. However, other anions can be used, such as methylsulfate, ethylsulfate, acetate, formate, sulfate, carbonate, fatty acid anions and the like. In one aspect, the anion A may comprise chloride or methylsulfate. The anion, in some aspects, may carry a double charge. In this aspect,  $A^-$  represents half a group.

In one embodiment, the fabric softening agent is chosen from at least one of the following: ditallowoyloxyethyl dimethyl ammonium chloride, dihydrogenated-tallowoyloxyethyl dimethyl ammonium chloride, ditallow dimethyl ammonium chloride, dihydrogenatedtallow dimethyl ammonium chloride, ditallowoyloxyethyl methylhydroxyethylammonium methyl sulfate, dihydrogenated-tallowoyloxyethyl methyl hydroxyethylammonium chloride, or combinations thereof.

#### Polyssacharides

One aspect of the invention provides a fabric enhancer composition comprising a cationic starch as a fabric softening active. In one embodiment, the fabric care compositions of the present invention generally comprise cationic starch at a level of from about 0.1% to about 7%, alternatively from about 0.1% to about 5%, alternatively from about 0.3% to about 3%, and alternatively from about 0.5% to about 2.0%, by weight of the composition. Suitable cationic starches for use in the present compositions are commercially-available from Cerestar under the trade name

C\*BOND® and from National Starch and Chemical Company under the trade name CATO® 2A.

#### Sucrose Esters

Nonionic fabric care benefit agents can comprise sucrose esters, and are typically derived from sucrose and fatty acids. Sucrose ester is composed of a sucrose moiety having one or more of its hydroxyl groups esterified.

Sucrose is a disaccharide having the following formula:



Alternatively, the sucrose molecule can be represented by the formula:  $M(OH)_8$ , wherein M is the disaccharide backbone and there are total of 8 hydroxyl groups in the molecule.

Thus, sucrose esters can be represented by the following formula:



wherein x is the number of hydroxyl groups that are esterified, whereas  $(8-x)$  is the hydroxyl groups that remain unchanged; x is an integer selected from 1 to 8, alternatively from 2 to 8, alternatively from 3 to 8, or from 4 to 8; and  $R^1$  moieties are independently selected from  $C_1-C_{22}$  alkyl or  $C_1-C_{30}$  alkoxy, linear or branched, cyclic or acyclic, saturated or unsaturated, substituted or unsubstituted.

In one embodiment, the  $R^1$  moieties comprise linear alkyl or alkoxy moieties having independently selected and varying chain length. For example,  $R^1$  may comprise a mixture of linear alkyl or alkoxy moieties wherein greater than about 20% of the linear chains are  $C_{18}$ , alternatively greater than about 50% of the linear chains are  $C_{18}$ , alternatively greater than about 80% of the linear chains are  $C_{18}$ .

In another embodiment, the  $R^1$  moieties comprise a mixture of saturate and unsaturated alkyl or alkoxy moieties; the degree of unsaturation can be measured by "Iodine Value" (hereinafter referred as "IV", as measured by the standard AOCS method). The IV of the sucrose esters suitable for use herein ranges from about 1 to about 150, or from about 2 to about 100, or from about 5 to about 85. The  $R^1$  moieties may be hydrogenated to reduce the degree of unsaturation. In the case where a higher IV is preferred, such as from about 40 to about 95, then oleic acid and fatty acids derived from soybean oil and canola oil are the starting materials.

In a further embodiment, the unsaturated  $R^1$  moieties may comprise a mixture of "cis" and "trans" forms about the unsaturated sites. The "cis"/"trans" ratios may range from about 1:1 to about 50:1, or from about 2:1 to about 40:1, or from about 3:1 to about 30:1, or from about 4:1 to about 20:1.

#### Dispersible Polyolefins

Generally, all dispersible polyolefins that provide fabric care benefits can be used as water insoluble fabric care benefit agents in the present invention. The polyolefins can be in the format of waxes, emulsions, dispersions or suspensions. Non-limiting examples are discussed below.

In one embodiment, the polyolefin is chosen from a polyethylene, polypropylene, or a combination thereof. The polyolefin may be at least partially modified to contain

various functional groups, such as carboxyl, alkylamide, sulfonic acid or amide groups. In another embodiment, the polyolefin is at least partially carboxyl modified or, in other words, oxidized.

For ease of formulation, the dispersible polyolefin may be introduced as a suspension or an emulsion of polyolefin dispersed by use of an emulsifying agent. The polyolefin suspension or emulsion may comprise from about 1% to about 60%, alternatively from about 10% to about 55%, alternatively from about 20% to about 50% by weight of polyolefin. The polyolefin may have a wax dropping point (see ASTM D3954-94, volume 15.04—"Standard Test Method for Dropping Point of Waxes") from about 20° to about 170° C., alternatively from about 50° to about 140° C. Suitable polyethylene waxes are available commercially from suppliers including but not limited to Honeywell (A-C polyethylene), Clariant (Velustrol® emulsion), and BASF (LUWAX®).

When an emulsion is employed with the dispersible polyolefin, the emulsifier may be any suitable emulsification agent. Non-limiting examples include an anionic, cationic, nonionic surfactant, or a combination thereof. However, almost any suitable surfactant or suspending agent may be employed as the emulsification agent. The dispersible polyolefin is dispersed by use of an emulsification agent in a ratio to polyolefin wax of about 1:100 to about 1:2, alternatively from about 1:50 to about 1:5, respectively.

#### Polymer Latexes

Polymer latex is made by an emulsion polymerization which includes one or more monomers, one or more emulsifiers, an initiator, and other components familiar to those of ordinary skill in the art. Generally, all polymer latexes that provide fabric care benefits can be used as water insoluble fabric care benefit agents of the present invention. Additional non-limiting examples include the monomers used in producing polymer latexes such as: (1) 100% or pure butylacrylate; (2) butylacrylate and butadiene mixtures with at least 20% (weight monomer ratio) of butylacrylate; (3) butylacrylate and less than 20% (weight monomer ratio) of other monomers excluding butadiene; (4) alkylacrylate with an alkyl carbon chain at or greater than C<sub>6</sub>; (5) alkylacrylate with an alkyl carbon chain at or greater than C<sub>6</sub> and less than 50% (weight monomer ratio) of other monomers; (6) a third monomer (less than 20% weight monomer ratio) added into an aforementioned monomer systems; and (7) combinations thereof.

Polymer latexes that are suitable fabric care benefit agents in the present invention may include those having a glass transition temperature of from about -120° C. to about 120° C., alternatively from about -80° C. to about 60° C. Suitable emulsifiers include anionic, cationic, nonionic and amphoteric surfactants. Suitable initiators include initiators that are suitable for emulsion polymerization of polymer latexes. The particle size diameter ( $\chi_{50}$ ) of the polymer latexes can be from about 1 nm to about 10  $\mu$ m, alternatively from about 10 nm to about 1  $\mu$ m, or even from about 10 nm to about 20 nm.

#### Fatty Acid

One aspect of the invention provides a fabric softening composition comprising a fatty acid, such as a free fatty acid. The term "fatty acid" is used herein in the broadest sense to include unprotonated or protonated forms of a fatty acid; and includes fatty acid that is bound or unbound to another chemical moiety as well as the various combinations of these species of fatty acid. One skilled in the art will readily appreciate that the pH of an aqueous composition will dictate, in part, whether a fatty acid is protonated or

unprotonated. In another embodiment, the fatty acid is in its unprotonated, or salt form, together with a counter ion, such as, but not limited to, calcium, magnesium, sodium, potassium and the like. The term "free fatty acid" means a fatty acid that is not bound to another chemical moiety (covalently or otherwise) to another chemical moiety.

In one embodiment, the fatty acid may include those containing from about 12 to about 25, from about 13 to about 22, or even from about 16 to about 20, total carbon atoms, with the fatty moiety containing from about 10 to about 22, from about 12 to about 18, or even from about 14 (mid-cut) to about 18 carbon atoms.

The fatty acids of the present invention may be derived from (1) an animal fat, and/or a partially hydrogenated animal fat, such as beef tallow, lard, etc.; (2) a vegetable oil, and/or a partially hydrogenated vegetable oil such as canola oil, safflower oil, peanut oil, sunflower oil, sesame seed oil, rapeseed oil, cottonseed oil, corn oil, soybean oil, tall oil, rice bran oil, palm oil, palm kernel oil, coconut oil, other 15 tropical palm oils, linseed oil, tung oil, etc.; (3) processed and/or bodied oils, such as linseed oil or tung oil via thermal, pressure, alkali-isomerization and catalytic treatments; (4) a mixture thereof, to yield saturated (e.g. stearic acid), unsaturated (e.g. oleic acid), polyunsaturated (linoleic acid), branched (e.g. isostearic acid) or cyclic (e.g. saturated or unsaturated  $\alpha$ -disubstituted cyclopentyl or cyclohexyl derivatives of polyunsaturated acids) fatty acids.

Mixtures of fatty acids from different fat sources can be used.

In one aspect, at least a majority of the fatty acid that is present in the fabric softening composition of the present invention is unsaturated, e.g., from about 40% to 100%, from about 55% to about 99%, or even from about 60% to about 98%, by weight of the total weight of the fatty acid present in the composition, although fully saturated and partially saturated fatty acids can be used. As such, the total level of polyunsaturated fatty acids (TPU) of the total fatty acid of the inventive composition may be from about 0% to about 75% by weight of the total weight of the fatty acid present in the composition.

The cis/trans ratio for the unsaturated fatty acids may be important, with the cis/trans ratio (of the C18:1 material) being from at least about 1:1, at least about 3:1, from about 4:1 or even from about 9:1 or higher.

Branched fatty acids such as isostearic acid are also suitable since they may be more stable with respect to oxidation and the resulting degradation of color and odor quality.

The Iodine Value or "IV" measures the degree of unsaturation in the fatty acid. In one embodiment of the invention, the fatty acid has an IV from about 10 to about 140, from about 15 to about 100 or even from about 15 to about 60.

Another class of fatty ester fabric care actives is softening oils, which include but are not limited to, vegetable oils (such as soybean, sunflower, and canola), hydrocarbon based oils (natural and synthetic petroleum lubricants, in one aspect polyolefins, isoparaffins, and cyclic paraffins), triolein, fatty esters, fatty alcohols, fatty amines, fatty amides, and fatty ester amines. Oils can be combined with fatty acid softening agents, clays, and silicones.

#### Clays

In one embodiment of the invention, the fabric care composition may comprise a clay as a fabric care active. In one embodiment clay can be a softener or co-softeners with another softening active, for example, silicone. Suitable clays include those materials classified geologically smectites.

## Silicone

In one embodiment, the fabric softening composition comprises a silicone. Suitable levels of silicone may comprise from about 0.1% to about 70%, alternatively from about 0.3% to about 40%, alternatively from about 0.5% to about 30%, alternatively from about 1% to about 20% by weight of the composition. Useful silicones can be any silicone comprising compound. In one embodiment, the silicone polymer is selected from the group consisting of cyclic silicones, polydimethylsiloxanes, aminosilicones, cationic silicones, silicone polyethers, silicone resins, silicone urethanes, and mixtures thereof. In one embodiment, the silicone is a polydialkylsilicone, alternatively a polydimethyl silicone (polydimethyl siloxane or "PDMS"), or a derivative thereof. In another embodiment, the silicone is chosen from an aminofunctional silicone, amino-polyether silicone, alkyloxylated silicone, cationic silicone, ethoxyLATED silicone, propoxylated silicone, ethoxylated/propoxylated silicone, quaternary silicone, or combinations thereof.

In another embodiment, the silicone may be chosen from a random or blocky organosilicone polymer having the following formula:



wherein:

j is an integer from 0 to about 98; in one aspect j is an integer from 0 to about 48; in one aspect, j is 0;

k is an integer from 0 to about 200, in one aspect k is an integer from 0 to about 50; when k=0, at least one of

R<sub>1</sub>, R<sub>2</sub> or R<sub>3</sub> is —X—Z;

m is an integer from 4 to about 5,000; in one aspect m is an integer from about 10 to about 4,000; in another aspect m is an integer from about 50 to about 2,000;

R<sub>1</sub>, R<sub>2</sub> and R<sub>3</sub> are each independently selected from the group consisting of H, OH, C<sub>1</sub>-C<sub>32</sub> alkyl, C<sub>1</sub>-C<sub>32</sub> substituted alkyl, C<sub>5</sub>-C<sub>32</sub> or C<sub>6</sub>-C<sub>32</sub> aryl, C<sub>5</sub>-C<sub>32</sub> or C<sub>6</sub>-C<sub>32</sub> substituted aryl, C<sub>6</sub>-C<sub>32</sub> alkylaryl, C<sub>6</sub>-C<sub>32</sub> substituted alkylaryl, C<sub>1</sub>-C<sub>32</sub> alkoxy, C<sub>1</sub>-C<sub>32</sub> substituted alkoxy and X—Z;

each R<sup>4</sup> is independently selected from the group consisting of H, OH, C<sub>1</sub>-C<sub>32</sub> alkyl, C<sub>1</sub>-C<sub>32</sub> substituted alkyl, C<sub>5</sub>-C<sub>32</sub> or C<sub>6</sub>-C<sub>32</sub> aryl, C<sub>5</sub>-C<sub>32</sub> or C<sub>6</sub>-C<sub>32</sub> substituted aryl, C<sub>6</sub>-C<sub>32</sub> alkylaryl, C<sub>6</sub>-C<sub>32</sub> substituted alkylaryl, C<sub>1</sub>-C<sub>32</sub> alkoxy and C<sub>1</sub>-C<sub>32</sub> substituted alkoxy;

each X in said alkyl siloxane polymer comprises a substituted or unsubstituted divalent alkylene radical comprising 2-12 carbon atoms, in one aspect each divalent alkylene radical is independently selected from the group consisting of —(CH<sub>2</sub>)<sub>s</sub>— wherein s is an integer from about 2 to about 8, from about 2 to about 4; in one aspect, each X in said alkyl siloxane polymer comprises a substituted divalent alkylene radical selected from the group consisting of: —CH<sub>2</sub>—CH(OH)—CH<sub>2</sub>—; —CH<sub>2</sub>—CH<sub>2</sub>—CH(OH)—; and



each Z is selected independently from the group consisting of



with the proviso that when Z is a quat, Q cannot be an amide, imine, or urea moiety and if Q is an amide, imine, or urea moiety, then any additional Q bonded to the same nitrogen as said amide, imine, or urea moiety must be H or a C<sub>1</sub>-C<sub>6</sub> alkyl, in one aspect, said additional Q is H; for Z A<sup>n-</sup> is a suitable charge balancing anion. In one aspect A<sup>n-</sup> is selected from the group consisting of Cl<sup>-</sup>, Br<sup>-</sup>, I<sup>-</sup>, methylsulfate, toluene sulfonate, carboxylate and phosphate; and at least one Q in said organosilicone is independently selected from



## 25

-continued



each additional Q in said organosilicone is independently selected from the group comprising of H,  $C_1$ - $C_{32}$  alkyl,  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl,  $C_6$ - $C_{32}$  substituted alkylaryl, 10



wherein each  $R_5$  is independently selected from the group 35 consisting of H,  $C_1$ - $C_{32}$  alkyl,  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl,  $C_6$ - $C_{32}$  substituted alkylaryl,  $-(\text{CH}_2\text{---CH}_2\text{---O---})_w\text{---L}$  and a siloxyl residue; 40

each  $R_6$  is independently selected from H,  $C_1$ - $C_{18}$  alkyl each L is independently selected from  $-\text{C}(\text{O})\text{---R}^7$  or  $R^7$ ;

w is an integer from 0 to about 500, in one aspect w is an integer from about 1 to about 200; in one aspect w is an integer from about 1 to about 50; each  $R_7$  is selected 45 independently from the group consisting of H;  $C_1$ - $C_{32}$  alkyl;  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl;  $C_6$ - $C_{32}$  substituted alkylaryl and a siloxyl residue; 50

each T is independently selected from H,



and wherein each v in said organosilicone is an integer from 60 1 to about 10, in one aspect, v is an integer from 1 to about 5 and the sum of all v indices in each Q in the said organosilicone is an integer from 1 to about 30 or from 1 to about 20 or even from 1 to about 10.

In another embodiment, the silicone may be chosen from 65 a random or blocky organosilicone polymer having the following formula:

## 26



wherein

j is an integer from 0 to about 98; in one aspect j is an integer from 0 to about 48; in one aspect, j is 0;

k is an integer from 0 to about 200; when k=0, at least one of  $R_1$ ,  $R_2$  or  $R_3$ = $X\text{---Z}$ , in one aspect, k is an integer from 0 to about 50

m is an integer from 4 to about 5,000; in one aspect m

is an integer from about 10 to about 4,000; in another aspect m is an integer from about 50 to about 2,000;

$R_1$ ,  $R_2$  and  $R_3$  are each independently selected from the group consisting of H, OH,  $C_1$ - $C_{32}$  alkyl,  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl,  $C_6$ - $C_{32}$  substituted alkylaryl,  $C_1$ - $C_{32}$  alkoxy,  $C_1$ - $C_{32}$  substituted alkoxy and  $X\text{---Z}$ ;

each  $R^4$  is independently selected from the group consisting of H, OH,  $C_1$ - $C_{32}$  alkyl,  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl,  $C_6$ - $C_{32}$  substituted alkylaryl,  $C_1$ - $C_{32}$  alkoxy and  $C_1$ - $C_{32}$  substituted alkoxy;

each X comprises of a substituted or unsubstituted divalent alkylene radical comprising 2-12 carbon atoms; in one aspect each X is independently selected from the group consisting of  $-(\text{CH}_2)_s\text{---O---}$ ;  $-\text{CH}_2\text{---CH(OH)}\text{---CH}_2\text{---O---}$ ;



wherein each s independently is an integer from about 2 to about 8, in one aspect s is an integer from about 2 to about 4;

At least one Z in the said organosiloxane is selected from the group consisting of  $R_5$ ;



27



provided that when X is

then  $Z=\text{---OR}_5$  or

wherein  $\text{A}^-$  is a suitable charge balancing anion. In one aspect  $\text{A}^-$  is selected from the group consisting of  $\text{Cl}^-$ ,  $\text{Br}^-$ , <sup>40</sup>

$\text{I}^-$ , methylsulfate, toluene sulfonate, carboxylate and phosphate and

each additional Z in said organosilicone is independently <sup>45</sup> selected from the group comprising of H,  $\text{C}_1\text{-C}_{32}$  alkyl,  $\text{C}_1\text{-C}_{32}$  substituted alkyl,  $\text{C}_5\text{-C}_{32}$  or  $\text{C}_6\text{-C}_{32}$  aryl,  $\text{C}_5\text{-C}_{32}$  or  $\text{C}_6\text{-C}_{32}$  substituted aryl,  $\text{C}_6\text{-C}_{32}$  alkylaryl,  $\text{C}_6\text{-C}_{32}$  substituted alkylaryl,  $\text{R}_5$ ,

 $\text{A}^-$ 

28



provided that when X is

then  $Z=\text{---OR}_5$  or

each  $\text{R}_5$  is independently selected from the group consisting of H;  $\text{C}_1\text{-C}_{32}$  alkyl;  $\text{C}_1\text{-C}_{32}$  substituted alkyl,  $\text{C}_5\text{-C}_{32}$  or  $\text{C}_6\text{-C}_{32}$  aryl,  $\text{C}_5\text{-C}_{32}$  or  $\text{C}_6\text{-C}_{32}$  substituted aryl or  $\text{C}_6\text{-C}_{32}$  alkylaryl, or  $\text{C}_6\text{-C}_{32}$  substituted alkylaryl,  $-(\text{CH}_6\text{---CH}_6\text{---O})_w\text{---CH}_6\text{---CH}_6\text{---L}$  and siloxyl residue wherein each L is independently selected from  $\text{---O---C}(\text{O})\text{---R}^7$  or  $\text{---O---R}^7$ ;



w is an integer from 0 to about 500, in one aspect w is an integer from 0 to about 200, one aspect w is an integer from 0 to about 50;

each  $\text{R}_6$  is independently selected from H or  $\text{C}_1\text{-C}_{18}$  alkyl; each  $\text{R}_7$  is independently selected from the group consisting of H;  $\text{C}_1\text{-C}_{32}$  alkyl;  $\text{C}_1\text{-C}_{32}$  substituted alkyl,  $\text{C}_5\text{-C}_{32}$  or  $\text{C}_6\text{-C}_{32}$  aryl,  $\text{C}_5\text{-C}_{32}$  or  $\text{C}_6\text{-C}_{32}$  substituted aryl,  $\text{C}_6\text{-C}_{32}$  alkylaryl, and  $\text{C}_6\text{-C}_{32}$  substituted aryl, and a siloxyl residue;

each T is independently selected from H;



wherein each v in said organosilicone is an integer from 1 to about 10, in one aspect, v is an integer from 1 to

about 5 and the sum of all v indices in each Z in the said organosilicone is an integer from 1 to about 30 or from 1 to about 20 or even from 1 to about 10.

In one embodiment, the silicone is one comprising a relatively high molecular weight. A suitable way to describe the molecular weight of a silicone includes describing its viscosity. A high molecular weight silicone is one having a viscosity of from about 10 cSt to about 3,000,000 cSt, or from about 100 cSt to about 1,000,000 cSt, or from about 1,000 cSt to about 600,000 cSt, or even from about 6,000 cSt to about 300,000 cSt.

In one embodiment, the silicone comprises a blocky cationic organopolysiloxane having the formula:



wherein:

M=[SiR<sub>1</sub>R<sub>2</sub>R<sub>3</sub>O<sub>1/2</sub>], [SiR<sub>1</sub>R<sub>2</sub>G<sub>1</sub>O<sub>1/2</sub>], [SiR<sub>1</sub>G<sub>1</sub>G<sub>2</sub>O<sub>1/2</sub>], [SiG<sub>1</sub>G<sub>2</sub>G<sub>3</sub>O<sub>1/2</sub>], or combinations thereof;

D=[SiR<sub>1</sub>R<sub>2</sub>O<sub>2/2</sub>], [SiR<sub>1</sub>G<sub>1</sub>O<sub>2/2</sub>], [SiG<sub>1</sub>G<sub>2</sub>O<sub>2/2</sub>] or combinations thereof;

T=[SiR<sub>1</sub>O<sub>3/2</sub>], [SiG<sub>1</sub>O<sub>3/2</sub>] or combinations thereof;

Q=[SiO<sub>4/2</sub>];

w=is an integer from 1 to (2+y+2z);

x=is an integer from 5 to 15,000;

y=is an integer from 0 to 98;

z=is an integer from 0 to 98;

R<sub>1</sub>, R<sub>2</sub> and R<sub>3</sub> are each independently selected from the group consisting of H, OH, C<sub>1</sub>-C<sub>32</sub> alkyl, C<sub>1</sub>-C<sub>32</sub> substituted alkyl, C<sub>5</sub>-C<sub>32</sub> or C<sub>6</sub>-C<sub>32</sub> aryl, C<sub>5</sub>-C<sub>32</sub> or C<sub>6</sub>-C<sub>32</sub> substituted aryl, C<sub>6</sub>-C<sub>32</sub> alkylaryl, C<sub>6</sub>-C<sub>32</sub> substituted alkylaryl, C<sub>1</sub>-C<sub>32</sub> alkoxy, C<sub>1</sub>-C<sub>32</sub> substituted alkoxy, C<sub>1</sub>-C<sub>32</sub> alkylamino, and C<sub>1</sub>-C<sub>32</sub> substituted alkylamino;

at least one of M, D, or T incorporates at least one moiety G<sub>1</sub>, G<sub>2</sub> or G<sub>3</sub>; and G<sub>1</sub>, G<sub>2</sub>, and G<sub>3</sub> are each independently selected from the formula:



wherein:

X comprises a divalent radical selected from the group consisting of C<sub>1</sub>-C<sub>32</sub> alkylene, C<sub>1</sub>-C<sub>32</sub> substituted alkylene, C<sub>5</sub>-C<sub>32</sub> or C<sub>6</sub>-C<sub>32</sub> arylene, C<sub>5</sub>-C<sub>32</sub> or C<sub>6</sub>-C<sub>32</sub> substituted arylene, C<sub>6</sub>-C<sub>32</sub> arylalkylene, C<sub>6</sub>-C<sub>32</sub> substituted arylalkylene, C<sub>1</sub>-C<sub>32</sub> alkoxy, C<sub>1</sub>-C<sub>32</sub> substituted alkoxy, C<sub>1</sub>-C<sub>32</sub> alkyleneamino, C<sub>1</sub>-C<sub>32</sub> substituted alkyleneamino, ring-opened epoxide, and ring-opened glycidyl, with the proviso that if X does not comprise a repeating alkylene oxide moiety then X can further comprise a heteroatom selected from the group consisting of P, N and O;

each R<sub>4</sub> comprises identical or different monovalent radicals selected from the group consisting of H, C<sub>1</sub>-C<sub>32</sub> alkyl, C<sub>1</sub>-C<sub>32</sub> substituted alkyl, C<sub>5</sub>-C<sub>32</sub> or C<sub>6</sub>-C<sub>32</sub> aryl, C<sub>5</sub>-C<sub>32</sub> or C<sub>6</sub>-C<sub>32</sub> substituted aryl, C<sub>6</sub>-C<sub>32</sub> alkylaryl, and C<sub>6</sub>-C<sub>32</sub> substituted alkylaryl;

E comprises a divalent radical selected from the group consisting of C<sub>1</sub>-C<sub>32</sub> alkylene, C<sub>1</sub>-C<sub>32</sub> substituted alkylene, C<sub>5</sub>-C<sub>32</sub> or C<sub>6</sub>-C<sub>32</sub> arylene, C<sub>5</sub>-C<sub>32</sub> or C<sub>6</sub>-C<sub>32</sub> substituted arylene, C<sub>6</sub>-C<sub>32</sub> arylalkylene, C<sub>6</sub>-C<sub>32</sub> substituted arylalkylene, C<sub>1</sub>-C<sub>32</sub> alkoxy, C<sub>1</sub>-C<sub>32</sub> substituted alkoxy, C<sub>1</sub>-C<sub>32</sub> alkyleneamino, C<sub>1</sub>-C<sub>32</sub> substituted alkyleneamino, ring-opened epoxide and ring-opened glycidyl, with the proviso that if E does not comprise a repeating alkylene oxide moiety then E can further comprise a heteroatom selected from the group consisting of P, N, and O;

E' comprises a divalent radical selected from the group consisting of C<sub>1</sub>-C<sub>32</sub> alkylene, C<sub>1</sub>-C<sub>32</sub> substituted alkylene, C<sub>5</sub>-C<sub>32</sub> or C<sub>6</sub>-C<sub>32</sub> arylene, C<sub>5</sub>-C<sub>32</sub> or C<sub>6</sub>-C<sub>32</sub> substituted arylene, C<sub>6</sub>-C<sub>32</sub> arylalkylene, C<sub>6</sub>-C<sub>32</sub> substituted arylalkylene, C<sub>1</sub>-C<sub>32</sub> alkoxy, C<sub>1</sub>-C<sub>32</sub> substituted alkoxy, C<sub>1</sub>-C<sub>32</sub> alkyleneamino, C<sub>1</sub>-C<sub>32</sub> substituted alkyleneamino, ring-opened epoxide and ring-opened glycidyl, with the proviso that if E' does not comprise a repeating alkylene oxide moiety then E' can further comprise a heteroatom selected from the group consisting of P, N, and O;

p is an integer independently selected from 1 to 50;

n is an integer independently selected from 1 or 2;

when at least one of G<sub>1</sub>, G<sub>2</sub>, or G<sub>3</sub> is positively charged, A<sup>-t</sup> is a suitable charge balancing anion or anions such that the total charge, k, of the charge-balancing anion or anions is equal to and opposite from the net charge on the moiety G<sub>1</sub>, G<sub>2</sub> or G<sub>3</sub>; wherein t is an integer independently selected from 1, 2, or 3; and k≤(p\*2/t)+1; such that the total number of cationic charges balances the total number of anionic charges in the organopolysiloxane molecule; and wherein at least one E does not comprise an ethylene moiety.

#### Process of Making Polymers

Polymers useful in the present invention can be made by one skilled in the art. Examples of processes for making polymers include, but are not limited, solution polymerization, emulsion polymerization, inverse emulsion polymerization, inverse dispersion polymerization, and liquid dispersion polymer technology. In one aspect, a method of making a polymer having a chain transfer agent (CTA) value in a range greater than 10,000 ppm by weight of the polymer is disclosed. Another aspect of the invention is directed to providing a polymer having a cross linker level greater than 5 ppm, alternatively greater than 45 ppm, by weight of the polymer.

In one aspect of making a polymer, the CTA is present in a range greater than about 100 ppm based on the weight of the polymer. In one aspect, the CTA is from about 100 ppm to about 10,000 ppm, alternatively from about 500 ppm to about 4,000 ppm, alternatively from about 1,000 ppm to about 3,500 ppm, alternatively from about 1,500 ppm to about 3,000 ppm, alternatively from about 1,500 ppm to about 2,500 ppm, alternatively combinations thereof based on the weight of the polymer. In yet another aspect, the CTA is greater than about 1,000 based on the weight of the polymer. It is also suitable to use mixtures of chain transfer agents.

In one aspect of the invention, the polymer comprises 5-100% by weight (wt-%) of at least one cationic monomer and 5-95 wt-% of at least one non-ionic monomer. The weight percentages relate to the total weight of the copolymer. In another aspect of the invention, the polymer comprises 0-50% by weight (wt-%) of an anionic monomer.

#### Cationic Monomers for Polymers

Suitable cationic monomers include dialkyl ammonium halides or compounds according to formula (I):



wherein:

R<sub>1</sub> is chosen from hydrogen, or C<sub>1</sub>-C<sub>4</sub> alkyl, in one aspect, R<sub>1</sub> is hydrogen or methyl;

R<sub>2</sub> is chosen from hydrogen or methyl, in one aspect, R<sub>1</sub> is hydrogen

R<sub>3</sub> is chosen from C<sub>1</sub>-C<sub>4</sub> alkylene, in one aspect, R<sub>3</sub> is ethylene;

R<sub>4</sub>, R<sub>5</sub>, and R<sub>6</sub> are each independently chosen from hydrogen, C<sub>1</sub>-C<sub>4</sub> alkyl, C<sub>1</sub>-C<sub>4</sub> alkyl alcohol, or C<sub>1</sub>-C<sub>4</sub> alkoxy, in one aspect, R<sub>4</sub>, R<sub>5</sub>, and R<sub>6</sub> are methyl;

X is chosen from —O—, or —NH—, in one aspect, X is —O—; and

Y is chosen from Cl, Br, I, hydrogensulfate or methysulfate, in one aspect, Y is C<sub>1</sub>.

The alkyl and alkoxy groups may be linear or branched.

The alkyl groups are methyl, ethyl, propyl, butyl, and isopropyl.

In one aspect, the cationic monomer of formula (I) is dimethyl aminoethyl acrylate methyl chloride. In another aspect, the cationic monomer of formula (I) is dimethyl aminoethyl methacrylate methyl chloride.

In another aspect, the cationic monomer is dialkyldimethyl ammonium chloride.

#### Non-Ionic Monomers for Polymers

Suitable non-ionic monomers include compounds of formula (II) wherein



wherein:

R<sub>7</sub> is chosen from hydrogen or C<sub>1</sub>-C<sub>4</sub> alkyl; in one aspect R<sub>7</sub> is hydrogen;

R<sub>8</sub> is chosen from hydrogen or methyl; in one aspect, R<sub>8</sub> is hydrogen; and

R<sub>9</sub> and R<sub>10</sub> are each independently chosen from hydrogen or C<sub>1</sub>-C<sub>4</sub> alkyl, C<sub>1</sub>-C<sub>4</sub> alkyl alcohol or C<sub>1</sub>-C<sub>4</sub> alkoxy; in one aspect, R<sub>9</sub> and R<sub>10</sub> are each independently chosen from hydrogen or methyl.

In one aspect, the non-ionic monomer is acrylamide.

In another aspect, the non-ionic monomer is hydroxyethyl acrylate.

#### Anionic Monomers for Polymers

Suitable anionic monomer may include the group consisting of acrylic acid, methacrylic acid, itaconic acid, crotonic acid, maleic acid, fumaric acid, as well as monomers performing a sulfonic acid or phosphonic acid functions, such as 2-acrylamido-2-methyl propane sulfonic acid (ATBS), and their salts.

#### Cross-Linking Agent for Polymers

The cross-linking agent contains at least two ethylenically unsaturated moieties. In one aspect, the cross-linking agent contains at least two or more ethylenically unsaturated moieties; in one aspect, the cross-linking agent contains at least three or more ethylenically unsaturated moieties.

Suitable cross-linking agents include divinyl benzene, tetraallylammonium chloride; allyl acrylates; allyl acrylates and methacrylates, diacrylates and dimethacrylates of glycols and polyglycols, allyl methacrylates; and tri- and tetramethacrylates of polyglycols; or polyol polyallyl ethers such as polyallyl sucrose or pentaerythritol triallyl ether, butadiene, 1,7-octadiene, allyl-acrylamides and allyl-meth-

acrylamides, bisacrylamidoacetic acid, N,N'-methylene-bisacrylamide and polyol polyallyl ethers, such as polyallyl-saccharose and pentaerythritol triallyl ether, ditrimethylolpropane tetraacrylate, pentaerythrityl tetraacrylate, pentaerythrityl tetraacrylate ethoxylate, pentaerythrityl tetramethacrylate, pentaerythrityl triacrylate, pentaerythrityl triacrylate ethoxylate, triethanolamine trimethacrylate, 1,1,1-trimethylolpropane triacrylate, 1,1,1-trimethylolpropane triacrylate ethoxylate, trimethylolpropane tris(polyethylene glycol ether) triacrylate, 1,1,1-trimethylolpropane trimethacrylate, tris-(2-hydroxyethyl)-1,3,5-triazine-2,4,6-trione triacrylate, tris-(2-hydroxyethyl)-1,3,5-triazine-2,4,6-trione trimethacrylate, dipentaerythrityl pentaacrylate, 3-(3-[(dimethyl-(vinyl)-silyl)-oxy]-1,1,5,5-tetramethyl-1,5-divinyl-3-trisiloxanyl)-propyl methacrylate, dipentaerythritol hexaacrylate, 1-(2-propenylloxy)-2,2-bis[(2-propenylloxy)-methyl]-butane, trimethacrylic acid-1,3,5-triazin-2,4,6-triyl-tri-2,1-ethandyl ester, glycerine triacrylate propoxylate, 1,3,5-triacyloylhexahydro-1,3,5-triazine, 1,3-dimethyl-1,1,3,3-tetravinylldisiloxane, pentaerythrityl tetravinyl ether, 1,3-dimethyl-1,1,3,3-tetravinylldisiloxane, (Ethoxy)-trivinylsilane, (Methyl)-trivinylsilane, 1,1,3,5,5-pentamethyl-1,3,5-trivinyltrisiloxane, 1,3,5-trimethyl-1,3,5-trivinylcyclotrisiloxane, 2,4,6-trimethyl-2,4,6-trivinylcyclotrisiloxane, 1,3,5-trimethyl-1,3,5-trivinyltrisiloxane, tris-(2-butanone oxime)-vinylsilane, 1,2,4-trivinylcyclohexane, trivinylphosphine, trivinylsilane, methyltriallylsilane, pentaerythrityl triallyl ether, phenyltriallylsilane, triallylamine, triallyl citrate, triallyl phosphate, triallylphosphine, triallyl phosphite, triallylsilane, 1,3,5-triallyl-1,3,5-triazine-2,4,6 (1H,3H,5H)-trione, trimellitic acid triallyl ester, trimethallyl isocyanurate, 2,4,6-tris-(allyloxy)-1,3,5-triazine, 1,2-Bis-(diallylamino)-ethane, pentaerythrityl tetratallate, 1,3,5,7-tetravinyl-1,3,5,7-tetramethylcyclotetrasiloxane, 1,3,5,7-tetravinyl-1,3,5,7-tetramethylcyclotetrasiloxane, tris-[(2-acryloyloxy)-ethyl]-phosphate, vinylboronic anhydride pyridine, 2,4,6-trivinylcyclotriboroxanepyridine, tetraallylsilane, tetraallyloxydisilane, 1,3,5,7-tetramethyl-1,3,5,7-tetravinylcyclotetrasilazane. Preferred compounds include alkyltritylammmonium chloride, pentaerythrityl triacrylate, pentaerythrityl tetraacrylate, tetraallylammonium chloride, 1,1,1-trimethylolpropane tri(meth)acrylate, or a mixture thereof. These preferred compounds can also be ethoxylated and mixtures thereof. In one aspect, the cross-linking agents are chosen from tetraallyl ammonium chloride, allyl-acrylamides and allyl-methacrylamides, bisacrylamidoacetic acid, and N,N'-methylene-bisacrylamide, and mixtures thereof. In one aspect, the cross-linking agent is tetraallyl ammonium chloride. In another aspect, the cross-linking agent is a mixture of pentaerythrityl triacrylate and pentaerythrityl tetraacrylate.

For Polymer 1, the crosslinker(s) is (are) included in the range of from about 45 ppm to about 5,000 ppm, alternatively from about 50 ppm to about 500 ppm; alternatively from about 100 ppm to about 400 ppm, alternatively from about 500 ppm to about 4,500 ppm, alternatively from about 550 ppm to about 4,000 ppm based on the weight of the polymer.

For Polymer 2, the crosslinker(s) is (are) included in the range from 0 ppm to about 40 ppm, alternatively from about 0 ppm to about 20 ppm; alternatively from about 0 ppm to about 10 ppm based on the weight of the polymer.

#### Chain Transfer Agent (CTA) for Polymers

The chain transfer agent includes mercaptans, malic acid, lactic acid, formic acid, isopropanol and hypophosphites, and mixtures thereof. In one aspect, the CTA is formic acid.

The CTA is present in a range greater than about 100 ppm based on the weight of the polymer. In one aspect, the CTA is present from about 100 ppm to about 10,000 ppm, alternatively from about 500 ppm to about 4,000 ppm, alternatively from about 1,000 ppm to about 3,500 ppm, alternatively from about 1,500 ppm to about 3,000 ppm, alternatively from about 1,500 ppm to about 2,500 ppm, alternatively combinations thereof based on the weight of the polymer. In yet another aspect, the CTA level is greater than about 1,000 based on the weight of the polymer. It is also suitable to use mixtures of chain transfer agents.

#### Molecular Weight Range for Polymers

In one aspect, the polymer comprises a Number Average Molecular Weight (Mn) from about 10,000 Daltons to about 15,000,000 Daltons, alternatively from about 1,500,000 Daltons to about 2,500,000 Daltons.

In another aspect, the polymer comprises a Weight Average Molecular Weight (Mw) from about 4,000,000 Daltons to about 11,000,000 Daltons, alternatively from about 4,000,000 Daltons to about 6,000,000 Daltons.

#### Stabilizing Agents for Polymer Synthesis and Examples

Stabilizing agent A (nonionic block copolymer): Polyglyceryl-dipolyhydroxystearate with CAS-No. 144470-58-6

Stabilizing agent B is a nonionic ABA-block copolymer with molecular weight of about 5000 g/mol, and a hydrophobic lipophilic balance value (HLB) of 5 to 6, wherein the A block is based on polyhydroxystearic acid and the B block on polyalkylene oxide, having the formula below:



Stabilizing agent C (nonionic block copolymer): PEG-30 Dipolyhydroxystearate, with CAS-Nr. 70142-34-6

Stabilizing agent D (nonionic block copolymer): Alcyd Polyethyleneglycol Poly-isobutene stabilizing surfactant with HLB 5-7.

#### Adjunct Materials

While not essential for the purposes of the present invention, the non-limiting list of adjuncts illustrated hereinafter are suitable for use in the instant compositions and may be desirably incorporated in certain aspects of the invention, for example to assist or enhance cleaning performance, for treatment of the substrate to be cleaned, or to modify the aesthetics of the composition as is the case with perfumes, colorants, dyes or the like. The precise nature of these additional components, and levels of incorporation thereof, will depend on the physical form of the composition and the nature of the fabric treatment operation for which it is to be used. Suitable adjunct materials include, but are not limited to, surfactants, builders, chelating agents, dye transfer inhibiting agents, dispersants, enzymes, and enzyme stabilizers, catalytic materials, bleach activators, hydrogen peroxide, sources of hydrogen peroxide, preformed peracids, polymeric dispersing agents, clay soil removal/anti-redeposition agents, brighteners, suds suppressors, dyes, hueing dyes, perfumes, perfume delivery systems, structure elasticizing agents, carriers, structurants, hydrotropes, processing aids, solvents and/or pigments.

As stated, the adjunct ingredients are not essential to Applicants' compositions. Thus, certain aspects of Applicants' compositions do not contain one or more of the following adjuncts materials: surfactants, builders, chelating agents, dye transfer inhibiting agents, dispersants, enzymes, and enzyme stabilizers, catalytic materials, bleach activa-

tors, hydrogen peroxide, sources of hydrogen peroxide, preformed peracids, polymeric dispersing agents, clay soil removal/anti-redeposition agents, brighteners, suds suppressors, dyes, hueing dyes, perfumes, perfume delivery systems, structure elasticizing agents, carriers, hydrotropes, process-

ing aids, solvents and/or pigments. However, when one or more adjuncts are present, such one or more adjuncts may be present as detailed below.

**Hueing Dye—**

The liquid laundry detergent composition may comprise a hueing dye. The hueing dyes employed in the present laundry care compositions may comprise polymeric or non-polymeric dyes, organic or inorganic pigments, or mixtures thereof. Preferably the hueing dye comprises a polymeric dye, comprising a chromophore constituent and a polymeric constituent. The chromophore constituent is characterized in that it absorbs light in the wavelength range of blue, red, violet, purple, or combinations thereof upon exposure to light. In one aspect, the chromophore constituent exhibits an absorbance spectrum maximum from about 520 nanometers to about 640 nanometers in water and/or methanol, and in another aspect, from about 560 nanometers to about 610 nanometers in water and/or methanol.

Although any suitable chromophore may be used, the dye chromophore is preferably selected from benzodifuranes, methine, triphenylmethanes, naphthalimides, pyrazole, napthoquinone, anthraquinone, azo, oxazine, azine, xanthene, triphenodioxazine and phthalocyanine dye chromophores. Mono and di-azo dye chromophores are may be preferred.

The hueing dye may comprise a dye polymer comprising a chromophore covalently bound to one or more of at least three consecutive repeat units. It should be understood that the repeat units themselves do not need to comprise a chromophore. The dye polymer may comprise at least 5, or at least 10, or even at least 20 consecutive repeat units.

The repeat unit can be derived from an organic ester such as phenyl dicarboxylate in combination with an oxyalkyleneoxy and a polyoxyalkyleneoxy. Repeat units can be derived from alkenes, epoxides, aziridine, carbohydrate including the units that comprise modified celluloses such as hydroxyalkylcellulose; hydroxypropyl cellulose; hydroxypropyl methylcellulose; hydroxybutyl cellulose; and, hydroxybutyl methylcellulose or mixtures thereof. The repeat units may be derived from alkenes, or epoxides or mixtures thereof. The repeat units may be C<sub>2</sub>-C<sub>4</sub> alkyleneoxy groups, sometimes called alkoxy groups, preferably derived from C<sub>2</sub>-C<sub>4</sub> alkylene oxide. The repeat units may be C<sub>2</sub>-C<sub>4</sub> alkoxy groups, preferably ethoxy groups.

For the purposes of the present invention, the at least three consecutive repeat units form a polymeric constituent. The polymeric constituent may be covalently bound to the chromophore group, directly or indirectly via a linking group. Examples of suitable polymeric constituents include polyoxyalkylene chains having multiple repeating units. In one aspect, the polymeric constituents include polyoxyalkylene chains having from 2 to about 30 repeating units, from 2 to about 20 repeating units, from 2 to about 10 repeating units or even from about 3 or 4 to about 6 repeating units. Non-limiting examples of polyoxyalkylene chains include ethylene oxide, propylene oxide, glycidol oxide, butylene oxide and mixtures thereof.

**Surfactants—**

The compositions according to the present invention may comprise a surfactant or surfactant system wherein the surfactant can be selected from nonionic surfactants, anionic surfactants, cationic surfactants, ampholytic surfactants, zwitterionic surfactants, semi-polar nonionic surfactants and mixtures thereof.

The surfactant is typically present at a level of from about 0.01% to about 60%, from about 0.1% to about 60%, from about 1% to about 50% or even from about 5% to about 40%

by weight of the subject composition. Alternatively, the surfactant may be present at a level of from about 0.01% to about 60%, from about 0.01% to about 50%, from about 0.01% to about 40%, from about 0.1% to about 25%, from about 1% to about 10%, by weight of the subject composition.

**Chelating Agents—**

The compositions herein may contain a chelating agent. Suitable chelating agents include copper, iron and/or manganese chelating agents and mixtures thereof. When a chelating agent is used, the composition may comprise from about 0.1% to about 15% or even from about 3.0% to about 10% chelating agent by weight of the subject composition.

**Dye Transfer Inhibiting Agents—**

The compositions of the present invention may also include one or more dye transfer inhibiting agents. Suitable polymeric dye transfer inhibiting agents include, but are not limited to, polyvinylpyrrolidone polymers, polyamine N-oxide polymers, copolymers of N-vinylpyrrolidone and N-vinylimidazole, polyvinyloxazolidones and polyvinylimidazoles or mixtures thereof.

When present in a subject composition, the dye transfer inhibiting agents may be present at levels from about 0.0001% to about 10%, from about 0.01% to about 5% or even from about 0.1% to about 3% by weight of the composition.

**Dispersants—**

The compositions of the present invention can also contain dispersants. Suitable water-soluble organic materials include the homo- or co-polymeric acids or their salts, in which the polycarboxylic acid comprises at least two carboxyl radicals separated from each other by not more than two carbon atoms.

**Perfumes—**

The dispersed phase may comprise a perfume that may include materials selected from the group consisting of perfumes such as 3-(4-t-butylphenyl)-2-methyl propanal, 3-(4-t-butylphenyl)-propanal, 3-(4-isopropylphenyl)-2-methylpropanal, and 2,6-dimethyl-5-heptenal, alpha-damascone, beta-damascone, gamma-damascone, beta-damascenone, 6,7-dihydro-1,1,2,3,3-pentamethyl-4(5H)-indanone, methyl-7,3-dihydro-2H-1,5-benzodioxepine-3-one, 2-[2-(4-methyl-3-cyclohexenyl-1-yl)propyl]cyclopentan-2-one, 2-sec-butylcyclohexanone, and beta-dihydro ionone, linalool, ethyllinalool, tetrahydrolinalool, and dihydromyrcenol.

**Perfume Delivery Technologies—**

The fluid fabric enhancer compositions may comprise one or more perfume delivery technologies that stabilize and enhance the deposition and release of perfume ingredients from treated substrate. Such perfume delivery technologies can also be used to increase the longevity of perfume release from the treated substrate. Perfume delivery technologies, methods of making certain perfume delivery technologies and the uses of such perfume delivery technologies are disclosed in US 2007/0275866 A1.

In one aspect, the fluid fabric enhancer composition may comprise from about 0.001% to about 20%, or from about 0.01% to about 10%, or from about 0.05% to about 5%, or even from about 0.1% to about 0.5% by weight of the perfume delivery technology. In one aspect, said perfume delivery technologies may be selected from the group consisting of: perfume microcapsules, pro-perfumes, polymer particles, functionalized silicones, polymer assisted delivery, molecule assisted delivery, fiber assisted delivery, amine assisted delivery, cyclodextrins, starch encapsulated accord, zeolite and inorganic carrier, and mixtures thereof:

In one aspect, said perfume delivery technology may comprise microcapsules formed by at least partially surrounding a benefit agent with a wall material. Said benefit agent may include materials selected from the group consisting of perfumes such as 3-(4-t-butylphenyl)-2-methyl propanal, 3-(4-t-butylphenyl)-propanal, 3-(4-isopropylphenyl)-2-methylpropanal, 3-(3,4-methylenedioxophenyl)-2-methylpropanal, and 2,6-dimethyl-5-heptenal,  $\alpha$ -damascone,  $\beta$ -damascone,  $\alpha$ -damascenone, 6,7-dihydro-1,1,2,3,3-pentamethyl-4(5H)-indanone, methyl-7, 3-dihydro-2H-1,5-benzodioxepine-3-one, 2-[2-(4-methyl-3-cyclohexenyl-1-yl)propyl]cyclopentan-2-one, 2-sec-butylcyclohexanone, and  $\beta$ -dihydro ionone, linalool, ethyllinalool, tetrahydrolinalool, and dihydromyrcenol; silicone oils, waxes such as polyethylene waxes; essential oils such as fish oils, jasmine, camphor, lavender; skin coolants such as menthol, methyl lactate; vitamins such as Vitamin A and E; sunscreens; glycerine; catalysts such as manganese catalysts or bleach catalysts; bleach particles such as perborates; silicon dioxide particles; antiperspirant actives; cationic polymers and mixtures thereof. Suitable benefit agents can be obtained from Givaudan Corp. of Mount Olive, N.J., USA, International Flavors & Fragrances Corp. of South Brunswick, N.J., USA, or Firmenich Company of Geneva, Switzerland. In one aspect, the microcapsule wall material may comprise: melamine, polyacrylamide, silicones, silica, polystyrene, polyurea, polyurethanes, polyacrylate based materials, gelatin, styrene malic anhydride, polyamides, and mixtures thereof. In one aspect, said melamine wall material may comprise melamine cross-linked with formaldehyde, melamine-dimethoxyethanol crosslinked with formaldehyde, and mixtures thereof. In one aspect, said polystyrene wall material may comprise polystyrene cross-linked with divinylbenzene. In one aspect, said polyurea wall material may comprise urea crosslinked with formaldehyde, urea crosslinked with gluteraldehyde, polyisocyanate reacted with a polyamine, a polyamine reacted with an aldehyde, and mixtures thereof. In one aspect, said polyacrylate based materials may comprise polyacrylate formed from methylmethacrylate/dimethylaminomethyl methacrylate, polyacrylate formed from amine acrylate and/or methacrylate and strong acid, polyacrylate formed from carboxylic acid acrylate and/or methacrylate monomer and strong base, polyacrylate formed from an amine acrylate and/or methacrylate monomer and a carboxylic acid acrylate and/or carboxylic acid methacrylate monomer, and mixtures thereof. In one aspect, the perfume microcapsule may be coated with a deposition aid, a cationic polymer, a non-ionic polymer, an anionic polymer, or mixtures thereof. Suitable polymers may be selected from the group consisting of: polyvinylformaldehyde, partially hydroxylated polyvinylformaldehyde, polyvinylamine, polyethyleneimine, ethoxylated polyethyleneimine, polyvinylalcohol, polyacrylates, and combinations thereof. In one aspect, one or more types of microcapsules, for example two microcapsules types having different perfume benefit agents may be used.

In one aspect, said perfume delivery technology may comprise an amine reaction product (ARP) or a thiol reaction product. One may also use "reactive" polymeric amines and/or polymeric thiols in which the amine and/or thiol functionality is pre-reacted with one or more PRMs to form a reaction product. Typically the reactive amines are primary and/or secondary amines, and may be part of a polymer or a monomer (non-polymer). Such ARPs may also be mixed with additional PRMs to provide benefits of polymer-assisted delivery and/or amine-assisted delivery. Nonlimiting examples of polymeric amines include polymers based on

polyalkylimines, such as polyethyleneimine (PEI), or polyvinylamine (PVAm). Nonlimiting examples of monomeric (non-polymeric) amines include hydroxyl amines, such as 2-aminoethanol and its alkyl substituted derivatives, and aromatic amines such as anthranilates. The ARPs may be premixed with perfume or added separately in leave-on or rinse-off applications. In another aspect, a material that contains a heteroatom other than nitrogen and/or sulfur, for example oxygen, phosphorus or selenium, may be used as an alternative to amine compounds. In yet another aspect, the aforementioned alternative compounds can be used in combination with amine compounds. In yet another aspect, a single molecule may comprise an amine moiety and one or more of the alternative heteroatom moieties, for example, thiols, phosphines and selenols. The benefit may include improved delivery of perfume as well as controlled perfume release. Suitable ARPs as well as methods of making same can be found in USPA 2005/0003980 A1 and U.S. Pat. No. 6,413,920 B1.

#### 20 Processes of Making Products

The compositions of the present invention can be formulated into any suitable form and prepared by any process chosen by the formulator, non-limiting examples of which are described in Applicants examples and in US 2013/0109612 A1 which is incorporated herein by reference.

In one aspect, the compositions disclosed herein may be prepared by combining the components thereof in any convenient order and by mixing, e.g., agitating, the resulting component combination to form a phase stable fabric and/or home care composition. In one aspect, a fluid matrix may be formed containing at least a major proportion, or even substantially all, of the fluid components with the fluid components being thoroughly admixed by imparting shear agitation to this liquid combination. For example, rapid stirring with a mechanical stirrer may be employed.

#### METHOD OF USE

The compositions of the present invention may be used in any conventional manner. In short, they may be used in the same manner as products that are designed and produced by conventional methods and processes. For example, compositions of the present invention can be used to treat a *situs inter alia* a surface or fabric. Typically at least a portion of the *situs* is contacted with an aspect of Applicants' composition, in neat form or diluted in a wash liquor, and then the *situs* is optionally washed and/or rinsed. For purposes of the present invention, washing includes but is not limited to, scrubbing, and mechanical agitation. The fabric may comprise any fabric capable of being laundered in normal consumer use conditions. When the wash solvent is water, the water temperature typically ranges from about 5° C. to about 90° C. and, when the *situs* comprises a fabric, the water to fabric mass ratio is typically from about 1:1 to about 100:1.

The consumer products of the present invention may be used as liquid fabric enhancers wherein they are applied to a fabric and the fabric is then dried via line drying and/or drying the an automatic dryer.

In one aspect a liquor that comprises a sufficient amount of a composition that comprises a fabric softener active, a silicone polymer and a cationic polymer, to satisfy the following equation:

$$[(a)+x(b)+y(c)]w=z$$

wherein, a is a weight percent of fabric softener active other than silicone polymer in said composition, preferably

a is from about 0 to about 20 weight percent, more preferably a is from about 1 to about 15 weight percent, more preferably a is from about 3 to about 10 weight percent, more preferably a is from about 5 to about 10 weight percent, most preferably a is from about 7 to about 10 weight percent; b is the weight percent silicone polymer in said composition, preferably b is from about 0 to about 10 weight percent, more preferably b is from about 0.5 to about 5 weight percent, most preferably b is from about 1 to about 3 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about 40; x is a number from about 1 to about 5, preferably x is a number about 2; y is a number from about 1 to about 10, preferably y is a number from about 1 to about 5, more preferably y is a number about 2; z is a number from about 1 to about 10, preferably z is a number from about 1 to about 7, more preferably, z is a number from about 2 to about 4, is disclosed. Preferably, said composition that comprises a fabric softener active, a silicone polymer and a cationic polymer is a composition that is disclosed and/or claimed herein. In one aspect, said liquor may comprise an anionic surfactant, preferably 1 ppm to 1000 ppm, more preferably 1 ppm to 100 ppm of an anionic surfactant. In one aspect of said liquor a divided by b is a number from about 0.5 to about 10, preferably a divided by b is a number from about 1 to about 10, more preferably a divided by b is a number from about 1 to about 4, most preferably a divided by b is a number from about 2 to about 3.

In one aspect a method of treating a fabric comprising optionally washing, rinsing and/or drying a fabric then contacting said fabric with a liquor that comprises a sufficient amount of a composition that comprises a fabric softener active, a silicone polymer and a cationic polymer, to satisfy the following equation:

$$[(a)+x(b)+y(c)]w=z$$

wherein, a is a weight percent of fabric softener active other than silicone polymer in said composition, preferably a is from about 0 to about 20 weight percent, more preferably a is from about 1 to about 15 weight percent, more preferably a is from about 3 to about 10 weight percent, more preferably a is from about 5 to about 10 weight percent, most preferably a is from about 7 to about 10 weight percent; b is the weight percent silicone polymer in said composition, preferably b is from about 0 to about 10 weight percent, more preferably b is from about 0.5 to about 5 weight percent, most preferably b is from about 1 to about 3 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about 40; x is a number from about 1 to about 5, preferably x is a number about 2; y is a number from about 1 to about 10, preferably y is a number from about 1 to about 5, more preferably y is a number about 2; z is a number from about 1 to about 10, preferably z is a

number from about 1 to about 7, more preferably, z is a number from about 2 to about 4. Preferably, said composition that comprises a fabric softener active, a silicone polymer and a cationic polymer is a composition that is disclosed and/or claimed herein. In one aspect, said liquor may comprise an anionic surfactant, preferably 1 ppm to 1000 ppm, more preferably 1 ppm to 100 ppm of an anionic surfactant. In one aspect of said method a divided by b is a number from about 0.5 to about 10, preferably a divided by b is a number from about 1 to about 10, more preferably a divided by b is a number from about 1 to about 4, most preferably a divided by b is a number from about 2 to about 3.

In one aspect a method of treating a fabric comprising optionally washing, rinsing and/or drying a fabric then contacting said fabric with a liquor that comprises a sufficient amount of a composition that comprises a fabric softener active and a cationic polymer, to satisfy the following equation:

$$[(a)+y(c)]w=z$$

wherein, a is a weight percent fabric softener active in said composition, preferably a is from about 0 to about 20 weight percent, more preferably a is from about 1 to about 15 weight percent, more preferably a is from about 3 to about 10 weight percent, more preferably a is from about 5 to about 10 weight percent, most preferably a is from about 7 to about 10 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about 40; y is a number from about 1 to about 10, preferably y is a number from about 1 to about 5, more preferably y is a number about 2; z is a number from about 1 to about 10, preferably z is a number from about 1 to about 7, more preferably, z is a number from about 2 to about 4, is disclosed. Preferably, said composition that comprises a fabric softener active and a cationic polymer is a composition disclosed and/or claimed herein. In one aspect, said liquor may comprise an anionic surfactant, preferably 1 ppm to 1000 ppm, more preferably 1 ppm to 100 ppm of an anionic surfactant.

In one aspect a liquor that comprises a sufficient amount of a composition that comprises a fabric softener active and a cationic polymer, to satisfy the following equation:

$$[(a)+y(c)]w=z$$

wherein, a is a weight percent fabric softener active in said composition, preferably a is from about 0 to about 20 weight percent, more preferably a is from about 1 to about 15 weight percent, more preferably a is from about 3 to about 10 weight percent, more preferably a is from about 5 to about 10 weight percent, most preferably a is from about 7 to about 10 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about

40; y is a number from about 1 to about 10, preferably y is a number from about 1 to about 5, more preferably y is a number about 2; z is a number from about 1 to about 10, preferably z is a number from about 1 to about 7, more preferably, z is a number from about 2 to about 4. Preferably, said composition that comprises a fabric softener active and a cationic polymer is a composition that is disclosed and/or claimed herein. In one aspect, said liquor may comprise an anionic surfactant, preferably 1 ppm to 1000 ppm, more preferably 1 ppm to 100 ppm of an anionic surfactant.

A liquor that comprises a sufficient amount of a composition that comprises a fabric softener active, a silicone polymer and a cationic polymer, to satisfy the following equation:

$$[(a)+x(b)+y(c)]w=z$$

wherein, a is a weight percent of fabric softener active other than silicone polymer in said composition is disclosed. Preferably a is from about 0 to about 20 weight percent, more preferably a is from about 1 to about 15 weight percent, more preferably a is from about 3 to about 10 weight percent, more preferably a is from about 5 to about 10 weight percent, most preferably a is from about 7 to about 10 weight percent; b is the weight percent silicone polymer in said composition, preferably b is from about 0 to about 10 weight percent, more preferably b is from about 0.5 to about 5 weight percent, most preferably b is from about 1 to about 3 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about 40; x is a number from about 1 to about 5, preferably x is a number about 2; y is a number from about 1 to about 10, preferably y is a number from about 1 to about 5, more preferably y is a number about 2; z is a number from about 1 to about 10, preferably z is a number from about 1 to about 7, more preferably, z is a number from about 2 to about 4. Preferably, said composition that comprises a fabric softener active, a silicone polymer and a cationic polymer is a composition according to any preceding claim. Preferably, said liquor comprises an anionic surfactant, preferably 1 ppm to 1000 ppm, more preferably 1 ppm to 100 ppm of an anionic surfactant.

A liquor that comprises a sufficient amount of a composition that comprises a fabric softener active and a cationic polymer, to satisfy the following equation:

$$[(a)+y(c)]w=z$$

wherein, a is a weight percent fabric softener active in said composition is disclosed. Preferably a is from about 0 to about 20 weight percent, more preferably a is from about 1 to about 15 weight percent, more preferably a is from about 3 to about 10 weight percent, more preferably a is from about 5 to about 10 weight percent, most preferably a is from about 7 to about 10 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from

about 15 to about 40; y is a number from about 1 to about 10, preferably y is a number from about 1 to about 5, more preferably y is a number about 2; z is a number from about 1 to about 10, preferably z is a number from about 1 to about 7, more preferably, z is a number from about 2 to about 4. Preferably, said composition that comprises a fabric softener active and a cationic polymer is a composition according the composition's disclosed by Applicants in this specification. Preferably, said liquor comprises an anionic surfactant, preferably 1 ppm to 1000 ppm, more preferably 1 ppm to 100 ppm of an anionic surfactant.

#### Test Methods

##### 15 Viscosity Slope Method 1

The viscosity slope value quantifies the rate at which the viscosity increases as a function of increasing polymer concentration. The viscosity slope of a single polymer or of a dual polymer system is determined from viscosity measurements conducted on a series of aqueous solutions which span a range of polymer concentrations. The viscosity slope of a polymer is determined from a series of aqueous polymer solutions and which are termed polymer solvent solutions. The aqueous phase is prepared gravimetrically by adding hydrochloric acid to deionized water to reach a pH of about 3.0. A series of polymer solvent solutions are prepared to logarithmically span between 0.01 and 1 weight percent of the polymer in the aqueous phase. Each polymer solvent solutions is prepared gravimetrically by mixing the polymer and solvent with a SpeedMixer DAC 150 FVZ-K (made by FlackTek Inc. of Landrum, S.C.) for 1 minute at 2,500 RPM in a Max 60 cup or Max 100 cup to the target polymer weight percent of the polymer solvent solution. Polymer solvent solutions are allowed to come to equilibrium by resting for at least 24 hours. Viscosity as a function of shear rate of each polymer solvent solutions is measured at 40 different shear rates using an Anton Paar Rheometer with a DSR 301 measuring head and concentric cylinder geometry. The time differential for each measurement is logarithmic over the range of 180 and 10 seconds and the shear rate range for the measurements is 0.001 to 500 1/seconds (measurements taken from the low shear rate to the high shear rate).

Viscosity at a shear rate of 0.01 1/seconds as a function of 45 polymer weight percent of the polymer solvent solution is fit using the equation  $Y=bX^a$  wherein X is the polymer concentration in the solvent polymer solution, Y is the polymer solvent solution viscosity, b is the extrapolated solvent polymer solution viscosity when X is extrapolated to unity and the exponent a is polymer concentration viscosity scaling power over the polymer concentration range where the exponent a is the highest value.

##### Viscosity Slope Method 2

The viscosity slope value quantifies the rate at which the 55 viscosity increases as a function of increasing polymer concentration. The viscosity slope of a single polymer or of a dual polymer system is determined from viscosity measurements conducted on a series of aqueous solutions which span a range of polymer concentrations and which are termed polymer solvent solutions. Viscosity analyses are conducted using an Anton Paar Dynamic Shear Rheometer model DSR 301 Measuring Head, equipped with a 32-place Automatic Sample Changer (ASC) with reusable metal concentric cylinder geometry sample holders, and Rheoplus 60 software version 3.62 (all from Anton Paar GmbH, Graz, Austria). All polymer solutions are mixed using a high-speed motorized mixer, such as a Dual Asymmetric Centri-

fuge SpeedMixer model DAC 150 FVZ-K (FlackTek Inc., Landrum, S.C., USA) or equivalent.

The aqueous phase diluent for all of the aqueous polymer solutions is prepared by adding sufficient concentrated hydrochloric acid (e.g. 16 Baume, or 23% HCl) to deionized water until a pH of about 3.0 is achieved. The polymer(s) are combined with the aqueous phase diluent in a mixer cup (such as the Flacktek Speedmixer Max 100 or Max 60) that is compatible with the mixer to be used and is of a suitable size to hold a sample volume of 35 mL to 100 mL. Sufficient polymer is added to the aqueous phase diluent to achieve a concentration of between 8000-10000 ppm of the single polymer, or of the polymer 2 in the case of a dual polymer system, and to yield a volume of between 35 mL to 100 mL. The mixture of the polymer(s) and the aqueous phase is mixed for 4 minutes at a speed of 3500 RPM. After mixing, this initial polymer solvent solution is put aside to rest in a sealed container for at least 24 hours.

A single viscosity measurement is obtained from each of 32 polymer solvent solutions wherein each solution has a different concentration of polymer. These 32 polymer solvent solutions comprise a series of solutions that span the concentration range of 1000 ppm to 4000 ppm, with the solutions spaced at concentration intervals of approximately every 100 ppm. Each of the 32 polymer solvent solution concentrations is prepared gravimetrically by mixing the initial 8000-10000 ppm polymer solvent solution with sufficient additional aqueous phase diluent to result in a solution having the required target concentration and a volume of 35 mL to 100 mL, which is then mixed for 2 minutes at a speed of 3500 RPM. All of the resultant polymer solvent solutions are put aside to rest in a sealed cup for at least 24 hours. Polymer solutions are loaded into the concentric cylinder sample holders of the rheometer's ASC, using a pipette to fill each cylinder up to the line indicating a volume of 23 mL. The samples are stored in the ASC of the rheometer at a temperature of approximately 21° C. for up to 36 hours until measured. The viscosity of each of the 32 polymer solvent solutions is measured at the shear rate of 0.0105 l/s, and the viscosity value in units of Pa·s is recorded as soon as the value being measured is stable and consistent. The recorded viscosity values measured at a shear rate of 0.0105 l/s are paired with the value of the respective concentration of the polymer solvent solution measured. The resultant paired data values are plotted as 32 data points on a graph with viscosity in units of Pa·s on the x-axis, and polymer concentration in units of ppm on the y-axis. This data set is subsampled repeatedly to yield 30 subsets, wherein each subset comprises three consecutive data points. The subset creation process begins with the data point at the lowest polymer concentration and advances in sequence increasing toward the highest polymer concentration, until 30 unique subsets have been created. The subset creation process advances up to higher concentrations in steps of 1 data point at a time.

The three data points in each subset are fit with the following linear equation, using linear least squares regression, to determine the value of the exponent "a" for each of the 30 subsets:

$$Y=bX^a$$

wherein;

X is the polymer concentration in the solvent polymer solution (in ppm),

Y is the polymer solvent solution viscosity (in Pa·s)

b is the extrapolated solvent polymer solution viscosity (in Pa·s) when X is extrapolated to the value of 1 ppm, and the exponent a is a unitless parameter.

The Viscosity Slope value reported for the material being tested is the highest value calculated for the exponent "a", of all of the 30 values calculated for the exponent "a" from the 30 subsets.

5 Brookfield Viscosity

Brookfield viscosity is measured using a Brookfield DV-E viscometer. The liquid is contained in a glass jar, where the width of the glass jar is from about 5.5 to 6.5 cm and the height of the glass jar is from about 9 to about 11 cm. For 10 viscosities below 500 cPs, use spindle LV2 at 60 RPM, and to measure viscosities from 500 to 2,000 cPs, use spindle LV3 at 60 RPM.

The test is conducted in accordance with the instrument's instructions. Initial Brookfield viscosity is defined as the Brookfield viscosity measured within 24 hours of making the subject composition.

Physical Stability

Physical stability is assessed by visual observation of the 20 product in an undisturbed glass jar, where the width of the glass jar is from about 5.5 to 6.5 cm and the height of the glass jar is from about 9 to about 11 cm, after 4 weeks at 25° C. Using a ruler with millimeter graduation, the height of the liquid in the jar and the height of any visually observed 25 phase separation are measured. The Stability Index is defined as the height of the phase split divided by the height of the liquid in the glass jar. A product with no visually observable phase split is given a stability index of zero.

K Value for Polymer 2

30 The sample consists of a solution of 1% on polymer and 3% on NaCl. With this purpose the calculated amount of sample is weighted in a 50 mL volumetric flask, dissolved initially with a small amount of the 3%-NaCl solution and then the flask is filled until the calibration mark (under the 35 meniscus). A magnetic bar is introduced in the flask and stirred for 30 min. (There should be no visible supernatant, otherwise, the sample should be filtered). Finally, the solution is transferred to the Ubeholde Viscometer and attached to the machine. The sample is tempered for 10 min in the 40 machine at 25° C. and four measurements are carried out. The machine pumps the sample solution through the capillary and waits 10 min before the measurement starts. Subsequently the fourfold measurement takes place (if an outlier occurs, a new measurement takes place automatically).

45 Method for Determining Weight Percent Water Soluble Fraction for Polymer 1

For the determination of soluble and insoluble parts of the 50 polymer, fractionation experiments using Analytical ultracentrifugation were performed. Sedimentation velocity runs using a Beckman Optima XL-I (Beckman Instruments, Palo Alto, USA) with interference optical detection system (wavelength 675 nm) was used. The samples have been measured at polymer concentrations below critical polymer overlap concentration using salt solution to insure polyelectrolyte screening effect. The centrifugation speed was varied between 1000 rpm and 45,000 rpm.

The sedimentation coefficient, defined as a median value 60 for each fraction, and the concentration of one sedimenting fraction were determined using a standard analysis Software (SEDFIT) using the density and viscosity of the solvent, and a specific refractive index increment of the polymer. The sedimentation coefficient is in units of Sved (1 Sved=10<sup>-13</sup> seconds). The standard deviation for the determination of weight fraction and sedimentation coefficients of water soluble and crosslinked water-swellable polymers is 3%, 10% and up to 30% respectively. The weight percent of soluble polymer is the AUC value.

45

Measurement of Weight Average Molecular Weight (Mw) for Polymer 2

The weight average molecular weights of the cationic polymers of the present invention are determined by the technique of Size Exclusion Chromatography (SEC). SEC separation is carried out under conditions including three hydrophilic vinyl polymer network Novema gel columns, in distilled water in the presence of 0.1% (w/w) trifluoroacetate and 0.1 M NaCl at 35° C. Calibration is conducted with narrowly distributed poly(2-vinylpyridine)-standard of company PSS, Deutschland with molecular weights Mw=839 to M=2.070.000.

## EXAMPLES

## Example 1: Synthesis of Polymer 1 (P1.1)

An aqueous phase of water soluble components is prepared by admixing together the following components:

2.26 g (0.5 pphm) of citric acid-1-hydrate,  
2.25 g (0.2 pphm) of an aqueous solution (40%) of pentasodium diethylenetriaminepentaacetate,  
179.91 g (39.98 pphm) of water,  
0.90 g (0.2 pphm) of formic acid (Chain transfer agent)  
337.5 g (60.0 pphm) of methyl chloride quaternised dimethylaminoethylacrylate (DMA3\*MeCl, 80% aqueous solution), and  
360.00 g (40.0 pphm) of acrylamide (50% aqueous solution).

An oil phase is prepared by admixing together the following components:

73.47 g (2.45 pphm) of stabilizing agent B (15% in solvent) as stabilizing surfactant,  
124.58 g (5.22 pphm) of a polymeric stabiliser stearyl methacrylate-methacrylic acid copolymer (18.87% in solvent),  
354.15 g (78.7 pphm) of 2-ethylhexyl stearate, and  
105.93 g (23.54 pphm) of dearomatised hydrocarbon solvent with a boiling point between 160° C. till 190° C.  
4.50 g (0.01 pphm) Pentaerythrityl tri/tetraacrylate (PETA) (1% i-Propanol solution).

The two phases are mixed together in a ratio of 43 parts oil phase to 57 parts aqueous phase under high shear to form a water-in-oil emulsion. The resulting water-in-oil emulsion is transferred to a reactor equipped with nitrogen sparge tube, stirrer and thermometer. 0.11 g (0.025 pphm) 2,2-Azobis(2-methylbutyronitrile) is added and the emulsion is purged with nitrogen to remove oxygen.

Polymerisation is effected by addition of a redox couple of sodium metabisulphite and tertiary butyl hydroperoxide (one shot: 2.25 g (1% in solvent/0.005 pphm) stepwise such that is a temperature increase of 1.5° C./min. After the isotherm is completed the emulsion held at 85° C. for 60 minutes. Then residual monomer reduction with 18.25 g (0.25 pphm) tertiary butyl hydroperoxide (6.16% in solvent) and 21.56 g (0.25 pphm) sodium metabisulphite (5.22% in emulsion) is started (1.5 hours feeding time).

Vacuum distillation is carried out to remove water and volatile solvent to give a final product, i.e. a dispersion containing 50% polymer solids.

To this product addition is made of 63.0 g (14.0 pphm) of a fatty alcohol alkoxylate [alcohol C<sub>6</sub>-C<sub>17</sub>(secondary) poly(3-6)ethoxylate: 97% secondary alcohol ethoxylate+3% poly(ethylene oxide)], (CAS No. 84133-50-6).

46

Examples P1.1.1 to P1.1.14 in Table 1 are prepared according to the same process as the one described above for Example 1.

## Example 2: Synthesis of Polymer 2 (P1.2)

An aqueous phase of water soluble components is prepared by admixing together the following components:

2.26 g (0.5 pphm) of citric acid-1-hydrate,  
2.25 g (0.2 pphm) of an aqueous solution (40%) of pentasodium diethylenetriaminepentaacetate,  
170.55 g (37.90 pphm) of water,  
9.00 g (0.10 pphm) of tetraethylammonium chloride (TAAC) (5% aqueous solution)  
0.90 g (0.2 pphm) of formic acid  
337.5 g (60.0 pphm) of methyl chloride quaternised dimethylaminoethylacrylate (DMA3\*MeCl 80% aqueous solution), and  
360.00 g (40.0 pphm) of acrylamide (50% aqueous solution).

An oil phase is prepared by admixing together the following components:

73.47 g (2.45 pphm) of stabilizing agent B (15% in solvent) as stabilizing surfactant,  
124.58 g (5.22 pphm) of a polymeric stabiliser stearyl methacrylate-methacrylic acid copolymer (18.87% in solvent),  
354.15 g (78.7 pphm) of 2-ethylhexyl stearate, and  
111.65 g (24.81 pphm) of dearomatised hydrocarbon solvent with a boiling point between 160° C. till 190° C.

The two phases are mixed together in a ratio of 43 parts oil phase to 57 parts aqueous phase under high shear to form a water-in-oil emulsion. The resulting water-in-oil emulsion is transferred to a reactor equipped with nitrogen sparge tube, stirrer and thermometer. 0.11 g (0.025 pphm) 2,2-Azobis(2-methylbutyronitrile) is added and the emulsion is purged with nitrogen to remove oxygen.

Polymerisation is effected by addition of a redox couple of sodium metabisulphite and tertiary butyl hydroperoxide (one shot: 2.25 g (1% in solvent/0.005 pphm)) stepwise such that is a temperature increase of 1.5° C./min. After the isotherm is completed the emulsion held at 85° C. for 60 minutes. Then residual monomer reduction with 18.25 g (0.25 pphm) tertiary butyl hydroperoxide (6.16% in solvent) and 21.56 g (0.25 pphm) sodium metabisulphite (5.22% in emulsion) is started (1.5 hours feeding time).

Vacuum distillation is carried out to remove water and volatile solvent to give a final product, i.e. a dispersion containing 50% polymer solids.

To this product addition is made of 63.0 g (14.0 pphm) of a fatty alcohol alkoxylate [alcohol C<sub>6</sub>-C<sub>17</sub>(secondary) poly(3-6)ethoxylate: 97% secondary alcohol ethoxylate+3% poly(ethylene oxide)], (CAS No. 84133-50-6).

Examples P1.2.1 to P1.2.28 in Table 1 are prepared according to the same process as the one described above for Example 2.

## Example 3: Synthesis of Polymer 1 (P1.3)

An aqueous phase of water soluble components is prepared by admixing together the following components:

2.26 g (0.5 pphm) of citric acid-1-hydrate,  
2.25 g (0.2 pphm) of an aqueous solution (40%) of pentasodium diethylenetriaminepentaacetate,  
170.55 g (37.90 pphm) of water,

9.00 g (0.10 pphm) of Trimethylolpropane tris(polyethylene glycol ether) triacrylate (TMPTA EOx) (5% aqueous solution)  
 0.90 g (0.2 pphm) of formic acid  
 337.50 g (60.0 pphm) of methyl chloride quaternised dimethylaminoethylacrylate (DMA3\*MeCl 80% aqueous solution), and  
 360.00 g (40.0 pphm) of acrylamide (50% aqueous solution).

An oil phase is prepared by admixing together the following components:

73.47 g (2.45 pphm) of stabilizing agent B (15% in solvent) as stabilizing surfactant,  
 124.58 g (5.22 pphm) of a polymeric stabiliser stearyl methacrylate-methacrylic acid copolymer (18.87% in solvent),  
 354.15 g (78.7 pphm) of 2-ethylhexyl stearate, and  
 111.65 g (24.81 pphm) of dearomatised hydrocarbon solvent with a boiling point between 160° C. till 190° C.

The two phases are mixed together in a ratio of 43 parts oil phase to 57 parts aqueous phase under high shear to form a water-in-oil emulsion. The resulting water-in-oil emulsion

is transferred to a reactor equipped with nitrogen sparge tube, stirrer and thermometer. 0.11 g (0.025 pphm) 2,2-Azobis(2-methylbutyronitrile) is added and the emulsion is purged with nitrogen to remove oxygen.

5 Polymerisation is effected by addition of a redox couple of sodium metabisulphite and tertiary butyl hydroperoxide (one shot: 2.25 g (1% in solvent/0.005 pphm) stepwise such that is a temperature increase of 1.5° C./min. After the isotherm is completed the emulsion held at 85° C. for 60 minutes. Then residual monomer reduction with 18.25 g (0.25 pphm) tertiary butyl hydroperoxide (6.16% in solvent) and 21.56 g (0.25 pphm) sodium metabisulphite (5.22% in emulsion) is started (1.5 hours feeding time).

10 Vacuum distillation is carried out to remove water and volatile solvent to give a final product, i.e. a dispersion containing 50% polymer solids.

15 To this product addition is made of 63.0 g (14.0 pphm) of a fatty alcohol alkoxylate [alcohol C<sub>6</sub>-C<sub>17</sub>(secondary) poly (3-6)ethoxylate: 97% secondary alcohol ethoxylate+3% 20 poly(ethylene oxide)], (CAS No. 84133-50-6).

Examples P1.3.1 to P1.3.2 in Table 1 is prepared according to the same process as the one described above for Example 3.

TABLE 1

| Example | Examples of Polymer 1      |                   |                   |                                |              |             |                  | Chain transfer agent (pphm) | Reaction speed ° C./min. |
|---------|----------------------------|-------------------|-------------------|--------------------------------|--------------|-------------|------------------|-----------------------------|--------------------------|
|         | Stabilizing agent B (pphm) | DMA3* MeCl (pphm) | Acrylamide (pphm) | Methylen bis acrylamide (pphm) | PETIA (pphm) | TAAC (pphm) | TMPTA-EOx (pphm) |                             |                          |
| P1.1    | 2.45                       | 60                | 40                |                                | 0.01         |             |                  | 0.2                         | +1.5                     |
| P1.1.1  | 2.45                       | 60                | 40                |                                | 0.05         |             |                  | 0.2                         | +1.5                     |
| P1.1.2  | 2.45                       | 60                | 40                |                                | 0.035        |             |                  | 0.2                         | +1.5                     |
| P1.1.3  | 2.45                       | 60                | 40                |                                | 0.035        |             |                  | 0.2                         | +1.5                     |
| P1.1.4  | 2.45                       | 60                | 40                |                                | 0.035        |             |                  | 0.2                         | +1.5                     |
| P1.1.5  | 2.45                       | 60                | 40                |                                | 0.035        |             |                  | 0.2                         | +1.5                     |
| P1.1.6  | 2.45                       | 60                | 40                |                                | 0.035        |             |                  | 0.1                         | +1.5                     |
| P1.1.7  | 2.45                       | 60                | 40                |                                | 0.035        |             |                  | 0.05                        | +1.5                     |
| P1.1.8  | 2.45                       | 60                | 40                |                                | 0.04         |             |                  | 0.1                         | +1.5                     |
| P1.1.9  | 2.45                       | 60                | 40                |                                | 0.035        |             |                  | 0.085                       | +1.5                     |
| P1.1.10 | 2.45                       | 60                | 40                |                                | 0.025        |             |                  |                             | +1.5                     |
| P1.1.11 | 2.45                       | 60                | 40                |                                | 0.035        |             |                  | 0.07                        | +1.5                     |
| P1.1.12 | 2.45                       | 40                | 60                |                                |              | 0.02        |                  | 0.05                        | +1.5                     |
| P1.1.13 | 2.45                       | DADMAC            | HEA               |                                |              | 0.03        |                  | 0.1                         | +1.5                     |
|         |                            | 40                | 60                |                                |              |             |                  |                             |                          |
| P1.1.14 | 2.45                       | DMAEMA* MeCl 60   | 40                |                                | 0.035        |             |                  | 0.2                         | +1.5                     |
| P1.2    | 2.45                       | 60                | 40                |                                | 0.1          |             |                  | 0.2                         | +1.5                     |
| P1.2.1  | 2.45                       | 60                | 40                |                                | 0.075        |             |                  | 0.2                         | +1.5                     |
| P1.2.2  | 2.45                       | 60                | 40                |                                | 0.075        |             |                  | 0.2                         | +1.5                     |
| P1.2.3  | 2.45                       | 60                | 40                |                                | 0.04         |             |                  | 0.1                         | +1.5                     |
| P1.2.4  | 2.45                       | 60                | 40                |                                | 0.049        |             |                  | 0                           | +1                       |
| P1.2.5  | 2.45                       | 60                | 40                |                                | 0.045        |             |                  | 0.05                        | +1.5                     |
| P1.2.6  | 2.45                       | 60                | 40                |                                | 0.04         |             |                  | 0.025                       | +1.5                     |
| P1.2.7  | 2.45                       | 60                | 40                |                                | 0.045        |             |                  | 0.0375                      | +1.5                     |
| P1.2.8  | 2.45                       | 60                | 40                |                                | 0.04         |             |                  | 0.025                       | +1.5                     |
| P1.2.9  | 2.45                       | 60                | 40                |                                | 0.045        |             |                  | 0.0375                      | +1.5                     |
| P1.2.10 | 2.45                       | 60                | 40                |                                | 0.04         |             |                  | 0.025                       | +1.5                     |
| P1.2.11 | 2.45                       | 60                | 40                |                                | 0.04         |             |                  | 0.025                       | +1.5                     |
| P1.2.12 | 2.45                       | 60                | 40                |                                | 0.04         |             |                  | 0.025                       | +1.5                     |
| P1.2.13 | 2.45                       | 60                | 40                |                                | 0.04         |             |                  | 0.025                       | +1.5                     |
| P1.2.14 | 2.45                       | 60                | 40                |                                | 0.04         |             |                  | 0.0125                      | +1.5                     |
| P1.2.15 | 2.45                       | 60                | 40                |                                | 0.04         |             |                  | 0.0125                      | +1.5                     |
| P1.2.16 | 2.45                       | 60                | 40                |                                | 0.04         |             |                  | 0.0125                      | +1.5                     |
| P1.2.17 | 2.45                       | 60                | 40                |                                | 0.04         |             |                  | 0.0125                      | +1.5                     |
| P1.2.18 | 2.45                       | 60                | 40                |                                | 0.04         |             |                  | 0.0188                      | +1.5                     |
| P1.2.19 | 2.45                       | 60                | 40                |                                | 0.04         |             |                  | 0.0125                      | +1.5                     |
| P1.2.20 | 2.45                       | 60                | 40                |                                | 0.04         |             |                  | 0.0125                      | +1.5                     |
| P1.2.21 | 2.45                       | 60                | 40                |                                | 0.04         |             |                  | 0.0125                      | +1.5                     |
| P1.2.22 |                            |                   |                   |                                |              | 0.04        |                  | 0.0125                      | +1.5                     |
| P1.2.23 | 2.45                       | MAPTAC            | AM                |                                |              | 0.03        |                  | 0.02                        | +1.5                     |
|         |                            |                   | 70                |                                | 30           |             |                  |                             |                          |

TABLE 1-continued

| Example | Examples of Polymer 1      |                   |                   |                                |              |             |                  |                             |                          |
|---------|----------------------------|-------------------|-------------------|--------------------------------|--------------|-------------|------------------|-----------------------------|--------------------------|
|         | Stabilizing agent B (pphm) | DMA3* MeCl (pphm) | Acrylamide (pphm) | Methylen bis acrylamide (pphm) | PETIA (pphm) | TAAC (pphm) | TMPTA-EOx (pphm) | Chain transfer agent (pphm) | Reaction-speed ° C./min. |
| P1.2.24 | 2.45                       | 70                | 30                |                                |              | 0.01        |                  | 0.02                        | +1.5                     |
| P1.2.25 | 2.45                       | 60                | 40                | 0.07                           |              |             |                  | 0.02                        | +1.5                     |
| P1.2.26 | 2.45                       | 60                | 40                |                                |              | 0.049       |                  |                             | +1.5                     |
| P1.2.27 | 2.45                       | 60                | 40                |                                |              | 0.04        | 0.125            |                             | +1.5                     |
| P1.2.28 | 2.45                       | 60                | 40                |                                |              | 0.04        | 0.125            |                             | +1.0                     |
| P1.3.1  | 2.45                       | 60                | 40                |                                |              |             | 0.1              | 0.2                         | +1.5                     |
| P1.3.2  | 2.45                       | 60                | 40                |                                |              |             | 0.04             | 0.05                        | +1.5                     |

DMA3\*MeCl = Dimethylamino Ethyl Acrylate methochloride

DMAEMA\*MeCl = DimethylAmino Ethyl MethAcrylate methochloride

AM = Acrylamide

HEA = Hydroxyethyl acrylate

MAPTAC = Trimethylaminopropyl ammonium acrylamide chloride

PETIA = pentaerythrityl triacrylate/pentaerythrityl tetraacrylate

TAAC = tetraallylammonium chloride

TMPTA = trimethylolp propane tris(polyethylene glycol ether) triacrylate

**Example 4: Synthesis for Polymer 2 that are Made by Solution Polymerization**

Into a 2 L glass reactor equipped with a thermometer, an anchor stirrer, a nitrogen feed and a reflux condenser, 0.57 g of a 40% aqueous solution of Trilon C, 10.96 g (0.057 mole) of citric acid and 747 g of ion exchanged water were charged. Thereafter, the solution was purged by a flow of nitrogen gas and the inner temperature was elevated to 70° C. Afterwards 0.57 g of Wako V50 in 36.09 g of ion exchanged water were added thereto, 90.06 g (0.634 mole) of 50% aqueous acrylamide solution and 230.05 g (1.188 mole) of a 84% solution of dimethylaminoethylacrylate-methochloride in 25.56 g of ion exchanged water were added continuously to the reaction system over 2 hours 45 min while keeping the inner temperature at 70° C. Thereafter, the inner temperature was kept at 70° C. for 1 hour to complete the reaction. Afterwards 1.15 g of Wako V50 in 7.16 g of ion exchanged water were added at once and the reaction stirred for 2 h, before cooling down. The obtained product is a 21.9% aqueous polymer solution having a pH of 2.8 and a K-value of 55.5.

**Example 5: Synthesis for Polymer 2 that are Made by Solution Polymerization**

25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7

TABLE 2-continued

| Examples of Polymer Two |                       |             |             |                |                |                   |                          |         |
|-------------------------|-----------------------|-------------|-------------|----------------|----------------|-------------------|--------------------------|---------|
| Polymer                 | Polymerization Method | Mono 1 Type | Mono 2 Type | Mono 1 (wt. %) | Mono 2 (wt. %) | Cross-linker Type | Cross-linker Level [ppm] | K Value |
| P2.13                   | Solution              | DMA3MeCl    | AM          | 40             | 60             | N/A               | 0                        | 25      |
| P2.14                   | Solution              | DMA3MeCl    | AM          | 60             | 40             | N/A               | 0                        | 20      |

Dimethylamino Ethyl Acrylate methochloride (DMA3MeCl)

DimethylAmino Ethyl MethAcrylate methochloride (DMAEMA)

Acrylamide (AM)

Hydroxyethyl acrylate (HEA)

Dialkyldimethyl ammonium chloride (DADMAC)

Trimethylaminopropyl ammonium acrylamide chloride (MAPTAC)

Tetra allyl ammonium chloride (TAAC)

Methylene bisacrylamide (MBA)

Acrylic Acid (AA)

## Example 6

## -continued

Compositions having the listed amounts of materials are made by combining the ammonium quat active with water using shear then the other materials are combined with the ammonium quat/water and mixed to form a fabric softener composition. Adjunct ingredients such as perfume, dye and stabilizer may be added as desired.

20

25

| Silicone Active          | Ammonium Quat Active | Polymer 1 From Table 1          | Polymer 2 From Table 2     |
|--------------------------|----------------------|---------------------------------|----------------------------|
| 1.0-3.0%; or<br>1.5-2.5% | 7-10%; or<br>4-8%    | 0.03-0.15%;<br>or<br>0.04-0.12% | or<br>0.03-0.12%           |
| 0-5.0%;<br>0-5.0%;       | 1-18%;<br>2-14%;     | 0.01-0.50%;<br>0.02-0.20%;      | 0.01-0.35%;<br>0.02-0.15%; |

| Silicone Active    | Ammonium Quat Active | Polymer 1 From Table 1     | Polymer 2 From Table 2     |
|--------------------|----------------------|----------------------------|----------------------------|
| 0-0.5%;<br>0-5.0%; | 1-18%;<br>2-14%;     | 0.01-0.50%;<br>0.02-0.20%; | 0.01-0.35%;<br>0.02-0.15%; |

30

## Example 7. Fabric Softener Products

|                                         | (% wt)  |         |         |         |         |         |
|-----------------------------------------|---------|---------|---------|---------|---------|---------|
|                                         | F1      | F2      | F3      | F4      | F5      | F6      |
| FSA <sup>a</sup>                        | 11.2    | 7       | 9       | —       | —       | —       |
| FSA <sup>b</sup>                        | —       | —       | —       | —       | —       | 6       |
| FSA <sup>c</sup>                        | —       | —       | —       | 14.5    | 13      | —       |
| Coco oil                                | 0.6     | 0.5     | 0.45    | —       | —       | —       |
| Low MW Alcohol <sup>d</sup>             | 1.11    | 0.7     | 0.9     | 1.5     | 1.3     | 0.5     |
| Perfume                                 | 1.75    | 0.6     | 2.1     | 1.5     | 2       | 1.2     |
| Perfume encapsulate <sup>e</sup>        | 0.19    | 0.6     | 0.5     | 0.25    | 0.6     | 0.4     |
| Calcium Chloride (ppm)                  | 0.06    | 0.03    | 0.025   | 0.12    | 0.06    | —       |
| Chelant <sup>f</sup>                    | 0.005   | 0.005   | 0.005   | 0.005   | 0.005   | 0.006   |
| Preservative <sup>g</sup>               | 0.04    | 0.04    | 0.02    | 0.04    | 0.03    | 0.05    |
| Acidulant (Formic Acid)                 | 0.051   | 0.03    | 0.04    | 0.02    | 0.03    | —       |
| Antifoam <sup>h</sup>                   | —       | —       | —       | —       | —       | 0.05    |
| Polymer 1 <sup>i</sup>                  | 0.17    | 0.15    | 0.2     | 0.12    | 0.16    | 0.35    |
| Polymer 2 <sup>i</sup>                  | —       | —       | —       | —       | —       | —       |
| Water soluble dialkyl quat <sup>j</sup> | 0.25    | 0.2     | 0.1     | 0.5     | —       | 0.25    |
| Dispersant <sup>k</sup>                 | —       | —       | —       | —       | —       | —       |
| Stabilizing Surfactant <sup>l</sup>     | —       | —       | —       | —       | —       | 0.1     |
| PDMS emulsion <sup>m</sup>              | —       | —       | 0.5     | —       | 2       | —       |
| Amino-functional                        | 3       | 2       | —       | 1       | —       | —       |
| Organosiloxane Polymer                  | —       | —       | —       | —       | —       | —       |
| Dye (ppm)                               | 0.03    | 0.03    | 0.02    | 0.04    | 0.04    | 0.02    |
| Hydrochloric Acid                       | 0.0075  | 0.0075  | 0.008   | 0.01    | 0.01    | 0.01    |
| Deionized Water                         | Balance | Balance | Balance | Balance | Balance | Balance |

|                                  | (% wt) |       |      |       |       |       |
|----------------------------------|--------|-------|------|-------|-------|-------|
|                                  | F7     | F8    | F9   | F10   | F11   | F12   |
| FSA <sup>a</sup>                 | 12     | 9.5   | 8    | 6.5   | 5.3   | 2.5   |
| FSA <sup>b</sup>                 | —      | —     | —    | —     | —     | —     |
| FSA <sup>c</sup>                 | —      | —     | —    | —     | —     | —     |
| Coco oil                         | 0.6    | 0.475 | 0.4  | 0.325 | 0.265 | 0.125 |
| Low MW Alcohol <sup>d</sup>      | 0.9    | 1.11  | 0.95 | 1.05  | 0.78  | 0.35  |
| Perfume                          | 3      | 1.41  | 1.00 | 0.55  | 1.55  | 1     |
| Perfume encapsulate <sup>e</sup> | 0.6    | 0.15  | 0.25 | 0.62  | 0.98  | 0.25  |
| Calcium Chloride (ppm)           | 0.07   | 0.23  | 0.16 | —     | —     | —     |
| Chelant <sup>f</sup>             | 0.005  | 0.01  | 0.01 | 0.01  | 0.01  | 0.01  |

-continued

|                                         |         |         |         |         |         |         |
|-----------------------------------------|---------|---------|---------|---------|---------|---------|
| Preservative <sup>g</sup>               | 0.04    | —       | —       | —       | —       | —       |
| Acidulent (Formic Acid)                 | 0.05    | 0.06    | 0.06    | 0.06    | 0.06    | —       |
| Antifoam <sup>h</sup>                   | —       | —       | —       | —       | —       | —       |
| Polymer 1 <sup>i</sup>                  | 0.14    | 0.08    | 0.12    | 0.06    | 0.04    | 0.08    |
| Polymer 2 <sup>i</sup>                  | —       | 0.12    | 0.12    | 0.08    | 0.04    | —       |
| Water soluble dialkyl quat <sup>j</sup> | 0.35    | 0.11    | 0.11    | —       | 0.52    | 0.1     |
| Dispersant <sup>k</sup>                 | —       | —       | —       | —       | —       | —       |
| Stabilizing Surfactant <sup>l</sup>     | —       | —       | —       | —       | —       | —       |
| PDMS emulsion <sup>m</sup>              | 2       | —       | —       | —       | —       | 3       |
| Amino-functional                        | —       | —       | —       | —       | —       | —       |
| Organosiloxane Polymer                  | —       | —       | —       | —       | —       | —       |
| Dye (ppm)                               | 0.02    | 0.03    | 0.03    | 0.03    | 0.03    | 0.02    |
| Hydrochloric Acid                       | 0.005   | 0.03    | 0.03    | 0.03    | 0.03    | 0.02    |
| Deionized Water                         | Balance | Balance | Balance | Balance | Balance | Balance |

|                                         | (% wt)  |         |         |         |         |         |
|-----------------------------------------|---------|---------|---------|---------|---------|---------|
|                                         | F13     | F14     | F15     | F16     | F17     | F18     |
| FSA <sup>a</sup>                        | 14.7    | 14.7    | 11.1    | 9.5     | 6.25    | 5.1     |
| FSA <sup>b</sup>                        | —       | —       | —       | —       | —       | —       |
| FSA <sup>c</sup>                        | —       | —       | —       | —       | —       | —       |
| Coco oil                                | 0.735   | 0.735   | 0.555   | 0.475   | 0.3125  | 0.255   |
| Low MW Alcohol <sup>d</sup>             | 0.88    | 0.58    | 0.45    | 0.52    | 0.33    | 0.22    |
| Perfume                                 | 1.65    | 1.65    | 1.65    | 1.4     | 3.12    | 0.65    |
| Perfume encapsulate <sup>e</sup>        | 0.26    | 0.26    | 0.26    | 0.43    | 0.26    | 0.75    |
| Calcium Chloride (ppm)                  | 0.23    | 0.23    | —       | 0.23    | 0.23    | 0.23    |
| Chelant <sup>f</sup>                    | 0.01    | 0.01    | 0.01    | 0.01    | 0.01    | 0.01    |
| Preservative <sup>g</sup>               | —       | 0.001   | —       | 0.001   | 0.001   | 0.001   |
| Acidulent (Formic Acid)                 | 0.06    | —       | —       | —       | —       | —       |
| Antifoam <sup>h</sup>                   | —       | —       | —       | —       | —       | —       |
| Polymer 1 <sup>i</sup>                  | 0.07    | 0.07    | 0.05    | 0.06    | 0.06    | 0.06    |
| Polymer 2 <sup>i</sup>                  | 0.09    | 0.09    | 0.05    | 0.09    | 0.09    | 0.09    |
| Water soluble dialkyl quat <sup>j</sup> | —       | 0.29    | 0.29    | 0.29    | 0.29    | 0.29    |
| Dispersant <sup>k</sup>                 | —       | —       | —       | —       | —       | —       |
| Stabilizing Surfactant <sup>l</sup>     | —       | —       | —       | —       | —       | —       |
| PDMS emulsion <sup>m</sup>              | —       | 1.12    | —       | —       | —       | —       |
| Amino-functional                        | —       | —       | 1.8     | 2.2     | 3.1     | 1.8     |
| Organosiloxane Polymer                  | —       | —       | —       | —       | —       | —       |
| Dye (ppm)                               | 0.03    | 0.03    | 0.03    | 0.03    | 0.03    | 0.03    |
| Hydrochloric Acid                       | 0.03    | 0.03    | 0.03    | 0.03    | 0.03    | 0.03    |
| Deionized Water                         | Balance | Balance | Balance | Balance | Balance | Balance |

|                                         | (% wt)  |         |         |         |         |         |
|-----------------------------------------|---------|---------|---------|---------|---------|---------|
|                                         | F19     | F20     | F21     | F22     | F23     | F24     |
| FSA <sup>a</sup>                        | 14.7    | 6.25    | 10.2    | 5       | 11      | 15      |
| FSA <sup>b</sup>                        | —       | —       | —       | —       | —       | —       |
| FSA <sup>c</sup>                        | —       | —       | —       | —       | —       | —       |
| Coco oil                                | 0.735   | 0.3125  | 0.51    | 0.3     | 0.6     | 0.8     |
| Low MW Alcohol <sup>d</sup>             | 0.58    | 0.11    | 0.58    | 0.95    | 0.95    | 0.95    |
| Perfume                                 | 1.65    | 0.35    | 1.65    | 1.00    | 1.00    | 1.00    |
| Perfume encapsulate <sup>e</sup>        | 0.26    | 1.33    | 0.26    | 0.25    | 0.25    | 0.25    |
| Calcium Chloride (ppm)                  | 0.23    | 0.42    | 0.23    | 0.16    | 0.16    | 0.16    |
| Chelant <sup>f</sup>                    | 0.01    | 0.01    | 0.01    | 0.01    | 0.01    | 0.01    |
| Preservative <sup>g</sup>               | 0.001   | —       | 0.001   | —       | —       | —       |
| Acidulent (Formic Acid)                 | —       | 0.06    | —       | 0.06    | 0.06    | 0.06    |
| Antifoam <sup>h</sup>                   | —       | 0.02    | —       | —       | —       | —       |
| Polymer 1 <sup>i</sup>                  | 0.03    | 0.25    | 0.01    | 0.12    | 0.12    | 0.12    |
| Polymer 2 <sup>i</sup>                  | 0.04    | 0.18    | 0.02    | 0.12    | 0.12    | 0.12    |
| Water soluble dialkyl quat <sup>j</sup> | 0.29    | 0.29    | 0.29    | 0.11    | 0.11    | 0.11    |
| Dispersant <sup>k</sup>                 | —       | —       | 0.15    | —       | —       | —       |
| Stabilizing Surfactant <sup>l</sup>     | —       | —       | 0.45    | —       | —       | —       |
| PDMS emulsion <sup>m</sup>              | 1.12    | —       | 0.85    | —       | —       | —       |
| Amino-functional                        | —       | 3.1     | 0.95    | —       | —       | —       |
| Organosiloxane Polymer                  | —       | —       | —       | —       | —       | —       |
| Dye (ppm)                               | 0.03    | 0.03    | —       | 0.03    | 0.03    | 0.03    |
| Hydrochloric Acid                       | 0.03    | 0.03    | 0.03    | 0.03    | 0.03    | 0.03    |
| Deionized Water                         | Balance | Balance | Balance | Balance | Balance | Balance |

|                  | (% wt) |     |     |     |
|------------------|--------|-----|-----|-----|
|                  | F25    | F26 | F27 | F28 |
| FSA <sup>a</sup> | 15     | 11  | 8   | 5   |
| FSA <sup>b</sup> | —      | —   | —   | —   |
| FSA <sup>c</sup> | —      | —   | —   | —   |
| Coco oil         | 0.8    | 0.6 | 0.4 | 0.3 |

|                                         |         |         |         |         |
|-----------------------------------------|---------|---------|---------|---------|
| Low MW Alcohol <sup>d</sup>             | 0.95    | 0.95    | 0.95    | 0.95    |
| Perfume                                 | 1.00    | 1.00    | 1.00    | 1.00    |
| Perfume encapsulate <sup>e</sup>        | 0.25    | 0.25    | 0.25    | 0.25    |
| Calcium Chloride (ppm)                  | 0.12    | 0.12    | 0.12    | 0.12    |
| Chelant <sup>f</sup>                    | 0.005   | 0.005   | 0.005   | 0.005   |
| Preservative <sup>g</sup>               | 0.04    | 0.04    | 0.04    | 0.04    |
| Acidulent (Formic Acid)                 | 0.02    | 0.02    | 0.02    | 0.02    |
| Antifoam <sup>h</sup>                   | —       | —       | —       | —       |
| Polymer 1 <sup>i</sup>                  | 0.08    | 0.08    | 0.08    | 0.08    |
| Polymer 2 <sup>i</sup>                  | —       | —       | —       | —       |
| Water soluble dialkyl quat <sup>j</sup> | —       | —       | —       | —       |
| Dispersant <sup>k</sup>                 | —       | —       | —       | —       |
| Stabilizing Surfactant <sup>l</sup>     | —       | —       | —       | —       |
| PDMS emulsion <sup>m</sup>              | —       | —       | —       | —       |
| Amino-functional                        | 1       | 1       | 1       | 1       |
| Organosiloxane Polymer                  | —       | —       | —       | —       |
| Dye (ppm)                               | 0.04    | 0.04    | 0.04    | 0.04    |
| Hydrochloric Acid                       | 0.01    | 0.01    | 0.01    | 0.01    |
| Deionized Water                         | Balance | Balance | Balance | Balance |

|                                         | (% wt)  |         |         |         |         |         |
|-----------------------------------------|---------|---------|---------|---------|---------|---------|
|                                         | F29     | F30     | F31     | F32     | F33     | F34     |
| FSA <sup>a</sup>                        | 3.5     | —       | 9.5     | 8.0     | 5.5     | —       |
| FSA <sup>b</sup>                        | —       | 7.5     | —       | —       | —       | 7.5     |
| Coco oil                                | —       | —       | —       | —       | 0.4     | —       |
| Low MW Alcohol <sup>d</sup>             | —       | —       | —       | —       | 1.3     | 0.5     |
| Perfume                                 | 1.75    | 0.6     | 1.0     | 0.65    | 2.5     | 1.2     |
| Perfume encapsulate <sup>e</sup>        | 0.19    | 0.65    | 0.35    | 0.25    | 0.11    | 0.4     |
| Calcium Chloride (ppm)                  | 0.06    | 0.03    | 0.025   | 0.12    | 0.06    | —       |
| Magnesium Chloride                      | —       | —       | —       | 0.3     | 0.08    | 0.5     |
| Chelant <sup>f</sup>                    | 0.005   | 0.005   | 0.005   | 0.005   | 0.005   | 0.006   |
| Preservative <sup>g</sup>               | 0.04    | 0.04    | 0.02    | 0.04    | 0.03    | 0.05    |
| Acidulent (Formic Acid)                 | 0.051   | 0.03    | 0.04    | 0.02    | 0.03    | —       |
| Antifoam <sup>h</sup>                   | —       | —       | —       | —       | —       | 0.05    |
| Polymer 1 <sup>i</sup>                  | 0.07    | 0.14    | 0.10    | 0.16    | 0.18    | 0.30    |
| Polymer 2 <sup>i</sup>                  | 0.03    | 0.06    | 0.05    | 0.04    | 0.02    | 0.15    |
| Water soluble dialkyl quat <sup>j</sup> | 0.2     | —       | —       | —       | —       | 0.3     |
| PDMS emulsion <sup>m</sup>              | —       | —       | —       | —       | 2       | —       |
| Amino-functional                        | —       | —       | —       | —       | —       | 1.5     |
| Organosiloxane Polymer                  | —       | —       | —       | —       | —       | —       |
| Dye (ppm)                               | 0.03    | 0.03    | 0.02    | 0.04    | 0.04    | 0.02    |
| Hydrochloric Acid                       | 0.0075  | 0.0075  | 0.008   | 0.01    | 0.01    | 0.01    |
| Deionized Water                         | Balance | Balance | Balance | Balance | Balance | Balance |

|                                  | (% wt) |       |       |       |       |
|----------------------------------|--------|-------|-------|-------|-------|
|                                  | F35    | F36   | F37   | F38   | F39   |
| FSA <sup>a</sup>                 | 8.0    | 8.0   | 8.0   | 8.0   | 9.5   |
| Perfume                          | 1.0    | 1.0   | 1.0   | 1.0   | 1.0   |
| Perfume encapsulate <sup>e</sup> | 0.35   | 0.35  | 0.35  | 0.35  | 0.35  |
| Calcium Chloride (ppm)           | —      | —     | —     | —     | 0.075 |
| Magnesium Chloride               | 0.7    | 0.7   | 0.7   | 0.7   | 0.7   |
| Chelant <sup>f</sup>             | 0.01   | 0.01  | 0.01  | 0.01  | 0.01  |
| Preservative <sup>g</sup>        | 0.001  | 0.001 | 0.001 | 0.001 | 0.001 |
| Formic Acid                      | 0.05   | 0.05  | 0.05  | 0.05  | 0.05  |
| Polymer 1 <sup>i</sup>           | 0.10   | 0.12  | 0.09  | 0.075 | —     |
| Polymer 2 <sup>i</sup>           | —      | —     | —     | —     | 0.15  |
| Dye (ppm)                        | 0.03   | 0.03  | 0.02  | 0.04  | 0.04  |

|                   |         |         |         |         |         |
|-------------------|---------|---------|---------|---------|---------|
| Hydrochloric Acid | 0.006   | 0.006   | 0.006   | 0.006   | 0.006   |
| Deionized Water   | Balance | Balance | Balance | Balance | Balance |

<sup>a</sup> N,N-di(alkanoyloxyethyl)-N,N-dimethylammonium chloride where alkyl consists predominantly of C16-C18 alkyl chains with an IV value of about 20 available from Evonik

<sup>b</sup> Methyl bis[ethyl (tallowate)-2-hydroxyethyl ammonium methyl sulfate available from Stepan

<sup>c</sup> N,N-di(alkanoyloxyethyl)-N,N-dimethylammonium chloride where alkyl consists predominantly of C16-C18 alkyl chains with an IV value of about 52 available from Evonik

<sup>d</sup> Low molecular weight alcohol such as ethanol or isopropanol

<sup>e</sup> Perfume microcapsules available ex Appleton Papers, Inc.

<sup>f</sup> Diethylenetriaminepentacetic acid or hydroxyl ethylened-1,1-diphosphonic acid

<sup>g</sup> 1,2-Benzisothiazolin-3-ONE (BIT) under the trade name Proxel available from Lonza

<sup>h</sup> Silicone antifoam agent available from Dow Corning ® under the trade name DC2310

<sup>i</sup> Polymer 1 are chosen from Table 1 and Polymer 2 are chosen from Table 2

<sup>j</sup> Didecyldimethyl ammonium chloride under the trade name Bardac ® 2280 or Hydrogenated tallowalkyl(2-ethylhexyl)dimethyl ammonium methylsulfate from AkzoNobel under the trade name Arquad ® HTL8-MS

<sup>k</sup> Non-ionic surfactant from BASF under the trade name Lutensol ® XL-70

<sup>l</sup> Non-ionic surfactant, such as TWEEN 20™ or TAE80 (tallow ethoxylated alcohol, with average degree of ethoxylation of 80)

<sup>m</sup> Polydimethylsiloxane emulsion from Dow Corning under the trade name DC346 ®.

<sup>n</sup> Rheovis CDE ® commercially available from BASF

#### Example 8. Fabric Preparation Example

Fabrics are assessed using Kenmore FS 600 and/or 80 series washer machines. Wash Machines are set at: 32° C./15°C wash/rinse temperature, 6 gpg hardness, normal cycle, and medium load (64 liters). Fabric bundles consist of 2.5 kilograms of clean fabric consisting of 100% cotton. Test swatches are included with this bundle and comprise of 100% cotton Euro Touch terrycloth towels (purchased from Standard Textile, Inc. Cincinnati, Ohio). Prior to treatment with any test products, the fabric bundles are stripped according to the Fabric Preparation-Stripping and Desizing procedure before running the test. Tide Free liquid detergent (1x recommended dose) is added under the surface of the water after the machine is at least half full. Once the water stops flowing and the washer begins to agitate, the clean fabric bundle is added. When the machine is almost full with rinse water, and before agitation has begun, the fabric care testing composition is slowly added (1x dose), ensuring that none of the fabric care testing composition comes in direct contact with the test swatches or fabric bundle. When the wash/rinse cycle is complete, each wet fabric bundle is transferred to a corresponding dryer. The dryer used is a Maytag commercial series (or equivalent) electric dryer, with the timer set for 55 minutes on the cotton/high heat/timed dry setting. This process is repeated for a total of three (3) complete wash-dry cycles. After the third drying cycle and once the dryer stops, 12 Terry towels from each fabric bundle are removed for actives deposition analysis. The fabrics are then placed in a constant Temperature/Relative Humidity (21° C., 50% relative humidity) controlled grading room for 12-24 hours and then graded for softness and/or actives deposition.

The Fabric Preparation-Stripping and Desizing procedure includes washing the clean fabric bundle (2.5 Kg of fabric comprising 100% cotton) including the test swatches of 100% cotton EuroTouch terrycloth towels for 5 consecutive wash cycles followed by a drying cycle. AATCC (American Association of Textile Chemists and Colorists) High Efficiency (HE) liquid detergent is used to strip/de-size the test swatch fabrics and clean fabric bundle (1x recommended dose per wash cycle). The wash conditions are as follows: Kenmore FS 600 and/or 80 series wash machines (or equivalent), set at: 48° C./48° C. wash/rinse temperature, water hardness equal to 0 gpg, normal wash cycle, and medium sized load (64 liters). The dryer timer is set for 55 minutes on the cotton/high/timed dry setting.

#### Example 9: Silicone on Fabric Measurement Method

Silicone is extracted from approximately 0.5 grams of fabric (previously treated according to the test swatch treat-

ment procedure) with 12 mL of either 50:50 toluene:methylisobutyl ketone or 15:85 ethanol:methylisobutyl ketone in 20 mL scintillation vials. The vials are agitated on a pulsed vortexer for 30 minutes. The silicone in the extract is quantified using inductively coupled plasma optical emission spectrometry (ICP-OES). ICP calibration standards of known silicone concentration are made using the same or a structurally comparable type of silicone raw material as the products being tested. The working range of the method is 8-2300 µg silicone per gram of fabric. Concentrations greater than 2300 µg silicone per gram of fabric can be assessed by subsequent dilution. Deposition efficiency index of silicone is determined by calculating as a percentage, how much silicone is recovered, via the aforementioned extraction and measurement technique, versus how much is delivered via the formulation examples. The analysis is performed on terrycloth towels (EuroSoft towel, sourced from Standard Textile, Inc, Cincinnati, Ohio) that are treated according to the wash procedure outlined herein.

#### Example 10: Example for Determining the Recovery Index for Organo Siloxane Polymer

The Recovery Index is measured using a Tensile and Compression Tester Instrument, such as the Instron Model 5565 (Instron Corp., Norwood, Mass., U.S.A.). The instrument is configured by selecting the following settings: the mode is Tensile Extension; the Waveform Shape is Triangle; the Maximum Strain is 10%, the Rate is 0.83 mm/sec, the number of Cycles is 4; and the Hold time is 15 seconds between cycles.

- 1) Determine the weight of one approximately 25.4 cm square swatch of 100% cotton woven fabric, (a suitable fabric is the Mercerized Combed Cotton Warp Sateen, Product Code 479, available from Testfabrics Inc., West Pittston, Pa., USA).
- 2) Determine the amount of organo siloxane polymer required to deposit 5 mg of the polymer per gram of fabric swatch and weigh that amount into a 50 ml plastic centrifuge tube with a lid.
- 3) Dilute the organo siloxane polymer to 1.3 times the weight of the swatch with a solvent that completely dissolves or disperses the organo siloxane polymer (examples: isopropyl alcohol, THF, N,N-dimethylacetamide, water).
- 4) Thoroughly disperse or dissolve organo siloxane with shaking or vortex stirring as needed.
- 5) Place fabric swatch lying flat into a stainless steel tray that is larger than the swatch.
- 6) Pour the organo siloxane polymer solution over the entire swatch as evenly as possible.

- 7) Fold the swatch twice to quarter, then roll it up while gently squeezing to disperse solution to the entire swatch.
- 8) Unfold and repeat Step 7, folding in the opposite direction
- 9) To make a control swatch, repeat the procedure described above using 1.3× weight of solvent only (nil active).
- 10) Lay each swatch on a separate piece of aluminum foil and place in a fume hood to dry overnight.
- 11) Cure each swatch in an oven with appropriate ventilation at 90° C. for 5 minutes, (a suitable oven is the Mathis Labdryer, with 1500 rpm fan rotation) (Werner Mathis AG, Oberhasli, Switzerland).
- 12) Condition fabrics in a constant temperature (21° C.+/-2° C.) and humidity (50% RH+/-5% RH) room for at least 6 hours.
- 13) With scissors, cut the edge of one entire side of each swatch in the warp direction and carefully remove fabric threads one at a time without stressing the fabric until an even edge is achieved.
- 14) Cut 4 strips of fabric from each swatch (die or rotary cut), parallel to the even edge, that are 2.54 cm wide and at least 10 cm long
- 15) Evenly clamp the top and bottom (narrower edges) of the fabric strip into the 2.54 cm grips on the tensile tester instrument with a 2.54 cm gap setting, loading a small amount of force (0.1N-0.2N) on the sample.
- 16) Strain to 10% at 0.83 mm/s and return to 2.54 cm gap at the same rate.
- 17) Release bottom clamp and re-clamp sample during the hold cycle, loading 0.1N-0.2N of force on the sample.
- 18) Repeat Steps 15-16 until 4 hysteresis cycles have been completed for the sample.
- 19) Analyze 4 fabric samples per treatment swatch by the above method and average the tensile strain values recorded at 0.1N unload for Cycle 4. Recovery is calculated as follows:

$$\% \text{ Recovery} = \frac{(10 - \text{Tensile Strain at 0.1N})}{10} \times 100$$

$$20) \text{ Recovery Index} = \frac{\% \text{ Recovery of Treatment}}{\% \text{ Recovery of Control}}$$

#### Example 11: Fabric Friction Measures Example

For the examples cited a Thwing-Albert FP2250 Friction/Peel Tester with a 2 kilogram force load cell is used to measure fabric to fabric friction. (Thwing Albert Instrument Company, West Berlin, N.J.). The sled is a clamping style sled with a 6.4 by 6.4 cm footprint and weighs 200 g (Thwing Albert Model Number 00225-218). A comparable instrument to measure fabric to fabric friction would be an instrument capable of measuring frictional properties of a horizontal surface. A 200 gram sled that has footprint of 6.4 cm by 6.4 cm and has a way to securely clamp the fabric without stretching it would be comparable. It is important, though, that the sled remains parallel to and in contact with the fabric during the measurement. The distance between the load cell to the sled is set at 10.2 cm. The crosshead arm height to the sample stage is adjusted to 25 mm (measured from the bottom of the cross arm to the top of the stage) to ensure that the sled remains parallel to and in contact with the fabric during the measurement. The following settings are used to make the measure:

|                       |             |
|-----------------------|-------------|
| T2 (Kinetic Measure): | 10.0 sec    |
| Total Time:           | 20.0 sec    |
| Test Rate:            | 20.0 cm/min |

5

The 11.4 cm×6.4 cm cut fabric piece is attached, per FIG. 2, to the clamping sled (10) with the face down (11) (so that the face of the fabric on the sled is pulled across the face of the fabric on the sample plate) which corresponds to friction sled cut (7) of FIG. 1. Referring to FIG. 2, the loops of the fabric on the sled (12) are oriented such that when the sled (10) is pulled, the fabric (11) is pulled against the nap of the loops (12) of the test fabric cloth (see FIG. 2). The fabric from which the sled sample is cut is attached to the sample table such that the sled drags over the area labeled "Friction Drag Area" (8) as seen in FIG. 1. The loop orientation (13) is such that when the sled is pulled over the fabric it is pulled against the loops (13) (see FIG. 2). Direction arrow (14) indicates direction of sled (10) movement.

The sled is placed on the fabric and attached to the load cell. The crosshead is moved until the load cell registers between ~1.0-2.0 gf, and is then moved back until the load reads 0.0 gf. At this point the sled drag is commenced and the Kinetic Coefficient of Friction (kCOF) recorded at least every second during the sled drag. The kinetic coefficient of friction is averaged over the time frame starting at 10 seconds and ending at 20 seconds for the sled speed set at 20.0 cm/min. For each treatment, at least ten replicate fabrics are measured.

#### Example 12: Perfume Release Headspace Over Fabric Measurement Method

Fabrics were treated with compositions of the current invention using the Fabric Preparation method described within. The perfume release over fabric data was generated using standard dynamic purge and trap analysis of fabric headspace with gas chromatography (GC) and detector to measure perfume headspace levels. The headspace analysis was performed on wet and dry fabric and total perfume counts were normalized to one of the test legs to show the relative benefit of compositions of the present invention. For example, a wet fabric perfume headspace (normalized to 1.0) shows that Leg C has 50% more perfume headspace above the wet fabric than Leg A.

GC—Detector Analysis of Fabric Samples for Perfume Release: A total of 3 pieces of treated fabric 1"×2" in size are placed into 3 clean 40 ml bottles (for a total of 9 fabrics) and allowed to equilibrate for about 1 hour. The fabric pieces are cut from different fabrics within each load to account for fabric-to-fabric variability. Instrument conditions should be modified to achieve adequate PRM signal detection while avoiding peak saturation. A DB 5 column was used with 20 sec sample collection with a ramp of 40-180° C. at 5-10 deg/sec and a detector temperature of 35° C.

Olfactive Panel—The Olfactive Panel is run with about 20 qualified panelists. Each panelist is given fabrics treated with compositions of the current invention to grade. A Panel typically consists of 4 to 6 treatments, which are randomized. Each panelist grades the fabric treatments for intensity (scale 0-100) based on the anchors that are prepared to provide intensities representing 20, 50, and 80 on a scale of 0-100). On the scale, 0 refers to a fabric with no scent intensity and 100 to a fabric with extremely strong/overpowering scent intensity. Panelists sniff fabrics and record an intensity grade for the Dry Fabric Odor (DFO). Optionally, panelists can sniff and grade fabrics after rubbing the dry fabric to give grades for Rubbed Fabric Odor (RFO). Optionally, panelists can evaluate other touch points such as wet fabric odor (WFO).

Fabrics were treated with compositions of the current invention using the Fabric Preparation method described within. The softness of the fabrics on a 1-10 scale were then evaluated by at least 20 panelists. The results are shown below in Tables 3, 4 and 5.

TABLE 3

| Softener Active Level (%) | Softener Active Dose (g) | Polymer 1                             | Polymer 2                             | Softness (1-10) | Wet Fabric Perfume Headspace (Normalized to 1.0) | Dry Fabric Perfume Headspace (Normalized to 1.0) |
|---------------------------|--------------------------|---------------------------------------|---------------------------------------|-----------------|--------------------------------------------------|--------------------------------------------------|
| 14.7                      | 45                       | 0.08% Rheovis CDE ®                   | —                                     | 6.0             | 1.0x                                             | 1.0x                                             |
| 9.5                       | 45                       | 0.12% Polymer 1 selected from Table 1 | 0.12% Polymer 2 selected from Table 2 | 7.2             | 1.5x                                             | 1.4x                                             |
| 13.3                      | 45                       | —                                     | —                                     | 6.1             |                                                  |                                                  |
| 9.5                       | 45                       | 0.08% Rheovis CDE ®                   | —                                     | 3.9             | 1.2x                                             | 0.9x                                             |

Rheovis CDE ® commercially available from BASF

25

TABLE 4

| Formula from Example 7 | Dose (g) | Polymer 1                       | Polymer 2                       | Dry Fabric Perfume Headspace (Normalized to 1) |
|------------------------|----------|---------------------------------|---------------------------------|------------------------------------------------|
| F25                    | 45       | Rheovis CDE ®                   | —                               | 1.0                                            |
| F26                    | 45       | Rheovis CDE ®                   | —                               | 1.1                                            |
| F27                    | 45       | Rheovis CDE ®                   | —                               | 0.6                                            |
| F28                    | 45       | Rheovis CDE ®                   | —                               | 0.5                                            |
| F24                    | 45       | Polymer 1 selected from Table 1 | Polymer 2 selected from Table 2 | 0.8                                            |

TABLE 4-continued

| 30 | Formula from Example 7                         | Dose (g) | Polymer 1                       | Polymer 2                       | Dry Fabric Perfume Headspace (Normalized to 1) |
|----|------------------------------------------------|----------|---------------------------------|---------------------------------|------------------------------------------------|
| 35 | F23                                            | 45       | Polymer 1 selected from Table 1 | Polymer 2 selected from Table 2 | 1.6                                            |
|    | F9                                             | 45       | Polymer 1 selected from Table 1 | Polymer 2 selected from Table 2 | 1.5                                            |
|    | F22                                            | 45       | Polymer 1 selected from Table 1 | Polymer 2 selected from Table 2 | 1.2                                            |
| 40 | Rheovis CDE ® commercially available from BASF |          |                                 |                                 |                                                |

TABLE 5

| Softener Active Level (%) | Dose (g) | Polymer 1 (%)                         | Polymer 2 (%)                         | Perfume Headspace (Normalized to 1) | Softness (coefficient of friction) | Viscosity (2 months) | Stability Index |
|---------------------------|----------|---------------------------------------|---------------------------------------|-------------------------------------|------------------------------------|----------------------|-----------------|
| 14.7                      | 25       | 0.15% Rheovis CDE ®                   | —                                     | 1.0                                 | 1.12                               | 0                    |                 |
| 8                         | 25       | 0.15% Rheovis CDE ®                   | —                                     | 0.9                                 | 1.38                               | 144                  | 0               |
| 8                         | 25       | 0.25% Polymer 1 selected from Table 1 | —                                     | 1.1                                 | 1.03                               | 4600                 | 0               |
| 8                         | 25       | 0.25% Zetag ®                         | —                                     | 1.7                                 | 1.03                               | 990                  | 0               |
| 8                         | 25       | —                                     | 0.25% Polymer 2 selected from Table 2 | 1.0                                 | 1.11                               | 96                   | 0.3             |
| 8                         | 25       | 0.12% Zetag ®                         | 0.12% Polymer 2 selected from Table 2 | 1.9                                 | 1.14                               | 234                  | 0               |

TABLE 5-continued

| Softener | Active | Perfume          |                                                | Softness                          | Viscosity                    | Stability  |       |
|----------|--------|------------------|------------------------------------------------|-----------------------------------|------------------------------|------------|-------|
| Level    | Dose   | Polymer 1        | Polymer 2                                      | Headspace<br>(Normalized<br>to 1) | (coefficient<br>of friction) | (2 months) | Index |
| (%)      | (g)    | (%)              | (%)                                            |                                   |                              |            |       |
| 8        | 25     | 0.06%<br>Zetag ® | 0.12%<br>Polymer 2<br>selected<br>from Table 2 | 1.4                               | 1.14                         | 107        | 0     |

Rheovis CDE ® commercially available from BASF

Zetag 9066FS ® commercially available from BASF

Example 14

Fabrics were treated with compositions of the current invention. The polymers in the fabric softener compositions were characterized using the methods described within. After treatment and drying for three consecutive times, the amount of silicone deposited on the fabrics was measured using the silicone extraction example described within. The results are shown below in Table 6 and Table 7.

TABLE 6

| Fabric softener composition examples for 30 g of product dosed/2700 g fabric treated |              |                            |                   |                   |                                       |                              |                                            |
|--------------------------------------------------------------------------------------|--------------|----------------------------|-------------------|-------------------|---------------------------------------|------------------------------|--------------------------------------------|
| Exam-<br>ple                                                                         | Example<br>7 | Formula<br>from<br>Table 1 | Polymer<br>1 Type | Polymer<br>2 Type | Viscosity<br>Slope of<br>Polymer<br>1 | Polymer<br>1<br>AUC<br>value | Silicone                                   |
|                                                                                      |              |                            |                   |                   |                                       |                              | Deposition<br>[ug<br>silicone/g<br>fabric] |
| 1                                                                                    | F1           | P1.2.4                     | None              |                   | 2.7                                   | 28%                          | 344                                        |
| 2                                                                                    | F1           | P1.2.6                     | None              |                   | 3.3                                   | 30%                          | 319                                        |
| CE1                                                                                  | F1           | Rheovis<br>CDE ®           | None              |                   |                                       |                              | 268                                        |

Rheovis CDE ® commercially available from BASF

TABLE 7

| Fabric softener composition examples for 24 g of product dosed/2700 g fabric treated |              |                            |                   |                   |                                       |                              |                                            |
|--------------------------------------------------------------------------------------|--------------|----------------------------|-------------------|-------------------|---------------------------------------|------------------------------|--------------------------------------------|
| Exam-<br>ple                                                                         | Example<br>7 | Formula<br>from<br>Table 1 | Polymer<br>1 Type | Polymer<br>2 Type | Viscosity<br>Slope of<br>Polymer<br>1 | Polymer<br>1<br>AUC<br>value | Silicone                                   |
|                                                                                      |              |                            |                   |                   |                                       |                              | Deposition<br>[ug<br>silicone/g<br>fabric] |
| 1                                                                                    | F1           | P1.1.5                     | None              |                   | 5.0                                   | 34%                          | 230                                        |
| 2                                                                                    | F1           | P1.1.10                    | None              |                   | 4.4                                   | 25%                          | 148                                        |
| 3                                                                                    | F1           | P1.2.26                    | None              |                   | 3.6                                   | 22%                          | 152                                        |
| 4                                                                                    | F1           | P1.2.27                    | None              |                   |                                       | 31%                          | 142                                        |
| 5                                                                                    | F1           | P1.2.28                    | None              |                   | 4.1                                   | 18%                          | 115                                        |
| 6                                                                                    | F1           | P1.3.1                     | None              |                   | 3.6                                   | 27%                          | 242                                        |
| CE1                                                                                  | F1           | Rheovis<br>CDE ®           | None              |                   |                                       |                              | 77                                         |

Rheovis CDE ® commercially available from BASF

Example 15

Fabrics were treated with compositions of the current invention using the Fabric Preparation method described within. The results are show below in Tables 8.

TABLE 8

Fabric softener composition examples for 49 g of product dosed/2700 g fabric treated.

| Formula<br>from<br>Example 7 | Dose<br>(g) | Polymer 1             | Polymer 2                | Dry<br>Fabric<br>Odor<br>(DFO)/<br>Rubbed<br>DFO |
|------------------------------|-------------|-----------------------|--------------------------|--------------------------------------------------|
| F35                          | 49          | selected from Table 1 |                          | 21.5/56.0                                        |
| F36                          | 49          | selected from Table 1 | selected from<br>Table 2 | 26.0/60.0                                        |
| F37                          | 49          | selected from Table 1 | selected from<br>Table 2 | 29.5/62.5                                        |
| F38                          | 49          | selected from Table 1 | selected from<br>Table 2 | 24.5/59.0                                        |
| F39                          | 49          | Rheovis CDE ®         |                          | 22.5/57.0                                        |

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "about 40 mm" is intended to mean "about 40 mm".

All documents cited in the Detailed Description of the Invention are, in relevant part, incorporated herein by reference; the citation of any document is not to be construed as an admission that it is prior art with respect to the present invention. To the extent that any meaning or definition of a term in this document conflicts with any meaning or definition of the same term in a document incorporated by reference, the meaning or definition assigned to the term in this written document shall govern.

While particular aspects of the present invention have been illustrated and described, it would be obvious to those skilled in the art that various other changes and modifications can be made without departing from the spirit and scope of the invention. It is therefore intended to cover in the appended claims all such changes and modifications that are within the scope of this invention.

55 What is claimed is:

1. A composition comprising, based upon total composition weight:

a.) from about 0.15% to about 0.2%, of a polymeric material comprising a first polymer and a second polymer, said first polymer being derived from the polymerization of from about 5 to 100 mole percent of a cationic vinyl addition monomer, from about 0 to 95 mole percent of a non-ionic vinyl addition monomer, from about 50 ppm to 1,950 ppm of a cross-linking agent comprising three or more ethylenic functions, and 0 ppm to about 10,000 ppm of a chain transfer agent,

said second polymer being derived from the polymerization of from about 5 to 99 mole percent of a cationic vinyl addition monomer, from about 0 to 95 mole percent of a non-ionic vinyl addition monomer, from about 1 to 49 percent of an anionic vinyl addition monomer, with the proviso that the sum of the cationic vinyl addition monomer, non-ionic vinyl addition monomer, and anionic vinyl addition monomer will not exceed 100 mole percent; from about 0 ppm to 45 ppm of a cross-linking agent comprising two or more ethylenic functions, and 0 ppm to about 10,000 ppm of a chain transfer agent,

wherein the cationic monomers are selected from the group consisting of methyl chloride quaternized dimethyl aminoethylammonium acrylate, methyl chloride quaternized dimethyl aminoethylammonium methacrylate and mixtures thereof, and the non-ionic monomers are acrylamide; and

b.) from about 8% to about 12%, based on total composition weight, of a fabric softener active that is an alkyl quaternary ammonium compound; and

c.) a perfume delivery system, said perfume delivery system comprising one or more types of perfume microcapsules;

said composition being a fabric and home care product.

2. The composition of claim 1 wherein, said polymeric material comprises a first polymer and a second polymer, said first polymer being derived from the polymerization of from about 10 to 95 mole percent of a cationic vinyl addition monomer; from about 10 to 90 mole percent of a non-ionic vinyl addition monomer; from about 55 ppm to 1,900 ppm of a cross-linking agent comprising three or more ethylenic functions; and 0 ppm to about 10,000 ppm of a chain transfer agent;

said second polymer being derived from the polymerization of from about 10 to 95 mole percent of a cationic vinyl addition monomer; from about 5 to 90 mole percent of a non-ionic vinyl addition monomer; from about 1 to 45 mole percent of an anionic vinyl addition monomer, with the proviso that the sum of the cationic vinyl addition monomer, non-ionic vinyl addition monomer, and anionic vinyl addition monomer will not exceed 100 mole percent; from about 0 ppm to 40 ppm of a cross-linking agent comprising two or more ethylenic functions; and from 0 ppm to about 10,000 ppm of a chain transfer agent.

3. A composition according to claim 1, further comprising a second fabric softener active selected from the group consisting of a silicone polymer, a polysaccharide, a clay, an amine, a fatty ester, a dispersible polyolefin, a polymer latex and mixtures thereof.

4. A composition according to claim 3, wherein; said silicone polymer is selected from the group consisting of cyclic silicones, polydimethylsiloxanes, amino-silicones, cationic silicones, silicone polyethers, silicone resins, silicone urethanes, and mixtures thereof;

said polysaccharide comprises a cationic starch;

said clay comprises a smectite clay; said dispersible polyolefin is selected from the group consisting of polyethylene, polypropylene and mixtures thereof; and

said fatty ester is selected from the group consisting of a polyglycerol ester, a sucrose ester, a glycerol ester and mixtures thereof.

5. A composition according to claim 3, said composition comprises, in addition to said fabric softener active, from

about 0.001% to about 5%, of a stabilizer that comprises a alkyl quaternary ammonium compound.

6. A composition according to claim 1, wherein said fabric softener active comprises a material selected from the group consisting of monoesterquats, diesterquats, triesterquats, and mixtures thereof.

7. A composition according to claim 1 wherein the fabric softening active has an Iodine Value of between 0-140 or when said fabric softening active comprises a partially hydrogenated fatty acid quaternary ammonium compound said fabric softening active has a Iodine Value of 25-60.

8. A composition according to claim 1, said composition further comprising a silicone polymer.

9. A composition according to claim 1, wherein said polymer is derived from an anionic monomer selected from the group consisting of acrylic acid, methacrylic acid, itaconic acid, crotonic acid, maleic acid, fumaric acid, monomers performing a sulfonic acid or phosphonic acid functions, and their salts;

wherein said cross-linking agent is selected from the group consisting of methylene bisacrylamide, ethylene glycol diacrylate, polyethylene glycol dimethacrylate, diacryamide, triallylamine, cyanomethylacrylate, vinyl oxyethylacrylate or methacrylate and formaldehyde, glyoxal, divinylbenzene, tetraallyl ammonium chloride, allyl acrylates, allyl methacrylates, diacrylates and dimethacrylates of glycols or polyglycols, butadiene, 1,7-octadiene, allylacrylamides or allylmethacrylamides, bisacrylamidoacetic acid, N,N'-methylenebisacrylamide or polyol polyallyl ethers, pentaerythritol triacrylate, pentaerythritol tetraacrylate, tetraallyl ammonium chloride, 1,1,1-trimethylolpropane tri(meth)acrylate; and tri- and tetramethacrylates of polyglycols; or polyol polyallyl ethers, ditrimethylolpropane tetraacrylate, pentaerythritol tetraacrylate ethoxylate, pentaerythritol tetramethacrylate, pentaerythritol triacrylate ethoxylate, triethanolamine trimethacrylate, 1,1,1-trimethylolpropane triacrylate, 1,1,1-trimethylolpropane triacrylate ethoxylate, trimethylolpropane tri(polyethylene glycol ether) triacrylate, 1,1,1-trimethylolpropane trimethacrylate, tris-(2-hydroxyethyl)-1,3,5-triazine-2,4,6-trione triacrylate, tris-(2-hydroxyethyl)-1,3,5-triazine-2,4,6-trione trimethacrylate, dipentaerythritol pentaacrylate, 3-(3-[dimethyl-(vinyl)-silyl]-oxy)-1,1,5,5-tetramethyl-1,5-divinyl-3-trisiloxanyl)-propyl methacrylate, dipentaerythritol hexaacrylate, 1-(2-propenoxy)-2,2-bis[(2-propenoxy)-methyl]-butane, trimethacrylic acid-1,3,5-triazin-2,4,6-triyltri-2,1-ethandiy ester, glycerine triacrylate, propoxylated, 1,3,5-triacyloylhexahydro-1,3,5-triazine, 1,3-dimethyl-1,1,3,3-tetravinyl disiloxane, pentaerythritol tetravinyl ether, 1,3-dimethyl-1,1,3,3-tetravinyl disiloxane, (Ethoxy)-trivinylsilane, (Methyl)-trivinylsilane, 1,1,3,5,5-pentamethyl-1,3,5-trivinyltrisiloxane, 1,3,5-trimethyl-1,3,5-trivinylcyclotrisiloxane, 2,4,6-trimethyl-2,4,6-trivinylcyclotrisiloxane, 1,3,5-trimethyl-1,3,5-trivinyltrisiloxane, tris-(2-butane oxime)-vinylsilane, 1,2,4-trivinylcyclohexane, trivinylphosphine, trivinylsilane, methyltrivinylsilane, phenyltrivinylsilane, triallylamine, triallyl citrate, triallyl phosphate, triallylphosphine, triallyl phosphite, triallylsilane, 1,3,5-triallyl-1,3,5-triazine-2,4,6(1H,3H,5H)-trione, trimellitic acid triallyl ester, trimethylallyl isocyanurate, 2,4,6-tris-(allyloxy)-1,3,5-triazine, 1,2-Bis-(diallylamo)-ethane, pentaerythritol tetratallate, 1,3,5,7-tetravinyl-1,3,5,7-tetramethyl-

67

cyclotetrasiloxane, 1,3,5,7-tetravinyl-1,3,5,7-tetramethylcyclotetrasiloxane, tris-[(2-acryloyloxy)ethyl]-phosphate, vinylboronic anhydride pyridine, 2,4,6-trivinylcyclotriboroxane pyridine, tetraallylsilane, tetraallyloxy silane, 1,3,5,7-tetramethyl-1,3,5,7-tetravinylcyclotetrasilazane and mixtures thereof; and wherein said chain transfer agent is selected from the group consisting of mercaptanes, malic acid, lactic acid, formic acid, isopropanol and hypophosphites, and mixtures thereof.

10. A composition according to claim 1, said composition having a Brookfield viscosity of from about 20 cps to about 1000 cps.

11. The composition according to claim 10, said composition has a Brookfield viscosity of from about 40 cps to about 300 cps.

12. The composition according to claim 10, said composition has a Brookfield viscosity of from about 50 cps to about 150 cps.

13. A composition according to claim 1, said composition comprising an adjunct material selected from the group consisting of surfactants, builders, chelating agents, dye transfer inhibiting agents, dispersants, enzymes, and enzyme

68

stabilizers, catalytic materials, bleach activators, hydrogen peroxide, sources of hydrogen peroxide, preformed peracids, polymeric dispersing agents, clay soil removal/anti-redeposition agents, brighteners, suds suppressors, dyes, hueing dyes, structure elasticizing agents, carriers, structurants, hydrotropes, processing aids, solvents and/or pigments and mixtures thereof.

14. A composition according to claim 1, said composition further comprising perfume.

15. A composition according to claim 1, said composition having a pH from about 2 to about 4.

16. The composition according to claim 1, wherein the anionic vinyl addition monomer is acrylic acid.

17. The composition according to claim 1, wherein the composition comprises, based upon total composition weight, from about 0.15% to about 0.24% of the polymeric material.

18. The composition according to claim 1, wherein the composition comprises, based upon total composition weight, from about 0.15% to about 0.2% of the polymeric material.

\* \* \* \* \*